



US006174636B1

(12) **United States Patent**  
**Fuller et al.**

(10) **Patent No.:** **US 6,174,636 B1**  
(b4) **Date of Patent:** **Jan. 16, 2001**

(54) **IMAGING MEMBERS CONTAINING ARYLENE ETHER ALCOHOL POLYMERS**

(75) Inventors: **Timothy J. Fuller**, Pittsford; **John F. Yanus**, Webster; **Damodar M. Pai**; **Markus R. Silvestri**, both of Fairport; **Ram S. Narang**, Macedon; **William W. Limburg**, Penfield; **Dale S. Renfer**, Webster, all of NY (US)

(73) Assignee: **Xerox Corporation**, Stamford, CT (US)

(\*) Notice: Under 35 U.S.C. 154(b), the term of this patent shall be extended for 0 days.

(21) Appl. No.: **09/326,170**

(22) Filed: **Jun. 4, 1999**

(51) **Int. Cl.<sup>7</sup>** ..... **G03G 5/05**

(52) **U.S. Cl.** ..... **430/58.7**; 430/56; 430/59.6; 430/59.1; 430/96

(58) **Field of Search** ..... 430/59.6, 59.1, 430/58.7, 96, 56

(56) **References Cited**

U.S. PATENT DOCUMENTS

|             |         |                        |          |
|-------------|---------|------------------------|----------|
| 2,125,968   | 8/1938  | Theimer                | 260/153  |
| 3,367,914   | 2/1968  | Herbert                | 260/53   |
| 3,455,868   | 7/1969  | D'Alessandro           | 260/38   |
| 3,914,194   | 10/1975 | Smith                  | 260/18 R |
| 4,086,209   | 4/1978  | Hara et al.            | 260/49   |
| 4,110,279   | 8/1978  | Nelson et al.          | 260/19 R |
| 4,435,496   | 3/1984  | Walls et al.           | 430/285  |
| 4,448,948   | 5/1984  | Tsubaki et al.         | 528/95   |
| 4,623,558   | 11/1986 | Lin                    | 427/44   |
| 4,667,010   | 5/1987  | Eldin                  | 528/125  |
| 4,739,032   | 4/1988  | Jones                  | 528/230  |
| 4,801,517   | 1/1989  | Frechet et al.         | 430/59   |
| 4,806,443   | 2/1989  | Yanus et al.           | 430/56   |
| 4,806,444   | 2/1989  | Yanus et al.           | 430/56   |
| 4,818,650   | 4/1989  | Limburg et al.         | 430/56   |
| 4,935,487   | 6/1990  | Yanus et al.           | 528/203  |
| 4,956,440   | 9/1990  | Limburg et al.         | 528/99   |
| 5,030,532   | 7/1991  | Limburg et al.         | 430/56   |
| 5,268,444   | 12/1993 | Jensen et al.          | 528/125  |
| 5,336,577   | 8/1994  | Spiewak et al.         | 430/59   |
| 5,336,720   | 8/1994  | Richards               | 525/78   |
| 5,438,082   | 8/1995  | Helmer-Metzmann et al. | 522/149  |
| 5,561,202   | 10/1996 | Helmer-Metzmann et al. | 525/471  |
| 5,728,498   | 3/1998  | Yanus et al.           | 430/59   |
| 5,750,300 * | 5/1998  | Nguyen et al.          | 430/96   |
| 5,874,192 * | 2/1999  | Fuller et al.          | 430/96   |
| 5,882,814 * | 3/1999  | Fuller et al.          | 430/96   |

FOREIGN PATENT DOCUMENTS

|              |         |       |
|--------------|---------|-------|
| 0-281-808    | 9/1988  | (EP). |
| 0 663 411 A1 | 7/1995  | (EP). |
| 0 698 823 A1 | 2/1996  | (EP). |
| 56-050-928   | 5/1981  | (JP). |
| 56-50-929    | 5/1981  | (JP). |
| 6-57-826     | 5/1981  | (JP). |
| 63-247757-A2 | 11/1988 | (JP). |
| 04294148     | 10/1992 | (JP). |

OTHER PUBLICATIONS

Daly, "Chloromethylation of Condensation Polymers Containing an Oxy-1,4-Phenylene Backbone," *Polymers Preprints* (1979), vol. 20, No.1, pp. 835-837.

Camps, "Chloromethylstyrene: Synthesis, Polymerization, Transformations, Applications," *JMS-Rev. Macromol. Chem. Phys.*, C22(3), 343-407 (1982-83).

(List continued on next page.)

\* cited by examiner

Primary Examiner—Christopher D. Rodee

(74) Attorney, Agent, or Firm—Judith L. Byorick

(57) **ABSTRACT**

Disclosed is an imaging member which comprises a conductive substrate, a photogenerating material, and a binder comprising a polymer of the formula



wherein A is



or a mixture of



wherein R is a hydrogen atom, an alkyl group, an aryl group, or mixtures thereof, B is one of specified groups, such as



or mixtures thereof, and n is an integer representing the number of repeating monomer units.

## OTHER PUBLICATIONS

- Tabata, "Pulse Radiolysis Studies on the Mechanism of the High Sensitivity of Chloromethylated Polystyrene as an Electron Negative Resist," 1984pp. 287–288.
- Jurek, "Deep UV Photochemistry of Copolymers of Trimethylsilylmethyl Methacrylate and Chloromethylstyrene," Polymer Preprints, 1988, pp. 546–547.
- Hergenrother, "Poly(arylene ethers)," Polymer, 1988, vol. 29, Feb.
- Havens, "Ethynyl-Terminated Polyarylates: Synthesis and Characterization," Journal of Polymer Science: Polymer Chemistry Edition, vol. 22 (1984), pp. 3011–3025.
- Hendricks, "Flare, A Low Dielectric Constant, High T<sub>g</sub>, Thermally Stable Poly(Arylene Ether) Dielectric for Microelectronic Circuit Interconnect Process Integration: Synthesis, Characterization, Thermomechanical Properties, and Thin-Film Processing Studies," Polymer Preprints 37(1) 150 (1996), vol. 37, No. 1, Mar. 1996, pp. 150–151.
- Zupancic, "Styrene Terminated Resins as Inerlevel Dielectrics for Multichip Modules," 1991, pp. 178–179.
- Percec, "Functional Polymers and Sequential Copolymers by Phase Transfer Catalysis, 2a)," Makromol Chem., 1984, pp. 1867–1880.
- Percec, "Functional Polymers and Sequential Copolymers by Phase Transfers Catalysis, 3a)," Makronal Chem., 1984, pp. 2319–2336.
- Percec, "Functional Polymers and Sequential Copolymers by Phase Transfer Catalysis 4. A New and Convenient Synthesis of p- and m-Hydrozymethylphenylacetylene," Polymer Bulletin 10, 223–230, 1983.
- Amato, "A New Preparation of Chloromethyl Methyl Ether Free of Bis(chloromethyl) Ether," 1979 Georg Thieme Publishers.
- McKillop, "A Simple and Inexpensive Procedure for Chloromethylation of Certain Aromatic Compounds," Tetrahedron Letters, vol. 24, No. 18, 1983, pp. 1933–1936.
- Tepeletsyna, "Synthesis of Intermediates for Production of Heat Resistant Polymers (Chloromethylation of Diphenyl Oxide)," Zhurnal Prikladnoi Khimii, vol. 40, No. 11, Nov., 1967, pp. 2540–2546.

**FIG. 1****FIG. 2**

**FIG. 3****FIG. 4**

IMAGING MEMBERS CONTAINING  
ARYLENE ETHER ALCOHOL POLYMERS

## BACKGROUND OF THE INVENTION

The present invention is directed to high performance polymers, processes for the preparation thereof, and articles and processes for the use thereof. More specifically, the present invention is directed to high performance polymers suitable for applications such as electrophotographic imaging members and the like. One embodiment of the present invention is directed to an imaging member which comprises a conductive substrate, a photogenerating material, and a binder comprising a polymer of the formula



wherein A is



or a mixture of



wherein R is a hydrogen atom, an alkyl group, an aryl group, or mixtures thereof, B is



-continued



$-(CH_2)_v-$ ,

wherein v is an integer of from 1 to about 20,



wherein z is an integer of from 2 to about 20,



wherein  $u$  is an integer of from 1 to about 20,



wherein  $w$  is an integer of from 1 to about 20,



wherein  $R_1$  and  $R_2$  each, independently of the other, are 65 hydrogen atoms, alkyl groups, or aryl groups, and  $p$  is an integer of 0 or 1,



10 wherein  $p$  is an integer of 0 or 1,



15

wherein  $t$  is an integer of from 1 to about 20,



20



25



30



35



40

wherein (1)  $Z$  is



45



50



55



60



or  $\text{Ar}-(X)_p-\text{Ar}$

wherein p is 0 or 1; (2) Ar is



or



(3) G is an alkyl group selected from alkyl or isoalkyl groups containing from about 2 to about 10 carbon atoms; (4) Ar' is



or



(5) X is



wherein s is 0, 1, or 2,



10 and (6) q is 0 or 1; or mixtures thereof, hydroxy-substituted, hydroxyalkyl-substituted, or hydroxyaryl-substituted derivatives thereof, or mixtures thereof, and n is an integer representing the number of repeating monomer units.

In one specific embodiment of the present invention, the polymer is of the formula



25 wherein P is a substituent which enables crosslinking of the polymer, a, b, c, and d are each integers of 0, 1, 2, 3, or 4, provided that at least one of a, b, c, and d is equal to or greater than 1 in at least some of the monomer repeat units 30 of the polymer.

In another specific embodiment of the present invention, the polymer is prepared by a process which comprises (1) providing a precursor polymer of the formula



40 wherein A is



B is



-continued



wherein v is an integer of from 1 to about 20,



wherein z is an integer of from 2 to about 20,



10 wherein u is an integer of from 1 to about 20,



wherein w is an integer of from 1 to about 20,



**9**

5

wherein  $R_1$  and  $R_2$  each, independently of the other, are hydrogen atoms, alkyl groups, or aryl groups, and  $p$  is an integer of 0 or 1,

**10**or  $\text{---Ar---}(X)_p\text{---Ar---}$ 

wherein  $p$  is 0 or 1; (2)  $\text{Ar}$  is



15

wherein  $p$  is an integer of 0 or 1,

 $\text{---}(\text{CH}_2\text{O})_t\text{---}$ 

wherein  $t$  is an integer of from 1 to about 20,



20



or



25

30 (3)  $\text{G}$  is an alkyl group selected from alkyl or isoalkyl groups containing from about 2 to about 10 carbon atoms; (4)  $\text{Ar}'$  is



35



40



45

50 (5)  $\text{X}$  is



55



60



65

wherein (1)  $\text{Z}$  is



-continued



wherein s is 0, 1, or 2,



and (6) q is 0 or 1; or mixtures thereof, hydroxy-substituted, 25 hydroxyalkyl-substituted, or hydroxyaryl-substituted derivatives thereof, or mixtures thereof, and n is an integer representing the number of repeating monomer units, and 30 (2) reacting the precursor polymer with borane, resulting in formation of a polymer of the formula



wherein A is



or a mixture of



wherein R is a hydrogen atom, an alkyl group, an aryl group, 55 or mixtures thereof.

In yet another specific embodiment of the present invention, the polymer is prepared by a process which comprises (1) providing a precursor polymer of the formula 60



10 B is



13



wherein v is an integer of from 1 to about 20,



wherein z is an integer of from 2 to about 20,



wherein u is an integer of from 1 to about 20,



wherein w is an integer of from 1 to about 20,



14

-continued



25

wherein R<sub>1</sub> and R<sub>2</sub> each, independently of the other, are hydrogen atoms, alkyl groups, or aryl groups, and p is an integer of 0 or 1,



35

wherein p is an integer of 0 or 1,



wherein t is an integer of from 1 to about 20,



50

$-\text{[C}_6\text{H}_4\text{C(=O)C}_6\text{H}_4\text{]}_p-$ ,



15

wherein (1) Z is



wherein p is 0 or 1; (2) Ar is



(3) G is an alkyl group selected from alkyl or isoalkyl groups containing from about 2 to about 10 carbon atoms; (4) Ar' is

or

16

(5) X is



30

wherein  $s$  is 0, 1, or 2,



40 and (6) q is 0 or 1; or mixtures thereof, hydroxy-substituted, hydroxyalkyl-substituted, or hydroxyaryl-substituted derivatives thereof, or mixtures thereof, and n is an integer representing the number of repeating monomer units, (2)  
45 reacting the precursor polymer with a reagent of the formula  $\text{RMgX}$ , wherein R is a hydrogen atom, an alkyl group, an aryl group, or mixtures thereof and X is a halogen atom, and (3) subsequent to step 2, adding water or acid to the precursor polymer, thereby resulting in formation of a  
50 polymer of the formula



60 wherein A is



or a mixture of



wherein R is a hydrogen atom, an alkyl group, an aryl group, or mixtures thereof.

The formation and development of images on the surface of photoconductive materials by electrostatic means is well known. The basic electrophotographic imaging process, as taught by C. F. Carlson in U.S. Pat. No. 2,297,691, entails placing a uniform electrostatic charge on a photoconductive imaging member, exposing the imaging member to a light and shadow image to dissipate the charge on the areas of the imaging member exposed to the light, and developing the resulting electrostatic latent image by depositing on the image a finely divided electroscopic material known as toner. In charge area development (CAD) systems, the toner will normally be attracted to those areas of the imaging member which retain a charge, thereby forming a toner image corresponding to the electrostatic latent image. In discharge area development (DAD) systems, the toner will normally be attracted to those areas of the imaging member which have less or no charge as a result of exposure to light, thereby forming a toner image corresponding to the electrostatic latent image. This developed image may then be transferred to a substrate such as paper. The transferred image may subsequently be permanently affixed to the substrate by heat, pressure, a combination of heat and pressure, or other suitable fixing means such as solvent or overcoating treatment.

Imaging members for electrophotographic imaging systems comprising selenium alloys vacuum deposited on substrates are known. Imaging members have also been prepared by coating substrates with photoconductive particles dispersed in an organic film forming binder. Coating of rigid drum substrates has been effected by various techniques such as spraying, dip coating, vacuum evaporation, and the like. Flexible imaging members can also be manufactured by processes that entail coating a flexible substrate with the desired photoconducting material.

Some photoresponsive imaging members consist of a homogeneous layer of a single material such as vitreous selenium, and others comprise composite layered devices containing a dispersion of a photoconductive composition. An example of a composite xerographic photoconductive member is described in U.S. Pat. No. 3,121,006, which discloses finely divided particles of a photoconductive inorganic compound dispersed in an electrically insulating organic resin binder. Imaging members prepared according to the teachings of this patent contain a binder layer with particles of zinc oxide uniformly dispersed therein coated on a paper backing. The binders disclosed in this patent include materials such as polycarbonate resins, polyester resins, polyamide resins, and the like.

Photoreceptor materials comprising inorganic or organic materials wherein the charge generating and charge transport functions are performed by discrete contiguous layers are also known. Additionally, layered photoreceptor members are disclosed in the prior art, including photoreceptors having an overcoat layer of an electrically insulating polymeric material. Other layered photoresponsive devices have been disclosed, including those comprising separate photo-generating layers and charge transport layers as described in U.S. Pat. No. 4,265,990, the disclosure of which is totally

incorporated herein by reference. Photoresponsive materials containing a hole injecting layer overcoated with a hole transport layer, followed by an overcoating of a photogenerating layer, and a top coating of an insulating organic resin, are disclosed in U.S. Pat. No. 4,251,612, the disclosure of which is totally incorporated herein by reference. Examples of photogenerating layers disclosed in these patents include trigonal selenium and phthalocyanines, while examples of transport layers include certain aryl diamines as illustrated therein.

In addition, U.S. Pat. No. 3,041,167 discloses an overcoated imaging member containing a conductive substrate, a photoconductive layer, and an overcoating layer of an electrically insulating polymeric material. This member can be employed in electrophotographic imaging processes by initially charging the member with an electrostatic charge of a first polarity, followed by exposing it to form an electrostatic latent image that can subsequently be developed to form a visible image.

U.S. Pat. No. 3,914,194 (Smith), the disclosure of which is totally incorporated herein by reference, discloses a formaldehyde copolymer resin having dependent unsaturated groups with the repeating unit



wherein R is an aliphatic acyl group derived from saturated acids having 2 to 6 carbons, olefinically unsaturated acids having 3 to 20 carbons, or an omega-carboxy-aliphatic acyl group derived from olefinically unsaturated dicarboxylic acids having 4 to 12 carbons or mixtures thereof, R<sub>1</sub> is independently hydrogen, an alkyl group of 1 to 10 carbon atoms, or halogen, Z is selected from oxygen, sulfur, the group represented by Z taken with the dotted line represents dibenzofuran and dibenzothiophene moieties, or mixtures thereof, n is a whole number sufficient to give a weight average molecular weight greater than about 500, m is 0 to 2, p and q have an average value of 0 to 1 with the proviso that the total number of p and q groups are sufficient to give greater than one unsaturated group per resin molecule. These resins are useful to prepare coatings on various substrates or for potting electrical components by mixing with reactive diluents and curing agents and curing.

“Chloromethylation of Condensation Polymers Containing an oxy-1,4-phenylene Backbone,” W. H. Daly et al., *Polymer Preprints*, Vol. 20, No. 1, 835 (1979), the disclosure of which is totally incorporated herein by reference, discloses the chloromethylation of polymers containing oxy-phenylene repeat units to produce film forming resins with high chemical reactivity. The utility of 1,4-bis (chloromethoxy) butane and 1-chloromethoxy-4-chlorobutane as chloromethylating agents are also described.

European Patent Application EP-0,698,823-A1 (Fahey et al.), the disclosure of which is totally incorporated herein by reference, discloses a copolymer of benzophenone and bisphenol A which was shown to have deep ultraviolet absorption properties. The copolymer was found useful as an antireflective coating in microlithography applications. Incorporating anthracene into the copolymer backbone enhanced absorption at 248 nm. The encapper used for the

copolymer varied depending on the needs of the user and was selectable to promote adhesion, stability, and absorption of different wavelengths.

M. Camps, M. Chatzopoulos, and J. Montheard, "Chloromethyl Styrene: Synthesis, Polymerization, Transformations, Applications," *JMS—Rev. Macromol. Chem. Phys.*, C22(3), 343–407 (1982-3), the disclosure of which is totally incorporated herein by reference, discloses processes for the preparation of chloromethyl-substituted polystyrenes, as well as applications thereof.

Y. Tabata, S. Tagawa, and M. Washio, "Pulse Radiolysis Studies on the Mechanism of the High Sensitivity of Chloromethylated Polystyrene as an Electron Negative Resist," *Lithography*, 25(1), 287 (1984), the disclosure of which is totally incorporated herein by reference, discloses the use of chloromethylated polystyrene in resist applications.

M. J. Jurek, A. E. Novembre, I. P. Heyward, R. Gooden, and E. Reichmanis, "Deep UV Photochemistry of Copolymers of Trimethyl-Silylmethyl Methacrylate and Chloromethylstyrene," *Polymer Preprints*, 29(1) (1988), the disclosure of which is totally incorporated herein by reference, discloses the use of an organosilicon polymer of chloromethylstyrene for resist applications.

P. M. Hergenrother, B. J. Jensen, and S. J. Havens, "Poly(arylene ethers)," *Polymer*, 29, 358 (1988), the disclosure of which is totally incorporated herein by reference, discloses several arylene ether homopolymers and copolymers prepared by the nucleophilic displacement of aromatic dihalides with aromatic potassium bisphenates. Polymer glass transition temperatures ranged from 114 to 310° C. and some were semicrystalline. Two ethynyl-terminated poly(arylene ethers) were synthesized by reacting hydroxy-terminated oligomers with 4-ethynylbenzoyl chloride. Heat induced reaction of the acetylenic groups provided materials with good solvent resistance. The chemistry, physical, and mechanical properties of the polymers are also disclosed.

S. J. Havens, "Ethynyl-Terminated Polyarylates: Synthesis and Characterization," *Journal of Polymer Science: Polymer Chemistry Edition*, vol. 22, 3011–3025 (1984), the disclosure of which is totally incorporated herein by reference, discloses hydroxy-terminated polyarylates with number average molecular weights of about 2500, 5000, 7500, and 10,000 which were synthesized and converted to corresponding 4-ethynylbenzoyloxy-terminated polyarylates by reaction with 4-ethynylbenzoyl chloride. The terminal ethynyl groups were thermally reacted to provide chain extension and crosslinking. The cured polymer exhibited higher glass transition temperatures and better solvent resistance than a high molecular weight linear polyarylate.

Solvent resistance was further improved by curing 2,2-bis(4-ethynylbenzoyloxy-4'-phenyl)propane, a coreactant, with the ethynyl-terminated polymer at concentrations of about 10 percent by weight.

N. H. Hendricks and K. S. Y. Lau, "Flare, a Low Dielectric Constant, High Tg, Thermally Stable Poly(arylene ether) Dielectric for Microelectronic Circuit Interconnect Process Integration: Synthesis, Characterization, Thermomechanical Properties, and Thin-Film Processing Studies," *Polymer Preprints*, 37(1), 150 (1996), the disclosure of which is totally incorporated herein by reference, discloses non-carbonyl containing aromatic polyethers such as fluorinated poly(arylene ethers) based on decafluorobiphenyl as a class of intermetal dielectrics for applications in sub-half micron multilevel interconnects.

J. J. Zupancic, D. C. Blazej, T. C. Baker, and E. A. Dinkel, "Styrene Terminated Resins as Interlevel Dielectrics for Multichip Models," *Polymer Preprints*, 32, (2), 178 (1991),

the disclosure of which is totally incorporated herein by reference, discloses vinylbenzyl ethers of polyphenols (styrene terminated resins) which were found to be photochemically and thermally labile, generating highly crosslinked networks. The resins were found to yield no volatile by-products during the curing process and high glass transition, low dielectric constant coatings. One of the resins was found to be spin coatable to varying thickness coatings which could be photodefined, solvent developed, and then hard baked to yield an interlevel dielectric.

Japanese Patent Kokai JP 04294148-A, the disclosure of which is totally incorporated herein by reference, discloses a liquid injecting recording head containing the cured matter of a photopolymerizable composition comprising (1) a graft polymer comprising (A) alkyl methacrylate, acrylonitrile, and/or styrene as the trunk chain and an —OH group-containing acryl monomer, (B) amino or alkylamino group-containing acryl monomer, (C) carboxyl group-containing acryl or vinyl monomers, (D) N-vinyl pyrrolidone, vinyl pyridine or its derivatives, and/or (F) an acrylamide as the side chain; (2) a linear polymer containing constitutional units derived from methyl methacrylate, ethyl methacrylate, isobutyl methacrylate, t-butyl methacrylate, benzyl methacrylate, acrylonitrile, isobornyl methacrylate, tricyclo-decane acrylate, tricyclodecane oxyethyl methacrylate, styrene, dimethylaminoethyl methacrylate, and/or cyclohexyl methacrylate, and constitutional unit derived from the above compounds (A), (B), (C), (D), (E), or (F) above; (3) an ethylenic unsaturated bond containing monomer; and (4) a photopolymerization initiator which contains (a) an organic peroxide, s-triazine derivative, benzophenone or its derivatives, quinones, N-phenylglycine, and/or alkylarylketones as a radical generator and (b) coumarin dyes, keto-coumarin dyes, cyanine dyes, merocyanine dyes, and/or xanthene dyes as a sensitizer. "Functional Polymers and Sequential Copolymers by Phase Transfer Catalysis, 2a: Synthesis and Characterization of Aromatic Poly(ether sulfone)s Containing Vinylbenzyl and Ethynylbenzyl Chain Ends," V. Percec and B. C. Auman, *Makromol. Chem.*, 185, 1867–1880 (1984), the disclosure of which is totally incorporated herein by reference, discloses a method for the synthesis of  $\alpha,\omega$ -bis(vinylbenzyl) aromatic poly(ether sulfone)s and their transformation into  $\alpha,\omega$ -bis(ethynylbenzyl) aromatic poly(ether sulfone)s. The method entails a fast and quantitative Williamson etherification of the  $\alpha,\omega$ -bis(hydroxyphenyl) polysulfone with a mixture of p- and m-chloromethylstyrenes in the presence of tetrabutylammonium hydrogen sulfate as phase transfer catalyst, a subsequent bromination, and then a dehydrobromination with potassium tert-butoxide. The DSC study of the thermal curing of the  $\alpha,\omega$ -bis(vinylbenzyl) aromatic poly(ether sulfone)s and  $\alpha,\omega$ -bis(ethynylbenzyl) aromatic poly(ether sulfone)s demonstrates high thermal reactivity for the styrene-terminated oligomers.

"Functional Polymers and Sequential Copolymers by Phase Transfer Catalysis, 3a: Synthesis and Characterization of Aromatic Poly(ether sulfone)s and Poly(oxy-2,6-dimethyl-1,4-phenylene) Containing Pendent Vinyl Groups," V. Percec and B. C. Auman, *Makromol. Chem.*, 185, 2319–2336 (1984), the disclosure of which is totally incorporated herein by reference, discloses a method for the syntheses of  $\alpha,\Omega$ -benzyl aromatic poly(ether sulfone)s (PSU) and poly(oxy-2,6-dimethyl-1,4-phenylene) (POP) containing pendant vinyl groups. The first step of the synthetic procedure entails the chloromethylation of PSU and POP to provide polymers with chloromethyl groups. POP, containing bromomethyl groups, was obtained by radical

bromination of the methyl groups. Both chloromethylated and bromomethylated starting materials were transformed into their phosphonium salts, and then subjected to a phase transfer catalyzed Wittig reaction to provide polymers with pendant vinyl groups. A PSU with pendant ethynyl groups was prepared by bromination of the PSU containing vinyl groups, followed by a phase transfer catalyzed dehydrobromination. DSC of the thermal curing of the polymers containing pendant vinyl and ethynyl groups showed that the curing reaction is much faster for the polymers containing vinyl groups. The resulting network polymers are flexible when the starting polymer contains vinyl groups, and very rigid when the starting polymer contains ethynyl groups.

"Functional Polymers and Sequential Copolymers by Phase Transfer Catalysis," V. Percec and P. L. Rinaldi, *Polymer Bulletin*, 70, 223 (1983), the disclosure of which is totally incorporated herein by reference, discloses the preparation of p- and m-hydroxymethylphenylacetylenes by a two step sequence starting from a commercial mixture of p- and m-chloromethylstyrene, i.e., by the bromination of the vinylic monomer mixture followed by separation of m- and p-brominated derivatives by fractional crystallization, and simultaneous dehydrobromination and nucleophilic substitution of the —Cl with —OH.

U.S. Pat. No. 4,110,279 (Nelson et al.), the disclosure of which is totally incorporated herein by reference, discloses a polymer derived by heating in the presence of an acid catalyst at between about 65° C. and about 250° C.: I. a reaction product, a cogeneric mixture of alkoxy functional compounds, having average equivalent weights in the range of from about 220 to about 1200, obtained by heating in the presence of a strong acid at about 50° C. to about 250° C.: (A) a diaryl compound selected from naphthalene, diphenyl oxide, diphenyl sulfide, their alkylated or halogenated derivatives, or mixtures thereof, (B) formaldehyde or form-aldehyde yielding derivative, (C) water, and (D) a hydroxy aliphatic hydrocarbon compound having at least one free hydroxyl group and from 1 to 4 carbon atoms, which mixture contains up to 50 percent unreacted (A); with II. at least one monomeric phenolic reactant selected from the group



wherein R is selected from the group consisting of hydrogen, alkyl radical of 1 to 20 carbon atoms, aryl radical of 6 to 20 carbon atoms, wherein R<sub>1</sub> represents hydrogen, alkyl, or aryl, m represents an integer from 1 to 3, o represents an integer from 1 to 5, p represents an integer from 0 to 3, X represents oxygen, sulfur, or alkylidene, and q represents an integer from 0 to 1; and III. optionally an aldehyde or aldehyde-yielding derivative or ketone, for from several minutes to several hours. The polymeric materials are liquids or low melting solids which are capable of further modification to thermoset resins. These polymers are capable of being thermoset by heating at a temperature of from about 130° C. to about 260° C. for from several minutes to several hours in the presence of a formaldehyde-yielding compound. These polymers are also capable of further modification by reacting under basic conditions with formaldehyde with or without a phenolic compound. The

polymers, both base catalyzed resoles and acid catalyzed novolacs, are useful as laminating, molding, film-forming, and adhesive materials. The polymers, both resoles and novolacs, can be epoxidized as well as reacted with a drying oil to produce a varnish resin.

U.S. Pat. No. 3,367,914 (Herbert), the disclosure of which is totally incorporated herein by reference, discloses thermosetting resinous materials having melting points in the range of from 150° C. to 350° C. which are made heating at 10 a temperature of from -10° C. to 100° C. for 5 to 30 minutes an aldehyde such as formaldehyde or acetaldehyde with a mixture of poly(aminomethyl) diphenyl ethers having an average of from about 1.5 to 4.0 aminomethyl groups. After the resins are cured under pressure at or above the melting 15 point, they form adherent tough films on metal substrates and thus are useful as wire coatings for electrical magnet wire for high temperature service at 180° C. or higher.

J. S. Amato, S. Karady, M. Sletzinger, and L. M. Weinstock, "A New Preparation of Chloromethyl Methyl Ether Free of Bis(chloromethyl) Ether," *Synthesis*, 970 20 (1979), the disclosure of which is totally incorporated herein by reference, discloses the synthesis of chloromethyl methyl ether by the addition of acetyl chloride to a slight excess of anhydrous dimethoxymethane containing a catalytic amount 25 of methanol at room temperature. The methanol triggers a series of reactions commencing with formation of hydrogen chloride and the reaction of hydrogen chloride with dimethoxymethane to form chloromethyl methyl ether and methanol in an equilibrium process. After 36 hours, a 30 near-quantitative conversion to an equimolar mixture of chloromethyl methyl ether and methyl acetate is obtained.

A. McKillop, F. A. Madjdabadi, and D. A. Long, "A Simple and Inexpensive Procedure for Chloromethylation of Certain Aromatic Compounds," *Tetrahedron Letters*, Vol. 35 24, No. 18, pp. 1933-1936 (1983), the disclosure of which is totally incorporated herein by reference, discloses the reaction of a range of aromatic compounds with methoxy-acetyl chloride and aluminum chloride in either nitromethane or carbon disulfide to result in chloromethylation in good to excellent yield.

E. P. Tepenitsyna, M. I. Farberov, and A. P. Ivanovskii, "Synthesis of Intermediates for Production of Heat Resistant Polymers (Chloromethylation of Diphenyl Oxide)," *Zhurnal Prikladnoi Khimii*, Vol. 40, No. 11, pp. 2540-2546 (1967), 45 the disclosure of which is totally incorporated herein by reference, discloses the chloromethylation of diphenyl oxide by (1) the action of paraformaldehyde solution in glacial acetic acid saturated with hydrogen chloride, and by (2) the action of paraformaldehyde solution in concentrated hydrochloric acid.

U.S. Pat. No. 2,125,968 (Theimer), the disclosure of which is totally incorporated herein by reference, discloses the manufacture of aromatic alcohols by the Friedel-Crafts reaction, in which an alkylene oxide is condensed with a Friedel-Crafts reactant in the presence of an anhydrous metal halide.

U.S. Pat. No. 5,994,425 and Copending U.S. application Ser. No. 09/221,024, filed Dec. 23, 1998, entitled "Curable Compositions," with the named inventors Timothy J. Fuller, 60 Ram S. Narang, Thomas W. Smith, David J. Luca, and Ralph A. Mosher, the disclosures of each of which are totally incorporated herein by reference, disclose an improved composition comprising a photopatternable polymer containing at least some monomer repeat units with photosensitivity-imparting substituents, said photopatternable polymer being of the general formula



or



wherein x is an integer of 0 or 1, A is one of several specified groups, such as



B is one of several specified groups, such as



or mixtures thereof, and n is an integer representing the number of repeating monomer units. Also disclosed is a process for preparing a thermal ink jet printhead with the aforementioned polymer and a thermal ink jet printhead containing therein a layer of a crosslinked or chain extended polymer of the above formula.

U.S. Pat. No. 5,849,809, filed Aug. 29, 1996, and Copending U.S. application Ser. No. 09/159,426, filed Sep. 23, 1998, entitled "Hydroxylated High Performance Curable Polymers," with the named inventors Ram S. Narang and Timothy J. Fuller, the disclosures of each of which are totally incorporated herein by reference, disclose a composition which comprises (a) a polymer containing at least some monomer repeat units with photosensitivity-imparting substituents which enable crosslinking or chain extension of the polymer upon exposure to actinic radiation, said polymer

being of the formula



or



wherein x is an integer of 0 or 1, A is one of several specified groups, such as



B is one of several specified groups, such as



or mixtures thereof, and n is an integer representing the number of repeating monomer units, wherein said photosensitivity-imparting substituents are hydroxylated groups; (b) at least one member selected from the group consisting of photoinitiators and sensitizers; and (c) an optional solvent. Also disclosed are processes for preparing the above polymers and methods of preparing thermal ink jet printheads containing the above polymers.

Copending U.S. application Ser. No. 08/705,488, filed Aug. 29, 1996, entitled "High Performance Polymer Compositions Having Photosensitivity-Imparting Substituents and Thermal Sensitivity-Imparting Substituents," and Copending U.S. application Ser. No. 09/221,690, filed Dec. 23, 1998, entitled "High Performance Polymer Compositions," with the named inventors Thomas W. Smith,

25

Timothy J. Fuller, Ram S. Narang, and David J. Luca, the disclosures of each of which are totally incorporated herein by reference, disclose a composition comprising a polymer with a weight average molecular weight of from about 1,000 to about 65,000, said polymer containing at least some monomer repeat units with a first, photosensitivity-imparting substituent which enables crosslinking or chain extension of the polymer upon exposure to actinic radiation, said polymer also containing a second, thermal sensitivity-imparting substituent which enables further polymerization of the polymer upon exposure to temperatures of about 140° C. and higher, wherein the first substituent is not the same as the second substituent, said polymer being selected from the group consisting of polysulfones, polyphenylenes, polyether sulfones, polyimides, polyamide imides, polyarylene ethers, polyphenylene sulfides, polyarylene ether ketones, phenoxy resins, polycarbonates, polyether imides, polyquinoxalines, polyquinolines, polybenzimidazoles, polybenzoxazoles, polybenzothiazoles, polyoxadiazoles, copolymers thereof, and mixtures thereof.

U.S. Pat. No. 5,889,077, filed Aug. 29, 1996, and Copending U.S. application Ser. No. 09/221,278, filed Dec. 23, 1998, entitled "Process for Direct Substitution of High Performance Polymers with Unsaturated Ester Groups," with the named inventors Timothy J. Fuller, Ram S. Narang, Thomas W. Smith, David J. Luca, and Raymond K. Crandall, the disclosures of each of which are totally incorporated herein by reference, disclose a process which comprises reacting a polymer of the general formula



or



wherein x is an integer of 0 or 1, A is one of several specified groups, such as



B is one of several specified groups, such as



26

-continued



or mixtures thereof, and n is an integer representing the number of repeating monomer units, with (i) a formaldehyde source, and (ii) an unsaturated acid in the presence of an acid catalyst, thereby forming a curable polymer with unsaturated ester groups. Also disclosed is a process for preparing an ink jet printhead with the above polymer.

U.S. Pat. No. 5,739,254, filed Aug. 29, 1996, and U.S. Pat. No. 5,753,783, filed Aug. 28, 1997, entitled "Process for Haloalkylation of High Performance Polymers," with the named inventors Timothy J. Fuller, Ram S. Narang, Thomas W. Smith, David J. Luca, and Raymond K. Crandall, the disclosures of each of which are totally incorporated herein by reference, disclose a process which comprises reacting a polymer of the general formula



or



55

50

45

40

35

30

25

20

15

10

5

1

0

wherein x is an integer of 0 or 1, A is one of several specified groups, such as



65

27

B is one of several specified groups, such as



or mixtures thereof, and  $n$  is an integer representing the number of repeating monomer units, with an acetyl halide and dimethoxymethane in the presence of a halogen-containing Lewis acid catalyst and methanol, thereby forming a haloalkylated polymer. In a specific embodiment, the haloalkylated polymer is then reacted further to replace at least some of the haloalkyl groups with photosensitivity-imparting groups. Also disclosed is a process for preparing a thermal ink jet printhead with the aforementioned polymer.

U.S. Pat. No. 5,761,809, filed Aug. 29, 1996, entitled "Processes for Substituting Haloalkylated Polymers With Unsaturated Ester, Ether, and Alkylcarboxymethylene Groups," with the named inventors Timothy J. Fuller, Ram S. Narang, Thomas W. Smith, David J. Luca, and Raymond K. Crandall, the disclosure of which is totally incorporated herein by reference, discloses a process which comprises reacting a haloalkylated aromatic polymer with a material selected from the group consisting of unsaturated ester salts, alkoxide salts, alkylcarboxylate salts, and mixtures thereof, thereby forming a curable polymer having functional groups corresponding to the selected salt. Another embodiment of the invention is directed to a process for preparing an ink jet printhead with the curable polymer thus prepared.

U.S. Pat. No. 5,958,995 and Copending U.S. application Ser. No. 09/220,273, filed Dec. 23, 1998, entitled "Blends Containing Curable Polymers," with the named inventors Ram S. Narang and Timothy J. Fuller, the disclosures of each of which are totally incorporated herein by reference, disclose a composition which comprises a mixture of (A) a first component comprising a polymer, at least some of the monomer repeat units of which have at least one photosensitivity-imparting group thereon, said polymer having a first degree of photosensitivity-imparting group substitution measured in milliequivalents of photosensitivity-imparting group per gram and being of the general formula

2

-continued

ON



15

wherein x is an integer of 0 or 1, A is one of several specified groups, such as



B is one of several specified groups, such as



or mixtures thereof, and n is an integer representing the number of repeating monomer units, and (B) a second component which comprises either (1) a polymer having a second degree of photosensitivity-imparting group substitution measured in milliequivalents of photosensitivity-imparting group per gram lower than the first degree of photosensitivity-imparting group substitution, wherein said second degree of photosensitivity-imparting group substitution may be zero, wherein the mixture of the first component and the second component has a third degree of photosensitivity-imparting group substitution measured in milliequivalents of photosensitivity-imparting group per gram which is lower than the first degree of photosensitivity-imparting group substitution and higher than the second degree of photosensitivity-imparting group substitution, or (2) a reactive diluent having at least one photosensitivity-imparting group per molecule and having a fourth degree of photosensitivity-imparting group substitution measured in milliequivalents of photosensitivity-imparting group per gram, wherein the mixture of the first component and the

29

second component has a fifth degree of photosensitivity-imparting group substitution measured in milliequivalents of photosensitivity-imparting group per gram which is higher than the first degree of photosensitivity-imparting group substitution and lower than the fourth degree of photosensitivity-imparting group substitution; wherein the weight average molecular weight of the mixture is from about 10,000 to about 50,000; and wherein the third or fifth degree of photosensitivity-imparting group substitution is from about 0.25 to about 2 milliequivalents of photosensitivity-imparting groups per gram of mixture. Also disclosed is a process for preparing a thermal ink jet printhead with the aforementioned composition.

U.S. Pat. No. 5,945,253 and Copending U.S. application Ser. No. 09/246,167, filed Feb. 8, 1999, entitled "High Performance Curable Polymers and Processes for the Preparation Thereof," with the named inventors Ram S. Narang and Timothy J. Fuller, the disclosures of each of which are totally incorporated herein by reference, disclose a composition which comprises a polymer containing at least some monomer repeat units with photosensitivity-imparting substituents which enable crosslinking or chain extension of the polymer upon exposure to actinic radiation, said polymer being of the formula



wherein x is an integer of 0 or 1, A is one of several specified groups, such as



B is one of several specified groups, such as



30

-continued



or mixtures thereof, and n is an integer representing the number of repeating monomer units, wherein said photosensitivity-imparting substituents are allyl ether groups, epoxy groups, or mixtures thereof. Also disclosed are a process for preparing a thermal ink jet printhead containing the aforementioned polymers and processes for preparing the aforementioned polymers.

U.S. Pat. No. 5,863,963, filed Aug. 29, 1996, and Copending U.S. application Ser. No. 09/163,672, filed Sep. 30, 1998, entitled "Halomethylated High Performance Curable Polymers," with the named inventors Ram S. Narang and Timothy J. Fuller, the disclosures of each of which are totally incorporated herein by reference, disclose a process which comprises the steps of (a) providing a polymer containing at least some monomer repeat units with halomethyl group substituents which enable crosslinking or chain extension of the polymer upon exposure to a radiation source which is electron beam radiation, x-ray radiation, or deep ultraviolet radiation, said polymer being of the formula



wherein x is an integer of 0 or 1, A is one of several specified groups, such as



31

B is one of several specified groups, such as



or mixtures thereof, and n is an integer representing the 25 number of repeating monomer units, and (b) causing the polymer to become crosslinked or chain extended through the photosensitivity-imparting groups. Also disclosed is a process for preparing a thermal ink jet printhead by the aforementioned curing process.

U.S. Pat. No. 6,007,877 and Copending U.S. application Ser. No. 09/247,104, filed Feb. 9, 1999, entitled "Aqueous Developable High Performance Curable Polymers," with the named inventors Ram S. Narang and Timothy J. Fuller, the disclosures of each of which are totally incorporated herein by reference, disclose a composition which comprises a polymer containing at least some monomer repeat units with water-solubility-imparting substituents and at least some monomer repeat units with photosensitivity-imparting substituents which enable crosslinking or chain extension of the polymer upon exposure to actinic radiation, said polymer being of the formula



or



32

wherein x is an integer of 0 or 1, A is one of several specified groups, such as



10 B is one of several specified groups, such as



20

30

35

or mixtures thereof, and n is an integer representing the 25 number of repeating monomer units. In one embodiment, a 40 single functional group imparts both photosensitivity and water solubility to the polymer. In another embodiment, a first functional group imparts photosensitivity to the polymer and a second functional group imparts water solubility 45 to the polymer. Also disclosed is a process for preparing a thermal ink jet printhead with the aforementioned polymers.

U.S. Pat. No. 5,814,426, filed Nov. 21, 1997, entitled 50 "Imaging Members Containing High Performance Polymers," with the named inventors Kathleen M. Carmichael, Timothy J. Fuller, Edward F. Grabowski, Damodar M. Pai, Leon A. Teuscher, John F. Yanus, and Paul 55 F. Zukoski, the disclosure of which is totally incorporated herein by reference, discloses an imaging member which comprises a conductive substrate, a photogenerating material, and a binder which comprises a polymer of the 60 formulae I, II, III, IV, V, VI VII VIII, IX, or X:





-continued



X



35

wherein x is an integer of 0 or 1, A is



-continued



40



45



50



55



60

65

**39**

-continued



or mixtures thereof, B is

**40**

-continued

20 wherein v is an integer of from 1 to about 20,  
-(CH2O)<sub>v</sub>,

wherein t is an integer of from 1 to about 20,



30 wherein z is an integer of from 2 to about 20,



40 wherein u is an integer of from 1 to about 20,



65

**41**

wherein w is an integer of from 1 to about 20,

**42****42**

-continued



5

or mixtures thereof, C is

10



15



20



25



or mixtures thereof, wherein R is an alkyl group, an aryl group, an arylalkyl group, or mixtures thereof, and m and n are integers representing the number of repeating units.

U.S. Pat. No. 5,882,814, filed Nov. 21, 1997, entitled "Imaging Members Containing High Performance Charge Transporting Polymers," with the named inventors Timothy J. Fuller, Damodar M. Pai, Leon A. Teuscher, and John F. Yanus, the disclosure of which is totally incorporated herein by reference, discloses an imaging member which comprises a conductive substrate, a photogenerating layer, and a charge transport layer comprising a polymer of the formulae I, II, III, IV, V, VI, VII, VIII, IX, or X:

I



II



III



-continued



IV



V



VI



-continued

VII



VIII



IX



X



-continued



wherein x is an integer of 0 or 1, A is



-continued

15



20

25 or mixtures thereof, B is



65

49



wherein v is an integer of from 1 to about 20,



wherein t is an integer of from 1 to about 20,



wherein z is an integer of from 2 to about 20,



wherein u is an integer of from 1 to about 20,



50



15 wherein w is an integer of from 1 to about 20,



51

wherein (1) Z is



52

(5) X is



wherein p is 0 or 1; (2) Ar is



30     wherein s is 0, 1, or 2,

40     and (6) q is 0 or 1; or mixtures thereof, wherein at least some  
45     of the "B" groups are of the formula

C is

(3) G is an alkyl group selected from alkyl or isoalkyl groups  
containing from about 2 to about 10 carbon atoms; (4) Ar' is



or mixtures thereof, wherein R is an alkyl group, an aryl group, an arylalkyl group, or mixtures thereof, and m and n are integers representing the number of repeating units.

U.S. Pat. No. 5,874,192, filed Nov. 21, 1997, entitled "Imaging Members with Charge Transport Layers Containing High Performance Polymer Blends," with the named inventors Kathleen M. Carmichael, Timothy J. Fuller, Edward F. Grabowski, Damodar M. Pai, Leon A. Teuscher, John F. Yanus, and Paul F. Zukoski, the disclosure of which is totally incorporated herein by reference, discloses an imaging member which comprises a conductive substrate, a photogenerating material, a charge transport material, and a polymeric binder comprising (a) a first polymer comprising a polycarbonate, and (b) a second polymer of the formulae I, II III, IV, V, VI, VII, VIII, IX, or X:







**59**

wherein x is an integer of 0 or 1, A is

**60**

or mixtures thereof, B is



wherein v is an integer of from 1 to about 20,

65

-(CH2O)<sub>7</sub>-

**61**

wherein t is an integer of from 1 to about 20,



wherein z is an integer of from 2 to about 20,



wherein u is an integer of from 1 to about 20,



wherein w is an integer of from 1 to about 20,

**62**

-continued



30 or mixtures thereof, C is



55 or mixtures thereof, wherein R is an alkyl group, an aryl group, an arylalkyl group, or mixtures thereof, and m and n are integers representing the numbers of repeating units.

Copending U.S. application Ser. No. 09/105,501, filed Jun. 26, 1998, entitled "Bonding Process," with the named inventors Lisa A. DeLouise and David J. Luca, the disclosure of which is totally incorporated herein by reference, discloses a process for bonding a first article to a second article which comprises (a) providing a first article comprising a polymer having photosensitivity-imparting substituents; (b) providing a second article comprising metal, plasma nitride, silicon, or glass; (c) applying to at least one of the first article and the second article an adhesion pro-

63

motor selected from silanes, titanates, or zirconates having (i) alkoxy, aryloxy, or arylalkyloxy functional groups and (ii) functional groups including at least one photosensitive aliphatic  $>C=C<$  linkage; (d) placing the first article in contact with the second article; and (e) exposing the first article, second article, and adhesion promoter to radiation, thereby bonding the first article to the second article with the adhesion promoter. In one embodiment of the present invention, the adhesion promoter is employed in microelectrical mechanical systems such as thermal ink jet printheads.

Copending U.S. application Ser. No. 09/120,746, filed Jul. 23, 1998, entitled "Improved Thermal Ink Jet Printhead and Process for the Preparation Thereof," with the named inventors Ram S. Narang, Gary A. Kneezel, Bidan Zhang, Almon P. Fisher, and Timothy J. Fuller, the disclosure of which is totally incorporated herein by reference, discloses an ink jet printhead which comprises (i) an upper substrate with a set of parallel grooves for subsequent use as ink channels and a recess for subsequent use as a manifold, the grooves being open at one end for serving as droplet emitting nozzles, and (ii) a lower substrate in which one surface thereof has an array of heating elements and addressing electrodes formed thereon, said lower substrate having an insulative layer deposited on the surface thereof and over the heating elements and addressing electrodes and patterned to form recesses therethrough to expose the heating elements and terminal ends of the addressing electrodes, the upper and lower substrates being aligned, mated, and bonded together to form the printhead with the grooves in the upper substrate being aligned with the heating elements in the lower substrate to form droplet emitting nozzles, said upper substrate comprising a material formed by crosslinking or chain extending a polymer of formula I

5

10

15

20

25

30

35

40

45

50

55

60

65

64

the monomer repeat units of the polymer, A is



or mixtures thereof, B is



or II



wherein x is an integer of 0 or 1, P is a substituent which imparts photosensitivity to the polymer, a, b, c, and d are each integers of 0, 1, 2, 3, or 4, provided that at least one of a, b, c, and d is equal to or greater than 1 in at least some of



wherein z is an integer of from 2 to about 20, and preferably from 2 to about 10,



wherein u is an integer of from 1 to about 20, and preferably from 1 to about 10,



55 or mixtures thereof, and n is an integer representing the number of repeating monomer units.

Copending U.S. application Ser. No. 09/217,330, filed Dec. 21, 1998, entitled "Improved Photoresist Compositions," with the named inventors Thomas W. Smith, David J. Luca, and Kathleen M. McGrane, the disclosure of which is totally incorporated herein by reference, discloses a composition comprising a blend of (a) a thermally reactive polymer selected from the group consisting of resoles, novolacs, thermally reactive polyarylene ethers, and mixtures thereof; and (b) a photoreactive epoxy resin that is photoreactive in the absence of a photocationic initiator.

60 U.S. Pat. No. 5,738,799, filed Sep. 12, 1996, the disclosure of which is totally incorporated herein by reference,

discloses an ink-jet printhead fabrication technique which enables capillary channels for liquid ink to be formed with square or rectangular cross-sections. A sacrificial layer is placed over the main surface of a silicon chip, the sacrificial layer being patterned in the form of the void formed by the desired ink channels. A permanent layer, comprising permanent material, is applied over the sacrificial layer, and, after polishing the two layers to form a uniform surface, the sacrificial layer is removed. Preferred materials for the sacrificial layer include polyimide while preferred materials for the permanent layer include polyarylene ether, although a variety of material combinations are possible.

Copending U.S. application Ser. No. 08/705,914, filed Aug. 29, 1996, entitled "Thermal Ink Jet Printhead With Ink Resistant Heat Sink Coating," with the named inventors Ram S. Narang and Timothy J. Fuller, the disclosure of which is totally incorporated herein by reference, discloses a heat sink for a thermal ink jet printhead having improved resistance to the corrosive effects of ink by coating the surface of the heat sink with an ink resistant film formed by electrophoretically depositing a polymeric material on the heat sink surface. In one described embodiment, a thermal ink jet printer is formed by bonding together a channel plate and a heater plate. Resistors and electrical connections are formed in the surface of the heater plate. The heater plate is bonded to a heat sink comprising a zinc substrate having an electrophoretically deposited polymeric film coating. The film coating provides resistance to the corrosion of higher pH inks. In another embodiment, the coating has conductive fillers dispersed therethrough to enhance the thermal conductivity of the heat sink. In one embodiment, the polymeric material is selected from the group consisting of polyethersulfones, polysulfones, polyamides, polyimides, polyamide-imides, epoxy resins, polyetherimides, polyarylene ether ketones, chloromethylated polyarylene ether ketones, acryloylated polyarylene ether ketones, polystyrene and mixtures thereof.

U.S. Pat. No. 5,843,259, filed Aug. 29, 1996, entitled "Method for Applying an Adhesive Layer to a Substrate Surface," with the named inventors Ram S. Narang, Stephen F. Pond, and Timothy J. Fuller, the disclosure of which is totally incorporated herein by reference, discloses a method for uniformly coating portions of the surface of a substrate which is to be bonded to another substrate. In a described embodiment, the two substrates are channel plates and heater plates which, when bonded together, form a thermal ink jet printhead. The adhesive layer is electrophoretically deposited over a conductive pattern which has been formed on the binding substrate surface. The conductive pattern forms an electrode and is placed in an electrophoretic bath comprising a colloidal emulsion of a preselected polymer adhesive. The other electrode is a metal container in which the solution is placed or a conductive mesh placed within the container. The electrodes are connected across a voltage source and a field is applied. The substrate is placed in contact with the solution, and a small current flow is carefully controlled to create an extremely uniform thin deposition of charged adhesive micelles on the surface of the conductive pattern. The substrate is then removed and can be bonded to a second substrate and cured. In one embodiment, the polymer adhesive is selected from the group consisting of polyamides, polyimides, polyamide-imides, epoxy resins, polyetherimides, polysulfones, polyether sulfones, polyarylene ether ketones, polystyrenes, chloromethylated polyarylene ether ketones, acryloylated polyarylene ether ketones, and mixtures thereof.

Copending U.S. application Ser. No. 08/697,750, filed Aug. 29, 1996, entitled "Electrophoretically Deposited

Coating For the Front Face of an Ink Jet Printhead," with the named inventors Ram S. Narang, Stephen F. Pond, and Timothy J. Fuller, the disclosure of which is totally incorporated herein by reference, discloses an electrophoretic deposition technique for improving the hydrophobicity of a metal surface, in one embodiment, the front face of a thermal ink jet printhead. For this example, a thin metal layer is first deposited on the front face. The front face is then lowered into a colloidal bath formed by a fluorocarbon-doped organic system dissolved in a solvent and then dispersed in a non-solvent. An electric field is created and a small amount of current through the bath causes negatively charged particles to be deposited on the surface of the metal coating. By controlling the deposition time and current strength, a very uniform coating of the fluorocarbon compound is formed on the metal coating. The electrophoretic coating process is conducted at room temperature and enables a precisely controlled deposition which is limited only to the front face without intrusion into the front face orifices. In one embodiment, the organic compound is selected from the group consisting of polyimides, polyamides, polyamide-imides, polysulfones, polyarylene ether ketones, polyethersulfones, polytetrafluoroethylenes, polyvinylidene fluorides, polyhexafluoro-propylenes, epoxies, polypentafluorostyrenes, polystyrenes, copolymers thereof, terpolymers thereof, and mixtures thereof.

U.S. Pat. No. 5,939,206 the disclosure of which is totally incorporated herein by reference, discloses an apparatus which comprises at least one semiconductor chip mounted on a substrate, said substrate comprising a graphite member having electrophoretically deposited thereon a coating of a polymeric material. In one embodiment, the semiconductor chips are thermal ink jet printhead subunits. In one embodiment, the polymeric material is of the general formula



wherein x is an integer of 0 or 1, A is one of several specified groups, such as



69

B is one of several specified groups, such as



or mixtures thereof, and n is an integer representing the number of repeating monomer units.

Japanese Patent Publication 63-247757 A2, the disclosure of which is totally incorporated herein by reference, discloses an electrophotographic photosensitive body consisting of a body in which a photoconductive layer laminated on a conductive support contains a charge generating substance and/or a charge transporting substance, and at least one polyether ketone polymer consisting of structural units which can be expressed by the following general formulae (I) and (II)

(I)



(II)



wherein m is 0 or 1 and Ar indicates



wherein R is an alkyl group, n is 0, 1, or 2, and X indicates



70



with R' and R'' each independently indicating —H, —CH3, —C2H5,



15 wherein the proportion of structural units in the polymer expressed by the general formula (I) is from 0.1 to 1.0 and the proportion of structural units in the polymer expressed by the general formula (II) is 0 to 0.9.

20 U.S. Pat. No. 5,336,577 (Spiewak et al.), the disclosure of which is totally incorporated herein by reference, discloses a thick organic ambipolar layer on a photoresponsive device which is simultaneously capable of charge generation and charge transport. In particular, the organic photoresponsive layer contains an electron transport material such as a fluorenylidene malonitrile derivative and a hole transport material such as a dihydroxy tetraphenyl benzadine containing polymer. These may be complexed to provide photoresponsivity, and/or a photoresponsive pigment or dye may also be included.

30 U.S. Pat. No. 4,801,517 (Frechet et al.), the disclosure of which is totally incorporated herein by reference, discloses an electrostaticographic imaging member and an electrophotographic imaging process for using the imaging member in which the imaging member comprises a substrate and at 35 least one electroconductive layer, the imaging member comprising a polymeric arylamine compound represented by the formula



45 wherein n is between about 5 and 5,000, m is 0 or 1, Z is selected from certain specified aromatic and fused ring groups, Ar is selected from certain specified aromatic groups, R is selected from certain specified alkyl groups, Ar' is selected from certain specified aromatic groups, and R'' and R''' are independently selected from certain specified alkylene groups.

50 U.S. Pat. No. 4,806,443 (Yanus et al.), the disclosure of which is totally incorporated herein by reference, discloses an electrostaticographic imaging member and an electrophotographic imaging process for using the imaging member in which the imaging member comprises a substrate and an 55 electroconductive layer, the imaging member comprising a polymeric arylamine compound represented by the formula



60 wherein n is between 5 and about 5,000, m is 0 or 1, y is 1, 2, or 3, Z is selected from certain specified aromatic and

fused ring groups, Ar is selected from certain specified aromatic groups, Ar' is selected from certain specified aromatic groups, and X' is an alkylene radical selected from the group consisting of alkylene and isoalkylene groups containing 2 to 10 carbon atoms. The imaging member may comprise a substrate, charge generation layer, and a charge transport layer.

U.S. Pat. No. 4,806,444 (Yanus et al.) and U.S. Pat. No. 4,935,487 (Yanus et al.), the disclosures of each of which are totally incorporated herein by reference, disclose an electrostatographic imaging member and an electrophotographic imaging process for using the imaging member in which the imaging member comprises a substrate and an electroconductive layer, the imaging member comprising a polymeric arylamine compound represented by the formula



wherein n is between about 5 and about 5,000, m is 0 or 1, Z is selected from certain specified aromatic and fused ring groups, Ar is selected from certain specified aromatic groups, and Ar' is selected from certain specified aromatic groups. The imaging member may comprise a substrate, charge generation layer, and a charge transport layer.

U.S. Pat. No. 4,818,650 (Limburg et al.) and U.S. Pat. No. 4,956,440 (Limburg et al.), the disclosures of each of which are totally incorporated herein by reference, disclose an electrostatographic imaging member and an electrophotographic imaging process for using the imaging member in which the imaging member comprises a substrate and at least one electroconductive layer, the imaging member comprising a polymeric arylamine compound represented by the formula



wherein R is selected from the group consisting of  $-\text{H}$ ,  $-\text{CH}_3$ , and  $-\text{C}_2\text{H}_5$ , m is between about 4 and about 1,000, A is selected from the group consisting of an arylamine group represented by the formula



wherein m is 0 or 1, Z is selected from certain specified aromatic and fused ring groups that also contain an oxygen or sulfur atom, certain linear or cyclic hydrocarbon groups, and certain amine groups, Ar is selected from certain specified aromatic groups, Ar' is selected from certain specified aromatic groups, and B is selected from the group consisting of the arylamine group as defined for A and



wherein Ar is as defined above and V is selected from an oxygen or sulfur atom, certain linear or cyclic hydrocarbon groups, or a phenylene group, and at least A or B contains the arylamine group. The imaging member may comprise a substrate, charge generation layer, and a charge transport layer.

U.S. Pat. No. 5,030,532 (Limburg et al.), the disclosure of which is totally incorporated herein by reference, discloses an electrostatographic imaging member comprising a support layer and at least one electrophotoconductive layer, said imaging member comprising a polyarylamine polymer represented by the formula



wherein n is between about 5 and about 5,000, or 0 if p>0, o is between about 9 and about 5,000, or is 0 if p>0 or n=0, p is between about 2 and about 100, or is 0 if n>0, X' and X'' are independently selected from a group having bifunctional linkages, Q is a divalent group derived from certain hydroxy terminated arylamine reactants, Q' is a divalent group derived from a hydroxy terminated polyarylamine containing the group defined for Q and having a weight average molecular weight between about 1,000 and about 80,000, and the weight average molecular weight of the polyarylamine polymer is between about 10,000 and about 1,000,000.

U.S. Pat. No. 5,438,082 (Helmer-Metzmann et al.) and U.S. Pat. No. 5,561,202 (Helmer-Metzmann et al.), the disclosures of each of which are totally incorporated herein by reference, disclose the production of a polymer electrolyte membrane from sulfonated aromatic polyether ketones. An aromatic polyether ketone of the formula



in which Ar is a phenylene ring having p- and/or m-bonds, Ar' is a phenylene, naphthylene, biphenylene, anthrylene, or other divalent aromatic unit, X, N, and M, independently of one another, are 0 or 1, Y is 0, 1, 2, or 3, and P is 1, 2, 3, or 4, is sulfonated and the sulfonic acid is isolated. At least 5 percent of the sulfonic groups in the sulfonic acid are converted into sulfonyl chloride groups, and these groups are reacted with an amine containing at least one crosslinkable substituent or a further functional group, and unreacted sulfonyl chloride groups are subsequently hydrolyzed. The resultant aromatic sulfonamide is isolated and dissolved in an organic solvent, the solution is converted into a film, and the crosslinkable substituents in the film are then crosslinked. In specific cases, the crosslinkable substituents can be omitted, in which case, sulfonated polyether ketone is converted into a film from solution. In another embodiment of the disclosed invention, the polymer may contain, in addition to units of the above formula, non-sulfonatable units such as those of the formula



In yet another embodiment of the disclosed invention, as disclosed in columns 8 and 9, mixtures of polymeric, crosslinkable sulfonamides and polymeric, non-crosslinkable, aromatic sulfonic acids can be converted jointly into membranes.

U.S. Pat. No. 4,623,558 (Lin), the disclosure of which is totally incorporated herein by reference, discloses a thermosetting plastisol dispersion composition comprising (1) poly(phenylene oxide) in powder form, which is insoluble in the reactive plasticizer at room temperature and plasticizable at a temperature at or above the fluxing temperature; (2) a liquid reactive plasticizer member of the group consisting of (a) at least one epoxide resin having an average of more than one epoxide group in the molecule, (b) at least one liquid monomer, oligomer, or prepolymer containing at least one ethylenically unsaturated group, and (c) a mixture of (a) and (b), said reactive plasticizer being capable of solvating the poly(phenylene oxide) at the fluxing temperature and being present in an amount ranging from 5 to 2,000 parts per 100 parts by weight of (1); and (3) 0.01 to 10 percent by weight of (2) of either a thermal initiator or photoinitiator for plasticizers present in the composition. The plastisol dispersion after fluxing can form a thermoset after the crosslinking reaction.

U.S. Pat. No. 4,667,010 (Eldin), the disclosure of which is totally incorporated herein by reference, discloses linear polyether resins containing 100 to 10 mol % of the repeating structural unit of formula I



and 90 to 0 mol % of the repeating structural unit of formula 10 II



20 wherein A is a linear unsubstituted or methyl-substituted alkylene group containing 4 to 100 carbon atoms in the linear alkylene chain, X is



wherein R is C<sub>1</sub>-C<sub>8</sub> alkyl or



wherein each of R<sup>1</sup> and R<sup>2</sup> is a hydrogen or a halogen atom, and Y is



wherein R<sup>3</sup> and R<sup>4</sup> are the same or different and each is a halogen atom, C<sub>1</sub>-C<sub>4</sub> alkyl, or C<sub>1</sub>-C<sub>4</sub> alkoxy, m and n are 0 or an integer from 1 to 4, and Z is a direct bond or a radical selected from the group consisting of





wherein each of R<sup>5</sup> and R<sup>6</sup> independently of the other is a hydrogen atom, C<sub>1</sub>–C<sub>4</sub> alkyl, or phenyl,



The resins are self-crosslinkable and can be crosslinked by heating to a temperature of not less than 250° C. or by 25 irradiation with energy-rich electromagnetic rays, affording products which are insoluble in organic solvents and which

ings. Upon selected exposure of the film or coating to imaging energies, the photosensitive species within the composition either itself undergoes a degradative reaction or promotes degradation of one or more of the other components of the composition. This selective modification can then be simply manifested by contacting the exposed surface of the film or coating, subsequent to such exposure, with an alkaline developing solution. The compositions are useful in the graphic arts and in the manufacture of printed circuit boards for the electronics industry.

U.S. Pat. No. 3,455,868 (D'Alessandro), the disclosure of which is totally incorporated herein by reference, discloses a friction composition of particulate friction material and a binder of a heat-hardenable resin and a thermoplastic polyarylene polyether. The thermoplastic polyarylene polyether is linear and of the basic structure composed of recurring units having the formula



20 wherein E is the residuum of the dihydric phenol and E' is the residuum of the benzenoid compound having an inert electron withdrawing group in at least one of the positions ortho and para to the valence bonds, and wherein both of 25 said residua are valently bonded to the ether oxygens through aromatic carbon atoms. Preferred linear thermoplastic polyarylene polyethers are composed of recurring units having the formula



35

have high glass transition temperatures. The heat crosslinking can, if desired, be carried out in the presence of radical formers such as inorganic or organic peroxides, including potassium peroxide sulfate or benzoyl peroxide, azo compounds such as azoisobutyronitrile, organic hydroperoxides, (x-haloacetophenones, benzoins or ethers thereof, benzophenones, benzil acetals, anthraquinones, arsines, phosphines, or thioureas. Crosslinking can also be carried out with energy-rich rays such as X-rays, accelerated electrons, or  $\gamma$ -rays emitted from a  $^{60}\text{Co}$  source.

U.S. Pat. No. 5,268,444 (Jensen et al.), the disclosure of which is totally incorporated herein by reference, discloses phenylethynyl-terminated poly(arylene ethers) which are prepared in a wide range of molecular weights by adjusting the monomer ratio and adding an appropriate amount of 4-fluoro-4'-phenylethynylbenzophenone during polymer synthesis. The resulting phenylethynyl-terminated poly(arylene ethers) react and crosslink upon curing for one hour at 350° C. to provide materials with improved solvent resistance, higher modulus, and better high temperature properties than the linear, uncrosslinked polymers.

U.S. Pat. No. 4,435,496 (Walls et al.), the disclosure of which is totally incorporated herein by reference, discloses novel photosensitive compositions containing a compound consisting essentially of repeating structural units of an alkyl aryl ether, which are endcapped with a substituent functional group containing an ethylenically unsaturated moiety, and a photosensitizing effective amount of a free radical generating compound. Through the selected exposure of films and coatings prepared from the composition, it is possible to record information in the materials in a manner to alter the physical and/or chemical properties of the films and coat-

40 groups selected from the group consisting of halogen, alkyl groups having from 1 to 4 carbon atoms, and alkoxy groups having from 1 to 4 carbon atoms, and where r and z are integers having a value from 0 to 4 inclusive, and preferably having a value of 0. In Example 14, the polyarylene polyether is of 45 the formula



50 U.S. Pat. No. 5,336,720 (Richards et al.), the disclosure of which is totally incorporated herein by reference, discloses an impact resistant graft polymer and an emulsion polymerization process comprising (1) an agglomerated rubber latex made from a rubber latex and a polymerized polymeric additive, and (2) a grafted polymer. Specifically, the graft polymer comprises: 1) from about 60 to about 95 parts by weight or more (as weight of solid component) of an agglomerated rubber latex (C) having the following composition:

55 (a) 100 parts by weight (as weight of solid component) of a synthetic rubber latex (A) having particle distribution between about 60 and about 200 nm, and a pH from about 8.0 to about 10.0; and

(b) from about 0.1 to about 5.0 parts by weight (as weight of solid component) of a polymerized polymeric additive (B) having an average particle diameter of about 100 to about 300 nm, and formed by polymerizing:

- (1) one or more monomer groups where at least one monomer group always contains at least 30% by weight of unsaturated carboxylic acid selected from acrylic acid, methacrylic acid, itaconic acid, acryloxypropionic acid, crotonic acid, and the like;
- (2) from about 5 to about 70% (by weight) of at least one alkyl acrylate having  $C_1-C_{12}$  alkyl group (such as methyl methacrylate, hydroxyethyl methacrylate, butyl acrylate, and the like; and
- (3) up to 80% (by weight) of other copolymerizable monomer(s); and

2) from about 5 to about 40 parts by weight of a grafted polymer (D) formed by polymerizing (a) 30% by weight or more of at least one monomer selected from styrene, acrylonitrile, methyl methacrylate, hydroxyethyl methacrylate, butyl acrylate, ethyl acrylate, and the like; and (b) 30% by weight or less of a vinyl monomer having  $CH_2=C<$  copolymerizable therewith. As stated at columns 4 an 5, bridging paragraph, in the preparation of the (B) component, the "other copolymerizable monomers" can be unsaturated aromatic compounds such as styrene, alpha-methylstyrene, and vinyltoluene; unsaturated nitrile compounds such as acrylonitrile and methacrylonitrile; alkyl methacrylates having  $C_1-C_{12}$  alkyl group, such as butyl acrylate and hydroxyethylmethacrylate; and diolefins such as butadiene. Crosslinkers or graftlinkers such as ethylenically unsaturated esters (e.g., allyl methacrylate and methallyl methacrylate, 1,3-butylene glycol dimethacrylate, trimethyl glycol propane triacrylate, and the like), or other ethylenically unsaturated monomers (e.g., divinyl benzene and trivinyl benzene) may be used, at levels typically less than or equal to 2% by weight.

EP 0 281 808, the disclosure of which is totally incorporated herein by reference, discloses a thermally stable radiation crosslinkable polymer system which cures without additional heat treatment which comprises a main component A which is a polyether acrylate or a compound in accordance with one of the structural formulae

CHY<sub>2</sub>

(1)

CHY<sub>2</sub>—CHY<sub>2</sub>

(2)



(3)

wherein Y denotes a radical of the structure



in which X is H, Cl, or OH and where A denotes the acyl radical of a substituted acrylic acid, and 1 to 10 percent by weight of a component B, different therefrom, as a crosslinking intensifier, which component B is selected from pentaerythritol triacrylate or tetraacrylate, dipentaerythritol pentaacrylate, or trimethylolpropane triacrylate. In one spe-

cific embodiment, the polyether acrylate has the general structure



JP 60-57826, the disclosure of which is totally incorporated herein by reference, discloses azido group containing polyether sulfones containing a repeating unit of the formula



wherein Ar<sub>1</sub> represents an aromatic hydrocarbon group with carbon number 6 to 10 (2+p), Ar<sub>2</sub> represents an aromatic hydrocarbon group with carbon number 6 to 10 (2+q), Ar<sub>3</sub> represents a divalent aromatic group with carbon number 6 to 15, and p and q represent 0, 1, or 2 and satisfy p+q=1 to 4. Specific examples of Ar<sub>1</sub> and Ar<sub>2</sub> include



methyl substitutes of the above,



-continued

Examples of suitable  $\text{Ar}_3$  groups include

and



The resin is heat resistant and photosensitive, and suitable for use as a photoresist for microprocessing.

JP 56-050929, the disclosure of which is totally incorporated herein by reference, discloses a polysulfone characterized by having a carbon-carbon double bond in the side chain, represented by the formula



15 wherein  $\text{Ar}_1$  is a  $(2+p)$  valence aromatic hydrocarbon group having 6 to 10 carbon atoms,  $\text{Ar}_2$  is a  $(2+q)$  valence aromatic hydrocarbon group having 6 to 10 carbon atoms,  $\text{Ar}_3$  is a divalent aromatic hydrocarbon group having 6 to 15 carbon atoms,  $-\text{X}_{11}-$  and  $-\text{X}_{12}-$  are the same or different and show connecting  $-\text{O}-$  or  $-\text{NR}_3-$ ,  $\text{R}_3$  is a hydrogen atom or univalent hydrocarbon group having 1 to 10 carbon atoms,  $\text{R}_{11}$  and  $\text{R}_{12}$  are the same or different and hydrogen atoms or methyl groups,  $\text{R}_{21}$  and  $\text{R}_{22}$  are the same or different and hydrogen atoms or phenyl groups,  $\text{r}_{21}$  and  $\text{r}_{22}$  are independently 1 or 2,  $\text{p}$  and  $\text{q}$  are independently 0, 1, or 2, and the equation  $\text{p}+\text{q}=1$  to 4 must be satisfied.

JP 56-050928, the disclosure of which is totally incorporated herein by reference, discloses a polysulfone characterized by having, in the side chain, a (meth)acrylate group comprising a constituting unit represented by the following general formula (I):



35 wherein  $\text{Ar}_1$  is a  $(2+p)$  valence aromatic hydrocarbon group having 6 to 10 carbon atoms,  $\text{Ar}_2$  is a  $(2+q)$  valence aromatic hydrocarbon group having 6 to 10 carbon atoms,  $\text{Ar}_3$  is a divalent aromatic hydrocarbon group having 6 to 15 carbon atoms which may contain the hetero atom S or O,  $-\text{X}_1-$  and  $-\text{X}_2-$  are the same or different and show connecting  $-\text{O}-$  or  $-\text{NR}_3-$ ,  $\text{R}_1$  is a hydrogen atom or univalent hydrocarbon group having 1 to 10 carbon atoms,  $\text{R}_2$  is an alkyl group having 2 to 5 carbon atoms, and furthermore,  $\text{R}_3$  is a hydrogen atom or methyl group;  $\text{p}$  and  $\text{q}$  are independently 0, 1, or 2, and the equation  $\text{p}+\text{q}=1$  to 4 must be satisfied.

U.S. Pat. No. 4,086,209 (Hara et al.), the disclosure of which is totally incorporated herein by reference, discloses substantially linear or at least partially crosslinked nitrogen-containing polymers having an aryleneimine or aryleneether unit in the main chain with an amino group or a group

81

derived from it being bonded as a pendant group to a nuclear carbon atom of the arylene group of the above unit. According to the number and type of the pendant groups, the polymers can have various useful properties such as thermal stability, hydrophilicity, oxidative reducibility, photosensitivity, color formability, or the ability to form coordination bonds. Further, the polymers have good solubility in aprotic polar organic solvents. Permselective membranes having good performance can be prepared from solutions of the polymers in these solvents.

EP 0 663 411, the disclosure of which is totally incorporated herein by reference, discloses a photoimaging resist ink containing (A) an unsaturated group-having polycarboxylic acid resin which is a reaction product of (c) succinic anhydride with an additive reaction product of (a) an epoxy resin with (b) an unsaturated group-having monocarboxylic acid, wherein (a) the epoxy resin is represented by the formula



wherein  $M$  stands for



n is at least 1 on the average, and m is 1 to n on the average. In specific embodiments, the resist further contains (B) a photopolymerization initiator, (C) a diluent, and (D) a curing component. In forming a solder resist pattern by exposing a coating film of a resist ink through a patterned film to ultraviolet light and developing the coating film to dissolve away the unexposed portions thereof, the resist ink is excellent in developability and photosensitivity, while the cure product thereof is excellent in flex resistance and folding resistance, heat resistance, and the like. The resist ink is especially suitable as a liquid solder resist ink for flexible printed circuit boards and thin pliable rigid circuit boards.

U.S. Pat. No. 4,448,948 (Tsubaki et al.), the disclosure of which is totally incorporated herein by reference, discloses an epoxy resin substantially represented by the general formula



wherein  $\text{Ar}^1$  is a residual group of a dihydric phenol derived from a compound having one or two benzene nuclei,  $\text{Ar}^2$  is a residual group of a halogen-substituted benzenoid compound having two halogen atoms on its nuclei and represented by the formula 60

82

wherein each of  $\text{Ar}^3$  and  $\text{Ar}^4$  is a hydrocarbon group having a divalent benzene nucleus and  $\text{Y}$  is a sulfone group or a carbonyl group, and  $n$  is an integer of from 1 to 50.

U.S. Pat. No. 5,728,498 (Yanus et al.), the disclosure of which is totally incorporated herein by reference, discloses a flexible electrophotographic imaging member including a supporting substrate coated with at least one imaging layer comprising hole transporting material containing at least two long chain alkyl carboxylate groups dissolved or molecularly dispersed in a film forming binder. Preferred charge transporting materials are of the formula



wherein m is 0 or 1, Z is selected from the group consisting of



and

-continued



$$-\text{Ar}^3-\text{Y}-\text{Ar}^4-$$

83

n is 0 or 1, Ar is selected from the group consisting of



R is selected from the group consisting of  $-\text{CH}_3$ ,  $-\text{C}_2\text{H}_5$ ,  $-\text{C}_3\text{H}_7$ , and  $-\text{C}_4\text{H}_9$ , Ar' is selected from the group consisting of



X is selected from the group consisting of  $-\text{CH}_2-$ ,  $-\text{C}(\text{CH}_3)_2-$ ,  $-\text{O}-$ ,  $-\text{S}-$ ,



84

s is 0, 1, or 2, and Q is represented by the formula



wherein p is 1 or 0,  $\text{R}_1$ ,  $\text{R}_2$ ,  $\text{R}_3$ ,  $\text{R}_4$  are independently selected from  $-\text{H}$ ,  $-\text{CH}_3$ ,  $-(\text{CH}_2)_v\text{CH}_3$ ,  $-\text{CH}(\text{CH}_3)_2$ ,  $-\text{C}(\text{CH}_3)_3$ , wherein v is 1 to 10, and s and n are independently selected from 0 to 10.

Copending U.S. application Ser. No. 09/326,169, filed concurrently herewith, entitled "Arylene Ether Alcohol Polymers," with the named inventors Timothy J. Fuller, John F. Yanus, Damodar M. Pai, Markus R. Silvestri, Ram S. Narang, William W. Limburg, and Dale S. Renfer, the disclosure of which is totally incorporated herein by reference, discloses a polymer of the formula



wherein A is



35 or a mixture of



wherein R is a hydrogen atom, an alkyl group, an aryl group, or mixtures thereof, B is one of specified groups, such as



60 or mixtures thereof, and n is an integer representing the number of repeating monomer units.

Copending U.S. application Ser. No. 09/325,837, filed concurrently herewith, entitled "Ink Jet Printheads Containing Arylene Ether Alcohol Polymers," with the named inventors Timothy J. Fuller, John F. Yanus, Damodar M. Pai, Markus R. Silvestri, Ram S. Narang, William W. Limburg, and Dale S. Renfer, the disclosure of which is totally

incorporated herein by reference, discloses an ink jet print-head containing a polymer of the formula



wherein P is a substituent which enables crosslinking of the polymer, a, b, c, and d are each integers of 0, 1, 2, 3, or 4, provided that at least one of a, b, c, and d is equal to or greater than 1 in at least some of the monomer repeat units of the polymer. A is



or a mixture of



wherein R is a hydrogen atom, an alkyl group, an aryl group, or mixtures thereof, B is one of specified groups, such as



or mixtures thereof, and  $n$  is an integer representing the number of repeating monomer units.

While known compositions and processes are suitable for their intended purposes, a need remains for improved photosensitive imaging members. A need also remains for improved binders for photosensitive imaging members. In addition, there is a need for polymeric binders suitable for use in photogenerating layers in imaging members. Further, a need remains for polymeric binders suitable for use in charge transport layers in imaging members. Additionally, there is a need for polymeric binders with high glass transition temperatures. There is also a need for polymeric binders which enable the incorporation of high loadings of charge transport materials and/or plasticizers therein. In addition, a need remains for polymeric binders which exhibit good film properties and good adhesion to imaging member substrates. Further, a need remains for polymeric binders for imaging members which have high resistance to 55 60 65

a wide variety of solvents. Additionally, a need remains for polymeric binders suitable for charge transport layers in imaging members which enable incorporation of charge transport materials such as N,N'-diphenyl-N,N'-bis(3"-methylphenyl)-(1,1'-biphenyl)-4,4'-diamine in the layer in amounts of 50 percent by weight and higher without resulting in severe plasticization. There is also a need for polymeric binders which can be coated onto photosensitive imaging members from a wide variety of solvents. Further, a need remains for polymeric binders in which charge transport molecules exhibit reduced or eliminated tendency to crystallize. In addition, there is a need for polymeric binders which have a reduced tendency to crystallize compared to widely used photoreceptor binder polymers. There is also a need for abrasion resistant and wear resistant photoconductive imaging members. Further, there is a need for photoconductive imaging members which are flat after oven drying. Additionally, there is a need for polymeric binders and transport polymers with improved wear and abrasion resistance compared to known polymers commonly used in photoconductive imaging members. A need also remains for photoconductive imaging members which are curl-free and stress-free after removal of coating solvents. In addition, a need remains for polymers suitable for use as adhesive layer materials in photoconductive imaging members. Further, a need remains for polymers suitable for use as protective overcoating layer materials in photoconductive imaging members. Additionally, a need remains for polymers which, when mixed with a solvent and coated onto an imaging member, adhere well to materials commonly used as photoconductive imaging member overcoats (such as LUCKAMIDE), particularly when the polymer is subjected to a one-shot drying process, wherein the overcoat is coated onto the layer containing the polymer of the present invention before said layer has dried. There is also a need for polymers that, when incorporated into photoconductive imaging members, exhibit improved wear resistance to bias charging rolls, including improvements of up to twice the wear resistance observed for commonly used, such as polycarbonates based on 1,1-cyclohexyl-4,4'-bisphenol.

## SUMMARY OF THE INVENTION

The present invention is directed to an imaging member which comprises a conductive substrate, a photogenerating material, and a binder comprising a polymer of the formula



$\epsilon_0$  wherein A is



or a mixture of



wherein R is a hydrogen atom, an alkyl group, an aryl group, or mixtures thereof, B is



-continued



10 wherein v is an integer of from 1 to about 20,



20 wherein z is an integer of from 2 to about 20,



30 wherein u is an integer of from 1 to about 20,



wherein w is an integer of from 1 to about 20,



89

-continued



90

wherein (1) Z is



wherein  $R_1$  and  $R_2$  each, independently of the other, are hydrogen atoms, alkyl groups, or aryl groups, and  $p$  is an integer of 0 or 1,

30 wherein  $p$  is 0 or 1; (2) Ar is

wherein  $p$  is an integer of 0 or 1,

$\text{---}(\text{CH}_2\text{O})_t\text{---}$

wherein  $t$  is an integer of from 1 to about 20,



50 (3) G is an alkyl group selected from alkyl or isoalkyl groups containing from about 2 to about 10 carbon atoms; (4) Ar' is



(5) X is



wherein  $s$  is 0, 1, or 2,



and (6) q is 0 or 1; or mixtures thereof, hydroxy-substituted, hydroxyalkyl-substituted, or hydroxyaryl-substituted derivatives thereof, or mixtures thereof, and n is an integer representing the number of repeating monomer units. 40

In one specific embodiment of the present invention, the polymer is of the formula 45



wherein P is a substituent which enables crosslinking of the polymer, a, b, c, and d are each integers of 0, 1, 2, 3, or 4, provided that at least one of a, b, c, and d is equal to or greater than 1 in at least some of the monomer repeat units of the polymer. 60

In another specific embodiment of the present invention, 65 the polymer is prepared by a process which comprises (1) providing a precursor polymer of the formula



wherein A is



B is



93

-continued



wherein v is an integer of from 1 to about 20,



wherein  $z$  is an integer of from 2 to about 20,



wherein  $u$  is an integer of from 1 to about 20,



94

wherein w is an integer of from 1 to about 20,



35 wherein  $R_1$  and  $R_2$  each, independently of the other, are hydrogen atoms, alkyl groups, or aryl groups, and  $p$  is an integer of 0 or 1,



45

wherein  $p$  is an integer of 0 or 1.

58

$$-(\text{CH}_2\text{O})_t-$$

wherein  $t$  is an integer of from 1 to about 20,



95



wherein (1) Z is



wherein p is 0 or 1; (2) Ar is



(3) G is an alkyl group selected from alkyl or isoalkyl groups containing from about 2 to about 10 carbon atoms; (4) Ar' is



96



10 (5) X is



wherein s is 0, 1, or 2,



45 and (6) q is 0 or 1; or mixtures thereof, hydroxy-substituted, hydroxyalkyl-substituted, or hydroxyaryl-substituted derivatives thereof, or mixtures thereof, and n is an integer representing the number of repeating monomer units, and  
 50 (2) reacting the precursor polymer with borane, resulting in formation of a polymer of the formula



60 wherein A is



97

or a mixture of



wherein R is a hydrogen atom, an alkyl group, an aryl group, or mixtures thereof.

In yet another specific embodiment of the present invention, the polymer is prepared by a process which comprises (1) providing a precursor polymer of the formula



wherein A is



B is



98

-continued



wherein v is an integer of from 1 to about 20,



wherein z is an integer of from 2 to about 20,



wherein u is an integer of from 1 to about 20,



99

-continued



wherein w is an integer of from 1 to about 20,



wherein  $R_1$  and  $R_2$  each, independently of the other, are hydrogen atoms, alkyl groups, or aryl groups, and  $p$  is an integer of 0 or 1,



wherein  $p$  is an integer of 0 or 1,

100

wherein  $t$  is an integer of from 1 to about 20,



wherein (1) Z is



55 wherein p is 0 or 1; (2) Ar is



$$-(\text{CH}_2\text{O})_i-$$

101

-continued



(3) G is an alkyl group selected from alkyl or isoalkyl groups containing from about 2 to about 10 carbon atoms; (4) Ar is or



or



(5) X is



wherein s is 0, 1, or 2,



and (6) q is 0 or 1; or mixtures thereof, hydroxy-substituted, hydroxyalkyl-substituted, or hydroxyaryl-substituted derivatives thereof, or mixtures thereof, and n is an integer representing the number of repeating monomer units, (2) reacting the precursor polymer with a reagent of the formula  $\text{RMgX}$ , wherein R is a hydrogen atom, an alkyl group, an

102

aryl group, or mixtures thereof and X is a halogen atom, and (3) subsequent to step 2, adding water or acid to the precursor polymer, thereby resulting in formation of a polymer of the formula

5



10

wherein A is



20 or a mixture of



25

wherein R is a hydrogen atom, an alkyl group, an aryl group, or mixtures thereof.

## 30 BRIEF DESCRIPTION OF THE DRAWINGS

FIGS. 1, 2, 3, and 4 are schematic cross-sectional views of examples of photoconductive imaging members of the present invention.

35

## DETAILED DESCRIPTION OF THE INVENTION

The present invention is directed to photosensitive imaging members containing polymers of the general formula

40



45 wherein A is



50 or a mixture of



55

wherein R is a (a) hydrogen atom, (b) an alkyl group, including unsubstituted alkyl groups and substituted alkyl groups, such as hydroxyalkyl groups, preferably with from 1 to about 20 carbon atoms, more preferably with from 1 to about 10 carbon atoms, and even more preferably with from

103

1 to about 5 carbon atoms, although the number of carbon atoms can be outside of this range, (c) an aryl group, including unsubstituted aryl groups and substituted aryl groups, such as hydroxyaryl groups, preferably with from 6 to about 18 carbon atoms, more preferably with from 6 to about 12 carbon atoms, and even more preferably with 6 carbon atoms, although the number of carbon atoms can be outside of this range, or (d) mixtures thereof, B is



25 wherein z preferably is an integer of from 2 to about 20, and more preferably from 2 to about 10,



35 wherein u preferably is an integer of from 1 to about 20, and more preferably from 1 to about 10,



65 wherein w preferably is an integer of from 1 to about 20, and more preferably from 1 to about 10,

**105**

wherein R<sub>1</sub> and R<sub>2</sub> each, independently of the other, are (a) hydrogen atoms, (b) alkyl groups, including unsubstituted alkyl groups and substituted alkyl groups, such as hydroxyalkyl groups, preferably with from 1 to about 20 carbon atoms, more preferably with from 1 to about 10 carbon atoms, and even more preferably with from 1 to about 5 carbon atoms, although the number of carbon atoms can be outside of this range, (c) aryl groups, including unsubstituted aryl groups and substituted aryl groups, such as hydroxyaryl groups, preferably with 6 to about 18 carbon atoms, more preferably with 6 to about 12 carbon atoms, and even more preferably with 6 carbon atoms, although the number of carbon atoms can be outside of this range, or (d) mixtures thereof, and p is an integer of 0 or 1,



wherein p is an integer of 0 or 1,

—(CH<sub>2</sub>O)<sub>t</sub>—**106**

wherein t is an integer of from 1 to about 20,

5



10



15



20



25

wherein (1) Z is

30



40



45



50



wherein p is 0 or 1; (2) Ar is



or

55

60

or

65

-continued



(3) G is an alkyl group selected from alkyl or isoalkyl groups containing from about 2 to about 10 carbon atoms; (4) Ar' is



or



(5) X is



wherein s is 0, 1, or 2,



and (6) q is 0 or 1; or mixtures thereof, hydroxy-substituted derivatives thereof, hydroxyalkyl-substituted derivatives thereof, with the hydroxyalkyl substituents preferably having from 1 to about 20 carbon atoms, more preferably from 1 to about 10 carbon atoms, and even more preferably from 1 to about 5 carbon atoms, although the number of carbon atoms can be outside of this range, hydroxyaryl-substituted

derivatives thereof, with the hydroxyaryl substituents preferably having from 6 to about 18 carbon atoms, more preferably from 6 to about 12 carbon atoms, and even more preferably about 6 carbon atoms, although the number of carbon atoms can be outside of this range, or mixtures thereof, and n is an integer representing the number of repeating monomer units. Specific examples of some preferred substituted derivatives include (but are not limited to)



15

wherein m and n are each integers of 0, 1, or 2,



20

wherein m and n are each integers of 0, 1, or 2,



35

wherein m, n, p, and q are each integers of 0, 1, or 2,



40



45

wherein m and n are each integers of 0, 1, or 2, and the like. Desirable values for n, and the corresponding weight average molecular weight and number average molecular weight, depend on the desired use for the polymer. For example, when the polymer is to be used as a binder polymer in an imaging member (either substituted or unsubstituted with crosslinking groups), the value of n is preferably such that the number average molecular weight of the material is

50 from about 10,000 to about 100,000, more preferably is from about 30,000 to about 100,000, and even more preferably is from about 30,000 to about 60,000, although the Mn can be outside these ranges; the weight average molecular weight of the material preferably is from about 20,000 to about 350,000, and more preferably is from about 100,000 to about 250,000, although the Mw can be outside these ranges; and the polydispersity (Mw/Mn) typically is from about 2 to about 9, and preferably is about 3, although higher or lower polydispersity values may also be used. The phenyl groups and the A and/or B groups may also be substituted, although the presence of two or more substituents on the B group ortho to the oxygen groups can render substitution difficult

109

when it is desired to place crosslinking functional groups onto the polymer. Substituents can be present on the polymer either prior to or subsequent to the placement of crosslinking functional groups thereon. Substituents can also be placed on the polymer during the process of placement of crosslinking functional groups thereon. Substituents and/or crosslinking groups can be placed on the polymer before, during, or after preparation of the polymer of the basic formula



Examples of suitable substituents include (but are not limited to) alkyl groups, including saturated, unsaturated, and cyclic alkyl groups, preferably with from 1 to about 6 carbon atoms, substituted alkyl groups, including saturated, unsaturated, and cyclic substituted alkyl groups, preferably with from 1 to about 6 carbon atoms, aryl groups, preferably with from 6 to about 24 carbon atoms, substituted aryl groups, preferably with from 6 to about 24 carbon atoms, arylalkyl groups, preferably with from 7 to about 30 carbon atoms, substituted arylalkyl groups, preferably with from 7 to about 30 carbon atoms, alkoxy groups, preferably with from 1 to about 6 carbon atoms, substituted alkoxy groups, preferably with from 1 to about 6 carbon atoms, aryloxy groups, preferably with from 6 to about 24 carbon atoms, substituted aryloxy groups, preferably with from 6 to about 24 carbon atoms, arylalkyloxy groups, preferably with from 7 to about 30 carbon atoms, substituted arylalkyloxy groups, preferably with from 7 to about 30 carbon atoms, hydroxy groups, and the like.

One preferred embodiment of the present invention is directed to a photosensitive imaging member containing a polymer of the formula



wherein  $n$  is an integer representing the number of repeating monomer units. Another preferred embodiment of the present invention is directed to a photosensitive imaging member containing a polymer of the formula



wherein  $n$  is an integer representing the number of repeating 60 monomer units.

Polymers useful for the imaging members of the present invention can be prepared by any desired or suitable process. For example, the polymers can be prepared by providing the corresponding poly(arylene ether ketone) and then reducing 65 the poly(arylene ether ketone) with borane to form the poly(arylene ether alcohol), as follows:

110



Typically, about 10 parts by weight of the corresponding poly(arylene ether ketone) are dissolved in about 100 grams of a suitable solvent, such as tetrahydrofuran, to which is added under inert atmosphere (such as argon) and with mechanical stirring a one Molar solution of a borane-tetrahydrofuran complex in tetrahydrofuran (available from, for example, Aldrich Chemical Co., Milwaukee, Wis.). 20 Generally, one mole of the borane-tetrahydrofuran complex is added for each polymeric carbonyl group to assure complete reduction of the carbonyl groups. Some or all of the keto groups can be reduced, depending on the amount of borane-tetrahydrofuran complex added. When not all of the carbonyl groups are reduced to alcohol groups, preferably at least about 0.1 percent of the carbonyl groups are reduced, more preferably at least about 10 percent of the carbonyl groups are reduced, and even more preferably at least about 30 percent of the carbonyl groups are reduced. Most 30 preferably, about 100 percent of the carbonyl groups are reduced.

Hydroxymethyl groups can also be placed on the polymer by using as a starting material the corresponding poly(arylene ether ketone) substituted with, for example, acetyl groups, as follows:





The backbone carbonyl groups are reduced by the borane-tetrahydrofuran complex at 25° C.; the pendant acetyl groups, however, generally are reduced under elevated temperatures (e.g., tetrahydrofuran boiling at reflux for up to about 2 hours). One mole of the borane-tetrahydrofuran complex is added to reduce each mole of acetyl groups to the corresponding hydroxymethyl groups.

The polymers for the imaging members of the present invention can also be prepared via a Grignard process. Specifically, about 10 parts by weight of the polymer in about 100 parts by weight of dry tetrahydrofuran are reacted with one molar equivalent of the Grignard reagent (RMgX, wherein R is the group ultimately added to the carbonyl bond in the polymer and X is a halogen, such as chlorine, bromine, or iodine) at ambient temperature (about 25° C.) with mechanical stirring under an inert atmosphere (such as argon). Subsequent addition of water or an acid yields the product. The reaction proceeds as follows:



The corresponding polyarylene ether ketone can be prepared by any desired or suitable process. Processes for the preparation of these materials are known, and disclosed in, for example, U.S. Pat. No. 5,849,809, U.S. Pat. No. 5,739,254, U.S. Pat. No. 5,753,783, U.S. Pat. No. 5,761,809, U.S. Pat. No. 5,863,963, U.S. Pat. No. 5,814,426, U.S. Pat. No. 5,874,192, Copending U.S. application Ser. No. 08/705,375, Copending U.S. application Ser. No. 09/221,024, Copending U.S. application Ser. No. 08/159,426, Copending U.S. application Ser. No. 08/705,488, Copending U.S. application Ser. No. 09/221,690, Copending U.S. application Ser. No. 08/697,761, Copending U.S. application Ser. No. 09/221,278, Copending U.S. application Ser. No. 08/705,376, Copending U.S. application Ser. No. 09/220,273, Copending U.S. application Ser. No. 08/705,372, Copending U.S. application Ser. No. 09/246,167, Copending U.S. application Ser. No. 09/163,672, Copending U.S. application Ser. No. 08/697,760, Copending U.S. application Ser. No. 09/247,

- 104, Copending U.S. application Ser. No. 08/976,238, Copending U.S. application Ser. No. 09/105,501, Copending U.S. application Ser. No. 09/120,746, and Copending U.S. application Ser. No. 09/217,330, the disclosures of each of which are totally incorporated herein by reference. Further background material is contained in, for example, P. M. Hergenrother, *J. Macromol. Sci. Rev. Macromol. Chem.*, C19 (1), 1-34 (1980); P. M. Hergenrother, B. J. Jensen, and S. J. Havens, *Polymer*, 29, 358 (1988); B. J. Jensen and P.M. Hergenrother, "High Performance Polymers," Vol. 1, No. 1) page 31 (1989), "Effect of Molecular Weight on Poly(arylene ether ketone) Properties"; V. Percec and B. C. Auman, *Makromol. Chem.* 185, 2319 (1984); "High Molecular Weight Polymers by Nickel Coupling of Aryl Polychlorides," I. Colon, G. T. Kwiatkowski, *J. of Polymer Science, Part A, Polymer Chemistry*, 28, 367 (1990); M. Ueda and T. Ito, *Polymer J.*, 23 (4), 297 (1991), "Ethynyl-Terminated Polyarylates: Synthesis and Characterization," S. J. Havens and P. M. Hergenrother, *J. of Polymer Science: Polymer Chemistry Edition*, 22, 3011 (1984); "Ethynyl-Terminated Polysulfones: Synthesis and Characterization," P. M. Hergenrother, *J. of Polymer Science: Polymer Chemistry Edition*, 20, 3131 (1982); K. E. Dukes, M. D. Forbes, A. S. Jeevarajan, A. M. Belu, J. M. DeDimone, R. W. Linton, and V. V. Sheares, *Macromolecules*, 29, 3081 (1996); G. Hougham, G. Tesoro, and J. Shaw, *Polym. Mater. Sci. Eng.*, 61, 369 (1989); V. Percec and B. C. Auman, *Makromol. Chem.*, 185, 617 (1984); "Synthesis and characterization of New Fluorescent Poly(arylene ethers)," S. Matsuo, N. Yakoh, S. Chino, M. Mitani, and S. Tagami, *Journal of Polymer Science: Part A: Polymer Chemistry*, 32, 1071 (1994); "Synthesis of a Novel Naphthalene-Based Poly(arylene ether ketone) with High Solubility and Thermal Stability," Mami Ohno, Toshikazu Takata, and Takeshi Endo, *Macromolecules*, 27, 3447 (1994); "Synthesis and Characterization of New Aromatic Poly(ether ketones)," F. W. Mercer, M. T. Mckenzie, G. Merlino, and M. M. Fone, *J. of Applied Polymer Science*, 56, 1397 (1995); H. C. Zhang, T. L. Chen, Y. G. Yuan, Chinese Patent CN 85108751 (1991); "Static and laser light scattering study of novel thermoplastics. 1. Phenolphthalein poly(aryl ether ketone)," C. Wu, S. Bo, M. Siddiq, G. Yang and T. Chen, *Macromolecules*, 29, 2989 (1996); "Synthesis of t-Butyl-Substituted Poly(ether ketone) by Nickel-Catalyzed Coupling Polymerization of Aromatic Dichloride", M. Ueda, Y. Seino, Y. Haneda, M. Yoneda, and J. -I. Sugiyama, *Journal of Polymer Science: Part A: Polymer Chemistry*, 32, 675 (1994); "Reaction Mechanisms: Comb-Like Polymers and Graft Copolymers from Macromers 2. Synthesis, Characterization and Homopolymerization of a Styrene Macromer of Poly(2,6-dimethyl-1,4-phenylene Oxide)," V. Percec, P. L. Rinaldi, and B. C. Auman, *Polymer Bulletin*, 10, 397 (1983); *Handbook of Polymer Synthesis Part A*, Hans R. Kricheldorf, ed., Marcel Dekker, Inc., New York-Basel-Hong Kong (1992); and "Introduction of Carboxyl Groups into Crosslinked Polystyrene," C. R. Harrison, P. Hodge, J. Kemp, and G. M. Perry, *Die Makromolekulare Chemie*, 176, 267 (1975), the disclosures of each of which are totally incorporated herein by reference. Further background on high performance polymers is disclosed in, for example, U.S. Pat. No. 2,822,351; U.S. Pat. No. 3,065,205; British Patent 1,060,546; British Patent 971,227; British Patent 1,078,234; U.S. Pat. No. 4,175,175; N. Yoda and H. Hiramoto, *J. Macromol. Sci.-Chem.*, A21(13 & 14) pp. 1641 (1984) (Toray Industries, Inc., Otsu, Japan; B. Sillion and L. Verdet, "Polyimides and other High-Temperature polymers", edited by M. J. M. Abadie and B. Sillion,

Elsevier Science Publishers B.V. (Amsterdam 1991); "Polyimides with Alicyclic Diamines. II. Hydrogen Abstraction and Photocrosslinking Reactions of Benzophenone Type Polyimides," Q. Jin, T. Yamashita, and K. Horie, *J. of Polymer Science: Part A: Polymer Chemistry*, 32, 503 (1994); Probimide™ 300, product bulletin, Ciba-Geigy Microelectronics Chemicals, "Photosensitive Polyimide System;" *High Performance Polymers and Composites*, J. I. Kroschwitz (ed.), John Wiley & Sons (New York 1991); and T. E. Atwood, D. A. Barr, T. A. King, B. Newton, and B. J. Rose, *Polymer*, 29, 358 (1988), the disclosures of each of which are totally incorporated herein by reference. Further information on radiation curing is disclosed in, for example, *Radiation Curing: Science and Technology*, S. Peter Pappas, ed., Plenum Press (New York 1992), the disclosures of each of which are totally incorporated herein by reference.

Substituted poly(arylene ether alcohol)s can also be prepared by this method; for example, a haloalkylated poly(arylene ether ketone) or an acryloylated poly(arylene ether ketone) can be reacted with borane to yield the corresponding poly(arylene ether alcohol)s as follows:



The acetyl or acetoxy group can be converted to a hydroxyl group by continuing the reaction with borane at from about 70 to about 80°C., as follows:



In some instances, the desired substituents on the final polymer can be present on the ketone precursor polymer prior to reduction thereof; for example, haloalkyl groups or cyano groups can be present on the polymer during the reduction process and emerge therefrom unchanged. Other groups may react with the borane reducing agent; for example, amide groups might be reduced to amino groups, hydroxyl groups might be converted to borate esters, acid groups and ester groups might be reduced to alcohols, and the like. The poly(arylene ether alcohol) can be further reacted with diisocyanates, acryloyl halides such as acryloyl chloride, methacryloyl halides such as methacryloyl chloride, isocyanato-ethyl acrylate moieties, isocyanato-ethyl methacrylate moieties, or the like to allow thermal and/or photochemical crosslinking of the modified resins. Generally, a molar equivalent of the hydroxy-substituted polymer is combined with a molar equivalent of the reacting agent, such as an isocyanate, and the reaction is allowed to proceed in a solvent, such as tetrahydrofuran, other polar aprotic solvents, or the like, at ambient temperature (about 25°C.) for about 16 hours. For example, the reaction of a poly(arylene ether alcohol) with isocyanato-ethyl methacrylate proceeds as follows:



115

The hydroxymethyl-substituted poly(arylene ether alcohol)s, such as



5

116



with one specific example being



are like phenolic resins, which can be thermally cured without further modification, especially with acidic catalysts. In particular, light activated cationic initiators can be used in this situation.

The polymers of the present invention suitable for use as photoresists or in other applications wherein crosslinking or chain extension of the polymer can occur via exposure to actinic radiation, heat, crosslinking agents, or combinations thereof, contain in at least some of the monomer repeat units thereof crosslinking substituents which enable crosslinking or chain extension of the polymer upon exposure to actinic radiation. Crosslinking substituents include photosensitivity-imparting substituents, which enable crosslinking or chain extension of the polymer upon exposure to actinic radiation, thermal sensitivity-imparting substituents, which enable crosslinking or chain extension of the polymer upon exposure to heat, chemical crosslinking substituents, which enable crosslinking or chain extension of the polymer upon reaction with a crosslinking agent, substituents which require two or more of actinic radiation, heat, and/or contact with a crosslinking agent to cause crosslinking or chain extension of the polymer, and the like. These polymers, while being encompassed by the more general formula



45

are more specifically represented by the formula



50

55

60

or a mixture of



30

35

40

wherein R is a (a) hydrogen atom, (b) an alkyl group, including unsubstituted alkyl groups and substituted alkyl groups, such as hydroxyalkyl groups, preferably with from 1 to about 20 carbon atoms, more preferably with from 1 to about 10 carbon atoms, and even more preferably with from 1 to about 5 carbon atoms, (c) an aryl group, including unsubstituted aryl groups and substituted aryl groups, such as hydroxyaryl groups, preferably with from 6 to about 18 carbon atoms, more preferably with from 6 to about 12 carbon atoms, and even more preferably with 6 carbon atoms, or (d) mixtures thereof, B is



wherein P is a substituent which enables crosslinking of the polymer, a, b, c, and d are each integers of 0, 1, 2, 3, or 4, provided that at least one of a, b, c, and d is equal to or greater than 1 in at least some of the monomer repeat units of the polymer, A is

-continued



wherein v preferably is an integer of from 1 to about 20, and 45 more preferably from 1 to about 10,



wherein z preferably is an integer of from 2 to about 20, and 55 more preferably from 2 to about 10,



wherein u preferably is an integer of from 1 to about 20, and 55 more preferably from 1 to about 10,

5



10



15



20



25

30



35



40



45



50



55

60 wherein R<sub>1</sub> and R<sub>2</sub> each, independently of the other, are (a) hydrogen atoms, (b) alkyl groups, including unsubstituted alkyl groups and substituted alkyl groups, such as hydroxy-alkyl groups, preferably with from 1 to about 20 carbon atoms, more preferably with from 1 to about 10 carbon atoms, and even more preferably with from 1 to about 5 carbon atoms, although the number of carbon atoms can be outside of this range, (c) aryl groups, including unsubstituted 65 aryl groups, and (d) groups of the formula  $\text{R}_1[\text{C}(\text{OH})_2\text{R}_2]_p$ , wherein R<sub>1</sub> and R<sub>2</sub> are as defined above, and p is an integer of from 1 to about 5.

119

aryl groups and substituted aryl groups, such as hydroxyaryl groups, preferably with from 6 to about 18 carbon atoms, more preferably with from 6 to about 12 carbon atoms, and even more preferably with 6 carbon atoms, although the number of carbon atoms can be outside of this range, or (d) mixtures thereof, and p is an integer of 0 or 1,



wherein  $p$  is an integer of 0 or 1,

$$-(\text{CH}_2\text{O})_i-$$

wherein  $t$  is an integer of from 1 to about 20,



wherein (1) Z is



120

-continued

wherein p is 0 or 1; (2) Ar is



or



25 (3) G is an alkyl group selected from alkyl or isoalkyl groups containing from about 2 to about 10 carbon atoms; (4) Ar' is



(5) X is



$$\begin{array}{c} \text{H} \\ | \\ \text{CH}_3 \end{array}$$

$$\begin{array}{c} | \\ \text{CH}_3 \\ \hline \text{---O---} \end{array}$$

The diagram shows a cyclohexane ring with a methyl group (a single line) attached to each of the two top carbons of the ring.

-continued



wherein s is 0, 1, or 2,



and (6) q is 0 or 1; or mixtures thereof, hydroxy-substituted derivatives thereof, hydroxyalkyl-substituted derivatives thereof, with the hydroxyalkyl substituents preferably having from 1 to about 20 carbon atoms, more preferably from 1 to about 10 carbon atoms, and even more preferably from 1 to about 5 carbon atoms, although the number of carbon atoms can be outside of this range, hydroxyaryl-substituted derivatives thereof, with the hydroxyaryl substituents preferably having from 6 to about 18 carbon atoms, more preferably from 6 to about 12 carbon atoms, and even more preferably about 6 carbon atoms, although the number of carbon atoms can be outside of this range, or mixtures thereof, and n is an integer representing the number of repeating monomer units.

Actinic radiation which activates crosslinking or chain extension of photosensitivity imparting crosslinking groups can be of any desired source and any desired wavelength, including (but not limited to) visible light, infrared light, ultraviolet light, electron beam radiation, x-ray radiation, or the like. Examples of suitable photosensitivity imparting groups include unsaturated ester groups, such as acryloyl groups, methacryloyl groups, cinnamoyl groups, crotonoyl groups, ethacryloyl groups, oleoyl groups, linoleoyl groups, maleoyl groups, fumaroyl groups, itaconoyl groups, citraconoyl groups, phenyfmaleoyl groups, esters of 3-hexene-1,6-dicarboxylic acid, and the like. Also suitable are alkylcarboxymethylene and ether groups. Under certain conditions, such as imaging with electron beam, deep ultraviolet, or x-ray radiation, halomethyl groups are also photoactive. Epoxy groups, allyl ether groups, hydroxyalkyl groups, and unsaturated ammonium, phosphonium, and ether groups are also suitable photoactive groups.

The photopatternable polymers containing these groups can be prepared by any suitable or desired process. For example, unsaturated ester groups can be placed directly on the polymer having no photosensitive groups by a process which comprises reacting the polymer with (i) a formaldehyde source, and (ii) an unsaturated acid in the presence of an acid catalyst, thereby forming a curable polymer with unsaturated ester groups, as disclosed in, for example, Copending U.S. application Ser. No. 08/697,761, filed Aug. 29, 1996, and Copending U.S. application Ser. No. 09/221, 278, filed Dec. 23, 1998, entitled "Process for Direct Substitution of High Performance Polymers with Unsaturated Ester Groups," with the named inventors Timothy J. Fuller, Ram S. Narang, Thomas W. Smith, David J. Luca, and Raymond K. Crandall, the disclosures of each of which are totally incorporated herein by reference.

Alternatively, one or more intermediate materials can be prepared. For example, the polymer backbone can be functionalized with a substituent which allows for the facile derivatization of the polymer backbone, such as hydroxyl groups, carboxyl groups, haloalkyl groups such as chloromethyl groups, hydroxyalkyl groups such as hydroxy methyl

groups, methoxy methyl groups, alkylcarboxymethylene groups, and the like. For example, the polymer can be substituted with photosensitivity-imparting groups such as unsaturated ester groups or the like by first preparing the 5 haloalkylated derivative and then replacing at least some of the haloalkyl groups with unsaturated ester groups, as disclosed in U.S. Pat. No. 5,739,254, filed Aug. 29, 1996, and U.S. Pat. No. 5,753,783, filed Aug. 28, 1997, entitled "Process for Haloalkylation of High Performance 10 Polymers," with the named inventors Timothy J. Fuller, Ram S. Narang, Thomas W. Smith, David J. Luca, and Raymond K. Crandall, and in U.S. Pat. No. 5,761,809, filed Aug. 29, 1996, entitled "Processes for Substituting Haloalkylated 15 Polymers With Unsaturated Ester, Ether, and Alkylcarboxymethylene Groups," with the named inventors Timothy J. Fuller, Ram S. Narang, Thomas W. Smith, David J. Luca, and Raymond K. Crandall, the disclosures of each of which are totally incorporated herein by reference. For example, the haloalkylated polymer can be substituted with unsaturated 20 ester groups by reacting the haloalkylated polymer with an unsaturated ester salt in solution. Ether groups and alkylcarboxymethylene groups can also be placed on the haloalkylated polymer by a process analogous to that employed to place unsaturated ester groups on the haloalkylated polymer, except that the corresponding alkylcarboxylate or alkoxide salt is employed as a reactant. Some or all of the haloalkyl groups can be replaced with unsaturated 25 ester, ether, or alkylcarboxymethylene substituents. Longer reaction times generally lead to greater degrees of substitution of haloalkyl groups with unsaturated ester, ether, or alkylcarboxymethylene substituents.

The haloalkylated polymer can be allyl ether substituted or epoxidized by first reacting the haloalkylated polymer with an unsaturated alcohol salt, such as an allyl alcohol salt, 30 in solution, to generate the allyl-substituted polymer; if desired, the allyl-substituted polymer can be converted to an epoxy-substituted polymer by reacting it with a peroxide, such as hydrogen peroxide, m-chloroperoxybenzoic acid, acetyl peroxide, and the like, as well as mixtures thereof, to 35 yield the epoxidized polyarylene ether, as disclosed in Copending U.S. application Ser. No. 08/705,372, filed Aug. 29, 1996, and Copending U.S. application Ser. No. 09/246, 167, filed Feb. 8, 1999, entitled "High Performance Curable 40 Polymers and Processes for the Preparation Thereof," with the named inventors Ram S. Narang and Timothy J. Fuller, 45 the disclosures of each of which are totally incorporated herein by reference. Some or all of the haloalkyl groups can be replaced with allyl ether or epoxy substituents. Longer reaction times generally lead to greater degrees of substitution 50 of haloalkyl groups with allyl ether or epoxy substituents. As also disclosed in the aforementioned references, the epoxidized polymer can also be prepared by reaction of the haloalkylated polymer with an epoxy-group-containing alcohol salt, such as a glycidolate salt, or an unsaturated 55 alcohol salt, such as those set forth hereinabove, in the presence of a molar excess of base (with respect to the unsaturated alcohol salt or epoxy-group-containing alcohol salt), such as sodium hydride, sodium hydroxide, potassium carbonate, quaternary alkyl ammonium salts, or the like, 60 under phase transfer conditions. Unsaturated or allyl ether groups can also be placed on the haloalkylated polymer by other methods, such as by a Grignard reaction, a Wittig reaction, or the like.

The haloalkylated polymer can be substituted with a 65 photosensitivity-imparting, water-solubility-enhancing (or water-dispersability-enhancing) group by reacting the haloalkylated polymer with an unsaturated amine,

phosphine, or alcohol, as disclosed in Copending U.S. application Ser. No. 08/697,760, filed Aug. 29, 1996, entitled "Aqueous Developable High Performance Curable Aromatic Ether Polymers," and Copending U.S. application Ser. No. 09/247,104, filed Feb. 9, 1999, entitled "Aqueous Developable High Performance Curable Polymers," with the named inventors Ram S.

Narang and Timothy J. Fuller, the disclosures of each of which are totally incorporated herein by reference. Some or all of the haloalkyl groups can be replaced with photosensitivity-imparting, water-solubility-enhancing or water-dispersability-enhancing) substituents. Longer reaction times generally lead to greater degrees of substitution of haloalkyl groups with photosensitivity-imparting, water-solubility-enhancing (or water-dispersability-enhancing) substituents. As also disclosed in the aforementioned references, the unsubstituted polymer can be substituted with two different functional groups, one of which imparts photosensitivity to the polymer and one of which imparts water solubility or water dispersability to the polymer. Examples of reactants which can be reacted with the polymer to substitute the polymer with suitable water solubility enhancing groups or water dispersability enhancing groups include tertiary amines, tertiary phosphines, alkyl thio ethers, and the like. These water solubility imparting substituents or water dispersability imparting substituents can be placed on the polymer by any suitable or desired process. For example, two equivalents of the nucleophilic reagent (amine, phosphine, or thio ether) can be allowed to react with one equivalent of the haloalkylated polymer at 25° C. in a polar aprotic solvent such as dimethylacetamide, dimethyl sulfoxide, N-methyl pyrrolidinone, dimethyl formamide, or the like, with the reactants present in the solvent in a concentration of about 30 percent by weight solids. Reaction times typically are from about 1 to about 24 hours, with 2 hours being typical. Alternatively, the water solubility imparting group or water dispersability imparting group can be nonionic. Nonionic substituents can be placed on the polymer by, for example, reacting from about 2 to about 10 milliequivalents of a salt of the nonionic group (such as an alkali metal salt or the like) with 1 equivalent of the haloalkylated polymer in a polar aprotic solvent such as tetrahydrofuran, dimethylacetamide, dimethyl sulfoxide, N-methyl pyrrolidinone, dimethyl formamide, or the like, in the presence of a base, such as at least about 2 equivalents of sodium hydroxide, at least about 1 equivalent of sodium hydride, or the like, at about 80° C. for about 16 hours. The substitution of poly(vinyl benzyl chloride) polymers with polyether chains is disclosed in further detail in, for example, Japanese Patent Kokai 78-79,833 (1978) and in Chem. Abstr., 89, 180603 (1978), the disclosures of each of which are totally incorporated herein by reference. Higher degrees of haloalkylation generally enable higher degrees of substitution with water solubility imparting groups or water dispersability imparting groups.

The hydroxymethylation of a polymer of the above formula can be accomplished by reacting the polymer in solution with formaldehyde or paraformaldehyde and a base, such as sodium hydroxide, potassium hydroxide, calcium hydroxide, ammonium hydroxide, tetramethylammonium hydroxide, or the like, as disclosed in U.S. Pat. No. 5,849,809, filed Aug. 29, 1996, and Copending U.S. application Ser. No. 09/159,426, filed Sep. 23, 1998, entitled "Hydroxymethylated High Performance Curable Polymers," with the named inventors Ram S. Narang and Timothy J. Fuller, the disclosures of each of which are totally incorporated herein by reference. Longer reaction times generally result in higher degrees of hydroxymethylation.

As also disclosed in the aforementioned references, the unsubstituted polymers can also be hydroxymethylated by first preparing the haloalkylated derivative and then replacing at least some of the haloalkyl groups with hydroxymethyl groups. Higher degrees of haloalkylation generally enable higher degrees of substitution with hydroxymethyl groups, and thereby enable greater photosensitivity of the polymer. Some or all of the haloalkyl groups can be replaced with hydroxymethyl substituents. Longer reaction times generally lead to greater degrees of substitution of haloalkyl groups with hydroxymethyl substituents.

Intermediate derivatives can also be prepared by any suitable or desired process. For example, suitable processes for haloalkylating polymers include reaction of the polymers with formaldehyde and hydrochloric acid, bischloromethyl ether, chloromethyl methyl ether, octylchloromethyl ether, or the like, generally in the presence of a Lewis acid catalyst. Bromination of a methyl group on the polymer can also be accomplished with elemental bromine via a free radical process initiated by, for example, a peroxide initiator or light. Halogen atoms can be substituted for other halogens already on a halomethyl group by, for example, reaction with the appropriate hydrohalic acid or halide salt. Methods for the haloalkylation of polymers are also disclosed in, for example, "Chloromethylation of Condensation Polymers Containing an Oxy-1,4-Phenylene Backbone," W. H. Daly et al., *Polymer Preprints*, Vol. 20, No. 1, 835 (1979), the disclosure of which is totally incorporated herein by reference. One specific process suitable for haloalkylating the polymer entails reacting the polymer with an acetyl halide, such as acetyl chloride, and dimethoxymethane in the presence of a halogen-containing Lewis acid catalyst, as disclosed in U.S. Pat. No. 5,739,254, filed Aug. 29, 1996, and U.S. Pat. No. 5,753,783, filed Aug. 28, 1997, entitled "Process for Haloalkylation of High Performance Polymers," with the named inventors Timothy J. Fuller, Ram S. Narang, Thomas W. Smith, David J. Luca, and Raymond K. Crandall, the disclosures of each of which are totally incorporated herein by reference.

Other procedures for placing functional groups on aromatic polymers are disclosed in, for example, W. H. Daly, S. Chotiwana, and R. Nielsen, *Polymer Preprints*, 20(1), 835 (1979); "Functional Polymers and Sequential Copolymers by Phase Transfer Catalysis, 3. Synthesis And Characterization of Aromatic Poly(ether sulfone)s and Poly(oxy-2,6-dimethyl-1,4-phenylene) Containing Pendant Vinyl Groups," V. Percec and B. C. Auman, *Makromol. Chem.*, 185, 2319 (1984); F. Wang and J. Roovers, *Journal of Polymer Science: Part A: Polymer Chemistry*, 32, 2413 (1994); "Details Concerning the Chloromethylation of Soluble High Molecular Weight Polystyrene Using Dimethoxymethane, Thionyl Chloride, And a Lewis Acid: A Full Analysis," M. E. Wright, E. G. Toplikar, and S. A. Svejda, *Macromolecules*, 24, 5879 (1991); "Functional Polymers and Sequential Copolymers by Phase Transfer Catalysts," V. Percec and P. L. Rinaldi, *Polymer Bulletin*, 10, 223 (1983); "Preparation of Polymer Resin and Inorganic Oxide Supported Peroxy-Acids and Their Use in the Oxidation of Tetrahydrothiophene," J.

A. Greig, R. D. Hancock, and D. C. Sherrington, *European Polymer J.*, 16, 293 (1980); "Preparation of Poly(vinylbenzyltriphenylphosphonium Perbromide) and Its Application in the Bromination of Organic Compounds," A. Akelah, M. Hassanein, and F. Abdel-Galil, *European Polymer J.*, 20 (3) 221 (1984); J. M. J. Frechet and K. K. Haque, *Macromolecules*, 8, 130 (1975); U.S. Pat. No. 3,914,194; U.S. Pat. No. 4,110,279; U.S. Pat. No. 3,367,914; "Synthesis of

125

Intermediates for Production of Heat Resistant Polymers (Chloromethylation of Diphenyl oxide)," E. P. Tepenitsyna, M. I. Farberov, and A. P. Ivanovski, *Zhumal Prikladnoi Khimii*, Vol. 40, No. 11, 2540 (1967); U.S. Pat. No. 3,000,839; Chem Abst. 56, 590f (1962); U.S. Pat. No. 3,128,258; Chem Abstr. 61, 4560a (1964); J. D. Doedens and H. P. Cordts, *Ind. Eng. Ch.*, 83, 59 (1961); British Patent 863,702; and Chem Abstr 55, 18667b (1961); the disclosures of each of which are totally incorporated herein by reference.

Thermal sensitivity-imparting groups are also suitable crosslinking groups for the polymers of the present invention. Examples of thermal sensitivity-imparting crosslinking groups include those disclosed in Copending U.S. application Ser. No. 08/705,488, filed Aug. 29, 1996, entitled "High Performance Polymer Compositions Having Photosensitivity-Imparting Substituents and Thermal Sensitivity-Imparting Substituents," and Copending U.S. application Ser. No. 09/221,690, filed Dec. 23, 1998, entitled "High Performance Polymer Compositions," with the named inventors Thomas W. Smith, Timothy J. Fuller, Ram S. Narang, and David J. Luca, the disclosures of each of which are totally incorporated herein by reference. The thermal sensitivity imparting groups can be placed on the polymer by any suitable or desired synthetic method. Processes for putting the above mentioned thermal sensitivity imparting groups on polymers are disclosed in, for example, "Polyimides," C. E. Sroog, *Prog. Polym. Sci.*, Vol. 16, 561-694 (1991); F. E. Arnold and L. S. Tan, *Symposium on Recent Advances in Polyimides and Other High Performance Polymers*, Reno, NEV. (July 1987); L. S. Tan and F. E. Arnold, *J. Polym. Sci. Part A*, 26, 1819 (1988); U.S. Pat. No. 4,973,636; and U.S. Pat. No. 4,927,907; the disclosures of each of which are totally incorporated herein by reference. Other procedures for placing thermally curable end groups on aromatic polymers are disclosed in, for example, P. M. Hergenrother, *J. Macromol. Sci. Rev. Macromol. Chem.*, C19 (1), 1-34 (1980); V. Percec and B. C. Auman, *Makromol. Chem.*, 185, 2319 (1984); S. J. Havens, and P. M. Hergenrother, *J. of Polymer Science: Polymer Chemistry Edition*, 22, 3011 (1984); P. M. Hergenrother, *J. of Polymer Science: Polymer Chemistry Edition*, 20, 3131 (1982); V. Percec, P. L. Rinaldi, and B. C. Auman, *Polymer Bulletin*, 10, 215 (1983); "Functional Polymers and Sequential Copolymers by Phase Transfer Catalysis, 2. Synthesis and Characterization of Aromatic Poly(ether sulfones Containing Vinylbenzyl and Ethynylbenzyl Chain Ends," V. Percec and B. C. Auman, *Makromol. Chem.* 185, 1867 (1984); "Functional Polymers and Sequential Copolymers by Phase Transfer Catalysis, 6. On the Phase Transfer Catalyzed Williamson Polyetherification as a New Method for the Preparation of Alternating Block copolymers," V. Percec, B. Auman, and P. L. Rinaldi, *Polymer Bulletin*, 10, 391 (1983); "Functional Polymers and Sequential Copolymers by Phase Transfer Catalysis, 3 Synthesis and Characterization of Aromatic Poly(ether sulfone)s and Poly(oxy-2,6-dimethyl-1,4-phenylene) Containing Pendant Vinyl Groups," V. Percec and B. C. Auman, *Makromol. Chem.*, 185, 2319 (1984); and "Phase Transfer Catalysis, Functional Polymers and Sequential Copolymers by PTC,5. Synthesis and Characterization of Polyformals of Polyether Sulfones," *Polymer Bulletin*, 70, 385 (1983); the disclosures of each of which are totally incorporated herein by reference. When both photosensitivity-imparting crosslinking groups and thermal sensitivity-imparting crosslinking groups are present on the polymers of the present invention, as disclosed in Copending U.S. application Ser. No. 08/705,488 and Copending U.S. application Ser. No. 09/221,690, the polymers can also

126

be cured in a two-stage process which entails (a) exposing the polymer to actinic radiation, thereby causing the polymer to become crosslinked or chain extended through the photosensitivity-imparting groups; and (b) subsequent to step (a), heating the polymer to a temperature sufficient to cause the thermal sensitivity-imparting groups to react, thereby causing further crosslinking or chain extension of the polymer through the thermal sensitivity imparting groups.

Examples of suitable thermal sensitivity imparting groups include ethynyl groups, such as those of the formula



wherein R is



a is an integer of 0 or 1, and R' is a hydrogen atom or a phenyl group, ethylenic linkage-containing groups, such as allyl groups, including those of the formula



wherein X and Y each, independently of the other, are hydrogen atoms or halogen atoms, such as fluorine, chlorine, bromine, or iodine, vinyl groups, including those of the formula



wherein R is an alkyl group, including both saturated, unsaturated, linear, branched, and cyclic alkyl groups, preferably with from 1 to about 30 carbon atoms, more preferably with from 1 to about 11 carbon atoms, even more preferably with from 1 to about 5 carbon atoms, a substituted alkyl group, an aryl group, preferably with from 6 to about 24 carbon atoms, more preferably with from 6 to about 18 carbon atoms, a substituted aryl group, an arylalkyl group, preferably with from 7 to about 30 carbon atoms, more preferably with from 7 to about 19 carbon atoms, or a substituted arylalkyl group, wherein the substituents on the substituted alkyl groups, substituted aryl groups, substituted arylalkyl groups, substituted alkoxy groups, substituted aryloxy groups, and substituted arylalkyloxy groups can be (but are not limited to) hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, mixtures thereof, and the like, wherein any two or more substituents can be joined together to form a ring, vinyl ether groups, such as those of the formula



epoxy groups, including those of the formula



R is an alkyl group, including both saturated, unsaturated, linear, branched, and cyclic alkyl groups, preferably with from 1 to about 30 carbon atoms, more preferably with from 1 to about 11 carbon atoms, even more preferably with from 1 to about 5 carbon atoms, a substituted alkyl group, an aryl group, preferably with from 6 to about 24 carbon atoms, more preferably with from 6 to about 18 carbon atoms, a substituted aryl group, an arylalkyl group, preferably with from 7 to about 30 carbon atoms, more preferably with from 7 to about 19 carbon atoms, or a substituted arylalkyl group, wherein the substituents on the substituted alkyl groups, substituted aryl groups, substituted arylalkyl groups, substituted alkoxy groups, substituted aryloxy groups, and substituted arylalkyloxy groups can be (but are not limited to) hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, mixtures thereof, and the like, wherein any two or more substituents can be joined together to form a ring, vinyl ether groups, such as those of the formula

mixtures thereof, and the like, wherein any two or more substituents can be joined together to form a ring, halomethyl groups, such as fluoromethyl groups, chloromethyl groups, bromomethyl groups, and iodomethyl groups, hydroxymethyl groups, benzocyclobutene groups, including those of the formula



phenolic groups ( $-\phi-OH$ ), provided that the phenolic groups are present in combination with either halomethyl groups or hydroxymethyl groups; the halomethyl groups or hydroxymethyl groups can be present on the same polymer bearing the phenolic groups or on a different polymer, or on a monomeric species present with the phenolic group substituted polymer; maleimide groups, such as those of the formula



biphenylene groups, such as those of the formula



5-norbornene-2,3-dicarboximido (nadimido) groups, such as those of the formula



alkylcarboxylate groups, such as those of the formula



wherein R is an alkyl group (including saturated, unsaturated, and cyclic alkyl groups), preferably with from 1 to about 30 carbon atoms, more preferably with from 6 to about 6 carbon atoms, a substituted alkyl group, an aryl group, preferably with from 6 to about 30 carbon atoms, more preferably with from 1 to about 2 carbon atoms, a substituted aryl group, an arylalkyl group, preferably with from 7 to about 35 carbon atoms, more preferably with from 7 to about 15 carbon atoms, or a substituted arylalkyl group, wherein the substituents on the substituted alkyl, aryl, and arylalkyl groups can be (but are not limited to) alkoxy

groups, preferably with from 1 to about 6 carbon atoms, aryloxy groups, preferably with from 6 to about 24 carbon atoms, arylalkyloxy groups, preferably with from 7 to about 30 carbon atoms, hydroxy groups, amine groups, imine groups, ammonium groups, pyridine groups, pyridinium groups, ether groups, ester groups, amide groups, carbonyl groups, thiocarbonyl groups, sulfate groups, sultonate groups, sulfide groups, sulfoxide groups, phosphine groups, phosphonium groups, phosphate groups, mercapto groups, nitroso groups, sulfone groups, acyl groups, acid anhydride groups, azide groups, and the like, wherein two or more substituents can be joined together to form a ring, and the like. Any desired or suitable degree of substitution can be employed. Preferably, the degree of substitution is from about 1 to about 4 thermal sensitivity imparting groups per repeat monomer unit, although the degree of substitution can be outside this range. Preferably, the degree of substitution is from about 0.5 to about 5 milliequivalents of thermal sensitivity imparting group per gram of polymer, and more preferably from about 0.75 to about 1.5 milliequivalents per gram, although the degree of substitution can be outside this range.

The temperature selected for the thermal crosslinking generally depends on the thermal sensitivity imparting group which is present on the polymer. For example, ethynyl groups preferably are cured at temperatures of from about 150 to about 300° C. Halomethyl groups preferably are cured at temperatures of from about 150 to about 260° C. Hydroxymethyl groups preferably are cured at temperatures of from about 150 to about 250° C. Phenylethynyl phenyl groups preferably are cured at temperatures of greater than about 250° C. Vinyl groups preferably are cured at temperatures of from about 80 to about 250° C. Allyl groups preferably are cured at temperatures of over about 200° C. Epoxy groups preferably are cured at temperatures of about 150° C. Maleimide groups preferably are cured at temperatures of from about 200 to about 300° C. Benzocyclobutene groups preferably are cured at temperatures of over about 200° C. 5-Norbornene-2,3-dicarboximidogroups preferably are cured at temperatures of from about 200 to about 300° C. Vinyl ether groups preferably are cured at temperatures of about 150° C. Phenolic groups in the presence of hydroxymethyl or halomethyl groups preferably are cured at temperatures of from about 150 to about 210° C. Alkylcarboxylate groups preferably are cured at temperatures of from about 150 to about 250° C. Curing temperatures usually do not exceed about 400° C., although higher temperatures can be employed provided that decomposition of the polymer does not occur. Higher temperature cures preferably take place in an oxygen-excluded environment.

Further examples of suitable crosslinking groups include isocyanate groups, acryloyl halide groups such as acryloyl chloride groups, vinyl benzyl halide groups such as vinyl benzyl chloride groups, ethynyl benzyl halide groups such as ethynyl benzyl chloride groups, methacryloyl halide groups such as methacryloyl chloride groups, 2-isocyanatoethyl methacrylate groups, diisocyanate groups, including toluene diisocyanate, hexane diisocyanate, and the like, and any other suitable functional group which enables crosslinking or chain extension of the polymer upon exposure to actinic radiation, heat, crosslinking agents, mixtures thereof, or the like.

Further information regarding photoresist compositions is disclosed in, for example, J. J. Zupancic, D. C. Blazej, T. C. Baker, and E. A. Dinkel, *Polymer Preprints*, 32, (2), 178 (1991); "High Performance Electron Negative Resist, Chloromethylated Polystyrene. A Study on Molecular

Parameters," S. Imamura, T. Tamamura, and K. Harada, *J. of Applied Polymer Science*, 27, 937 (1982); "Chloromethylated Polystyrene as a Dry Etching-Resistant Negative Resist for Submicron Technology", S. Imamura, *J. Electrochem. Soc.: Solid-state Science and Technology*, 126(9), 1628 (1979); "UV curing of composites based on modified unsaturated polyesters," W. Shi and B. Ranby, *J. of Applied Polymer Science*, Vol. 51, 1129 (1994); "Cinnamates VI. Light-Sensitive Polymers with Pendant o-, m- and p-hydroxycinnamate Moieties," F. Scigalski, M. Toczek, and J. Paczkowski, *Polymer*, 35, 692 (1994); and "Radiation-cured Polyurethane Methacrylate Pressure-sensitive Adhesives," G. Ansell and C. Butler, *Polymer*, 35 (9), 2001 (1994), the disclosures of each of which are totally incorporated herein by reference.

When the crosslinking groups are photosensitivity imparting groups, the photopatternable polymer can be cured by uniform exposure to actinic radiation at wavelengths and/or energy levels capable of causing crosslinking or chain extension of the polymer through the photosensitivity-imparting groups. Alternatively, the photopatternable polymer is developed by imagewise exposure of the material to radiation at a wavelength and/or at an energy level to which the photosensitivity-imparting groups are sensitive. Typically, a photoresist composition will contain the photopatternable polymer, an optional solvent for the photopatternable polymer, an optional sensitizer, and an optional photoinitiator. Solvents may be particularly desirable when the uncrosslinked photopatternable polymer has a high  $T_g$ . The solvent and photopatternable polymer typically are present in relative amounts of from 0 to about 99 percent by weight solvent and from about 1 to 100 percent polymer, preferably are present in relative amounts of from about 20 to about 60 percent by weight solvent and from about 40 to about 80 percent by weight polymer, and more preferably are present in relative amounts of from about 30 to about 60 percent by weight solvent and from about 40 to about 70 percent by weight polymer, although the relative amounts can be outside these ranges.

While not being limited to any particular theory, it is believed that exposure to, for example, ultraviolet radiation generally leads to crosslinking or chain extension at the "long" bond sites as shown below for the unsaturated ester-substituted polymer having, for example, acryloyl functional groups, wherein the ethylenic linkage in the acryloyl group is opened to form the link:



Similarly, it is believed that exposure to, for example, ultraviolet radiation generally leads to crosslinking or chain extension at the "long" bond sites as shown below for the

131

acrylate-isocyanate modified polymer, wherein the ethylenic linkage in the functional group is opened to form the link:



An analogous opening of the ethylenic linkage occurs for other unsaturated groups. The alkylcarboxymethylene and ether substituted polymers are curable by exposure to ultraviolet light, preferably in the presence of heat and one or more cationic initiators, such as triarylsulfonium salts, diaryliodonium salts, and other initiators as disclosed in, for example, Ober et al., *J.M.S.—Pure Appl. Chem.*, A30 (12), 877-897 (1993); G. E. Green, B. P. Stark, and S. A. Zahir, "Photocrosslinkable Resin Systems," *J. Macro. Sci.—Revs. Macro. Chem.*, C21(2), 187 (1981); H. F. Gruber, "Photoinitiators for Free Radical Polymerization," *Prog. Polym. Sci.*, Vol. 17, 953 (1992); Johann G. Kloosterboer, "Network Formation by Chain Crosslinking Photopolymerization and Its Applications in Electronics," *Advances in Polymer Science*, 89, Springer-Verlag Berlin Heidelberg (1988); and "Diaryliodonium Salts as Thermal Initiators of Cationic Polymerization," J. V. Crivello, T.P. Lockhart, and J. L. Lee, *J. of Polymer Science: Polymer Chemistry Edition*, 21, 97 (1983), the disclosures of each of which are totally incorporated herein by reference. While not being limited to any particular theory, it is believed that the cationic mechanism is as shown below for the methylcarboxymethylene polymer, wherein acetic acid is liberated and the "long" bond indicates the crosslinking or chain extension site:



132

-continued



The reaction is similar for the ether-substituted polymer, except that the corresponding alkanol is liberated.

15 The allyl ether substituted polymer is developed by imagewise exposure of the material to radiation at a wavelength to which it is sensitive. While not being limited to any particular theory, it is believed that exposure to, for example, ultraviolet radiation generally opens the ethylenic linkage in the allyl ether groups and leads to crosslinking or chain extension at the "long" bond sites as shown below:



For the epoxy-substituted polymer, while not being limited to any particular theory, it is believed that exposure to, for example, ultraviolet radiation generally causes generation of acidic species by the initiator, followed by reaction of the acidic species with the epoxy groups to cause ring opening and crosslinking or chain extension at the "long" bond sites as shown below:



133

-continued



5

10

15

Amine curing of the epoxidized polymer is also possible, with curing occurring upon the application of heat. While not being limited to any particular theory, it is believed that the curing scheme in one example is as follows:



20

25

30

35

40

45

55

For the halomethylated polymer, while not being limited to any particular theory, it is believed that exposure to, for example, e-beam, deep ultraviolet, or x-ray radiation generally results in free radical cleavage of the halogen atom from the methyl group to form a benzyl radical. Crosslinking or chain extension then occurs at the "long" bond sites as illustrated below:



134

-continued



5

10

15

20

25

30

35

40

45

55

60

For the hydroxyalkylated, haloalkylated, and allyl-substituted polymers of the present invention, one specific example of a class of suitable sensitizers or initiators is that of bis(azides), of the general formula

For the unsaturated ammonium or unsaturated phosphonium substituted polymers of the present invention, while not being limited to any particular theory, it is believed that exposure to, for example, ultraviolet radiation generally opens the ethylenic linkage in the photosensitivity-imparting groups and leads to crosslinking or chain extension at the "long" bond sites as shown below:



hv sensitizer

135



wherein R is



or



wherein R<sub>1</sub>, R<sub>2</sub>, R<sub>3</sub>, and R<sub>4</sub> each, independently of the others, is a hydrogen atom, an alkyl group, including saturated, unsaturated, and cyclic alkyl groups, preferably with from 1 to about 30 carbon atoms, and more preferably with from 1 to about 6 carbon atoms, a substituted alkyl group, an aryl group, preferably with from 6 to about 18 carbon atoms, and more preferably with about 6 carbon atoms, a substituted aryl group, an arylalkyl group, preferably with from 7 to about 48 carbon atoms, and more preferably with from about 7 to about 8 carbon atoms, or a substituted arylalkyl group, and x is 0 or 1, wherein the substituents on the substituted alkyl, aryl, and aryl groups can be (but are not limited to) alkyl groups, including saturated, unsaturated, linear, branched, and cyclic alkyl groups, preferably with from 1 to about 6 carbon atoms, substituted alkyl groups, preferably with from 1 to about 6 carbon atoms, aryl groups, preferably with from 6 to about 24 carbon atoms, substituted aryl groups, preferably with from 6 to about 24 carbon atoms, arylalkyl groups, preferably with from 7 to about 30 carbon atoms, substituted arylalkyl groups, preferably with from 7 to about 30 carbon atoms, alkoxy groups, preferably with from 6 to about 6 carbon atoms, substituted alkoxy groups, preferably with from 1 to about 6 carbon atoms, aryloxy groups, preferably with from 6 to about 24 carbon atoms, substituted aryloxy groups, preferably with from 6 to about 24 carbon atoms, arylalkyloxy groups, preferably with from 7 to about 30 carbon atoms, substituted arylalkyloxy groups, preferably with from 7 to about 30 carbon atoms, amine groups, imine groups, ammonium groups, pyridine groups, pyridinium groups, ether groups, ester groups, amide groups, carbonyl groups, thiocarbonyl groups, sulfate groups, sulfonate groups, sulfide groups, sulfoxide groups, phosphine groups, phosphonium groups, phosphate groups, mercapto groups, nitroso groups, sulfone groups, acyl groups, acid anhydride groups, azide groups, and the like, wherein the substituents on the substituted alkyl groups, substituted aryl groups, substituted arylalkyl groups, substituted alkoxy groups, substituted aryloxy groups, and substituted arylalkyloxy groups can be (but are not limited to) hydroxy groups, amine groups, imine groups, ammonium groups, pyridine groups,

136

pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, mixtures thereof, and the like, wherein any two or more substituents can be joined together to form a ring. Examples of suitable bis(azides) include 4,4'-diazidostilbene, of the formula



4,4'-diazidostilbene, of the formula



25 2,6-di(4'-azidobenzyl)-4-methylcyclohexanone, of the formula



4,4'-diazidobenzalacetone, of the formula



45 and the like. While not being limited to any particular theory, it is believed that exposure to, for example, ultraviolet radiation enables curing, as illustrated below for the hydroxymethylated polymer:



137



138



Alternatively, a hydroxyalkylated polymer can be further reacted to render it more photosensitive. For example, a hydroxymethylated polymer of the formula



can react with isocyanato-ethyl methacrylate, of the formula



(available from Polysciences, Warrington, Pa.) to form a photoactive polymer of the formula



wherein X and X' each, independently of the other, is —H or —OH (or —H or a halogen atom in the case of the haloalkylated polymer). Similarly, for the allyl-substituted polymer, it is believed that the curing reaction scheme is as follows:



This reaction can be carried out in tetrahydrofuran at 25° C. with 1 part by weight polymer, 1 part by weight isocyanato-ethyl methacrylate, and 50 parts by weight methylene chloride. Typical reaction temperatures are from about 0 to about 60 50° C., with 10 to 25° C. preferred. Typical reaction times are between about 1 and about 24 hours, with about 16 hours preferred. During exposure to, for example, ultraviolet radiation, the ethylenic bond opens and crosslinking or chain extension occurs at that site.

While not being limited to any particular theory, it is believed that thermal cure can also lead to extraction of the hydroxy group and to crosslinking or chain extension at the

139

"long" bond sites as shown below:



If desired, the hydroxyalkylated polymer can be further reacted with an unsaturated acid chloride to substitute some or all of the hydroxyalkyl groups with photosensitive groups such as acryloyl or methacryloyl groups or other unsaturated ester groups, as disclosed in U.S. Pat. No. 5,849,809 and Copending U.S. application Ser. No. 09/159,426. Some or all of the hydroxyalkyl groups can be replaced with unsaturated ester substituents. Longer reaction times generally lead to greater degrees of substitution of hydroxyalkyl groups with unsaturated ester substituents.

FIG. 1 illustrates schematically one embodiment of the imaging members of the present invention. Specifically, FIG. 1 shows a photoconductive imaging member comprising a conductive substrate 101, a photogenerating layer 103 comprising a photogenerating compound 102 dispersed in a resinous binder composition 104, and a charge transport layer 105, which comprises a charge transporting molecule 107 dispersed in a resinous binder composition 109. At least one of the resinous binder compositions 104 and 109 comprises a polymer of the specific formulae indicated herein.

FIG. 2 illustrates schematically essentially the same member as that shown in FIG. 1 with the exception that the charge transport layer is situated between the conductive substrate and the photogenerating layer. More specifically, FIG. 2 illustrates a photoconductive imaging member comprising a conductive substrate 121, a charge transport layer 123 comprising a charge transport composition 124 dispersed in a resinous binder composition 125, and a photogenerating layer 127 comprising a photogenerating compound 128 dispersed in a resinous binder composition 129. At least one of the resinous binder compositions 125 and 129 comprises a polymer of the specific formulae indicated herein.

FIG. 3 illustrates schematically a photoconductive imaging member of the present invention comprising a conductive substrate 131, an optional charge blocking metal oxide layer 133, an optional adhesive layer 135, a photogenerating layer 137 comprising a photogenerating compound 137a dispersed in a resinous binder composition 137b, a charge transport layer 139 comprising a charge transport compound 139a dispersed in a resinous binder 139b, an optional anticurl backing layer 136, and an optional protective over-coating layer 138. At least one of the layers 135, 136, 137, 138, and 139 comprises a polymer of the specific formulae indicated herein.

FIG. 4 illustrates schematically a photoconductive imaging member of the present invention comprising a conductive substrate 141 and a photogenerating layer 143 comprising a photogenerating compound 142 dispersed in a resinous binder composition 144. Resinous binder composition 144

140

comprises a polymer of the specific formulae indicated herein. Optionally, a charge transport material 145 can also be dispersed in binder 144.

The substrate can be formulated entirely of an electrically conductive material, or it can be an insulating material having an electrically conductive surface. The substrate is of an effective thickness, generally up to about 100 mils, and preferably from about 1 to about 50 mils, although the thickness can be outside of this range. The thickness of the substrate layer depends on many factors, including economic and mechanical considerations. Thus, this layer may be of substantial thickness, for example over 100 mils, or of minimal thickness provided that there are no adverse effects on the system. Similarly, the substrate can be either rigid or flexible. In a particularly preferred embodiment, the thickness of this layer is from about 3 mils to about 10 mils. For flexible belt imaging members, preferred substrate thicknesses are from about 65 to about 150 microns, and more preferably from about 75 to about 100 microns for optimum flexibility and minimum stretch when cycled around small diameter rollers of, for example, 19 millimeter diameter.

The substrate can be opaque or substantially transparent and can comprise numerous suitable materials having the desired mechanical properties. The entire substrate can comprise the same material as that in the electrically conductive surface or the electrically conductive surface can be merely a coating on the substrate. Any suitable electrically conductive material can be employed. Typical electrically conductive materials include copper, brass, nickel, zinc, chromium, stainless steel, conductive plastics and rubbers, aluminum, semitransparent aluminum, steel, cadmium, silver, gold, zirconium, niobium, tantalum, vanadium, hafnium, titanium, nickel, chromium, tungsten, molybdenum, paper rendered conductive by the inclusion of a suitable material therein or through conditioning in a humid atmosphere to ensure the presence of sufficient water content to render the material conductive, indium, tin, metal oxides, including tin oxide and indium tin oxide, and the like. The conductive layer can vary in thickness over substantially wide ranges depending on the desired use of the electrophotoconductive member. Generally, the conductive layer ranges in thickness from about 50 Angstroms to many centimeters, although the thickness can be outside of this range. When a flexible electrophotographic imaging member is desired, the thickness of the conductive layer typically is from about 20 Angstroms to about 750 Angstroms, and preferably from about 100 to about 200 Angstroms for an optimum combination of electrical conductivity, flexibility, and light transmission. When the selected substrate comprises a nonconductive base and an electrically conductive layer coated thereon, the substrate can be of any other conventional material, including organic and inorganic materials. Typical substrate materials include insulating non-conducting materials such as various resins known for this purpose including polycarbonates, polyamides, polyurethanes, paper, glass, plastic, polyesters such as Mylar (available from Du Pont) or Melinex 447 (available from ICI Americas, Inc.), and the like. The conductive layer can be coated onto the base layer by any suitable coating technique, such as vacuum deposition or the like. If desired, the substrate can comprise a metallized plastic, such as titanized or aluminized Mylar, wherein the metallized surface is in contact with the photogenerating layer or any other layer situated between the substrate and the photogenerating layer. The coated or uncoated substrate can be flexible or rigid, and can have any number of configurations, such as a plate, a cylindrical drum, a scroll, an endless flexible belt, or the like.

141

The outer surface of the substrate may comprise a metal oxide such as aluminum oxide, nickel oxide, titanium oxide, or the like.

The photoconductive imaging member may optionally contain a charge blocking layer situated between the conductive substrate and the photogenerating layer. Generally, electron blocking layers for positively charged photoreceptors allow holes from the imaging surface of the photoreceptor to migrate toward the conductive layer, while hole blocking layers for negatively charged photoreceptors allow electrons from the imaging surface of the photoreceptor to migrate toward the conductive layer. This layer may comprise metal oxides, such as aluminum oxide and the like, or materials such as silanes and nylons, nitrogen containing siloxanes or nitrogen containing titanium compounds such as trimethoxysilyl propylene diamine, hydrolyzed trimethoxysilyl propyl ethylene diamine, N-beta-(aminoethyl) gamma-amino-propyl trimethoxy silane, isopropyl 4-aminobenzene sulfonyl, di(dodecylbenzene sulfonyl) titanate, isopropyl di(4-aminobenzoyl)isostearoyl titanate, isopropyl tri(N-ethylamino-ethylamino)titanate, isopropyl trianthranil titanate, isopropyl tri(N,N-dimethyl-ethylamino)titanate, titanium-4-amino benzene sulfonate oxyacetate, titanium 4-aminobenzoate isostearate oxyacetate,  $[H_2N(CH_2)_4]CH_3Si(OCH_3)_2$ , (gamma-aminobutyl) methyl diethoxysilane, and  $[H_2N(CH_2)_3]CH_3Si(OCH_3)_2$  (gamma-aminopropyl) methyl diethoxysilane, as disclosed in U.S. Pat. Nos. 4,291,110, 4,338,387, 4,286,033 and 4,291,110, the disclosures of each of which are totally incorporated herein by reference, or the like. Additional examples of suitable materials include gelatin (e.g. Gelatin 225, available from Knox Gelatine Inc.), and/or Carboset 515 (B.F. Goodrich Chemical Company) dissolved in water and methanol, polyvinyl alcohol, polyamides, gamma-aminopropyl triethoxysilane, polyisobutyl methacrylate, copolymers of styrene and acrylates such as styrene/n-butyl methacrylate, copolymers of styrene and vinyl toluene, polycarbonates, alkyl substituted polystyrenes, styrene-olefin copolymers, polyesters, polyurethanes, polyterpenes, silicone elastomers, mixtures or blends thereof, copolymers thereof, and the like. A preferred blocking layer comprises a reaction product between a hydrolyzed silane and the oxidized surface of a metal ground plane layer. The oxidized surface inherently forms on the outer surface of most metal ground plane layers when exposed to air after deposition. The primary purpose of this layer is to prevent charge injection from the substrate during and after charging. This layer is typically of a thickness of less than 50 Angstroms to about 10 microns, preferably being no more than about 2 microns, and more preferably being no more than about 0.2 microns, although the thickness can be outside these ranges.

The blocking layer may be applied by any suitable conventional technique such as spraying, dip coating, draw bar coating, gravure coating, silk screening, air knife coating, reverse roll coating, vacuum deposition, chemical treatment or the like. For convenience in obtaining thin layers, the blocking layers are preferably applied in the form of a dilute solution, with the solvent being removed after deposition of the coating by conventional techniques such as by vacuum, heating and the like.

In some cases, intermediate adhesive layers between the substrate and subsequently applied layers may be desirable to improve adhesion. If such adhesive layers are utilized, they preferably have a dry thickness of from about 0.1 micron to about 5 microns, although the thickness can be outside of this range. Typical adhesive layers include film-forming polymers such as polyesters, polyvinylbutyral,

142

polyvinylpyrrolidones, polycarbonates, polyurethanes, polymethylmethacrylates, duPont 49,000 (available from E.I. duPont de Nemours and Company), Vitel PE100 (available from Goodyear Tire & Rubber), and the like as well as mixtures thereof. The high performance polymers of the present invention can also be employed in the adhesive layer of the imaging member, either alone or in combination with other materials. Since the surface of the substrate can be a charge blocking layer or an adhesive layer, the expression "substrate" as employed herein is intended to include a charge blocking layer with or without an adhesive layer on a charge blocking layer. Typical adhesive layer thicknesses are from about 0.05 micron (500 angstroms) to about 0.3 micron (3,000 angstroms), although the thickness can be outside this range. Conventional techniques for applying an adhesive layer coating mixture to the substrate include spraying, dip coating, roll coating, wire wound rod coating, gravure coating, Bird bar applicator coating, slot coating, or the like. Drying of the deposited coating may be effected by any suitable conventional technique, such as oven drying, infra red radiation drying, air drying, or the like.

The photogenerating layer may comprise single or multiple layers comprising inorganic or organic compositions and the like. One example of a generator layer is described in U.S. Pat. No. 3,121,006, the disclosure of which is totally incorporated herein by reference, wherein finely divided particles of a photoconductive inorganic compound are dispersed in an electrically insulating organic resin binder. Multi-photogenerating layer compositions may be utilized where a photoconductive layer enhances or reduces the properties of the photogenerating layer. Examples of this type of configuration are described in U.S. Pat. No. 4,415,639, the disclosure of which is totally incorporated herein by reference. Further examples of photosensitive members having at least two electrically operative layers include the charge generator layer and diamine containing transport layer members disclosed in U.S. Pat. No. 4,265,990, U.S. Pat. No. 4,233,384, U.S. Pat. No. 4,306,008, and U.S. Pat. No. 4,299,897, the disclosures of each of which are totally incorporated herein by reference; dyestuff generator layer and oxadiazole, pyrazalone, imidazole, bromopyrene, nitrofluorene and nitronaphthalimide derivative containing charge transport layers members, as disclosed in U.S. Pat. No. 3,895,944, the disclosure of which is totally incorporated herein by reference; generator layer and hydrazone containing charge transport layers members, disclosed in U.S. Pat. No. 4,150,987, the disclosure of which is totally incorporated herein by reference; generator layer and a tri-aryl pyrazoline compound containing charge transport layer members, as disclosed in U.S. Pat. No. 3,837,851, the disclosure of which is totally incorporated herein by reference; and the like.

The photogenerating or photoconductive layer contains any desired or suitable photoconductive material. The photoconductive layer or layers may contain inorganic or organic photoconductive materials. Typical inorganic photoconductive materials include amorphous selenium, trigonal selenium, alloys of selenium with elements such as tellurium, arsenic, and the like, amorphous silicon, cadmium sulfoselenide, cadmium selenide, cadmium sulfide, zinc oxide, titanium dioxide and the like. Inorganic photoconductive materials can, if desired, be dispersed in a film forming polymer binder.

Typical organic photoconductors include various phthalocyanine pigments, such as the X-form of metal free phthalocyanine described in U.S. Pat. No. 3,357,989, the disclosure of which is totally incorporated herein by

reference, metal phthalocyanines such as vanadyl phthalocyanine, copper phthalocyanine, and the like, quinacridones, including those available from DuPont as Monastral Red, Monastral Violet and Monastral Red Y, substituted 2,4-diamino-triazines as disclosed in U.S. Pat. No. 3,442,781, the disclosure of which is totally incorporated herein by reference, polynuclear aromatic quinones, Indofast Violet Lake B, Indofast Brilliant Scarlet, Indofast Orange, dibromoanthranthrones such as those available from DuPont as Vat orange 1 and Vat orange 3, squarylium, pyrazolones, polyvinylcarbazole-2,4,7-trinitrofluorenone, anthracene, benzimidazole perylene, polynuclear aromatic quinones available from Allied Chemical Corporation under the tradename Indofast Double Scarlet, Indofast Violet Lake B, Indofast Brilliant Scarlet and Indofast Orange, and the like. Many organic photoconductor materials may also be used as particles dispersed in a resin binder.

Examples of suitable binders for the photoconductive materials include thermoplastic and thermosetting resins such as polycarbonates, polyesters, including polyethylene terephthalate, polyurethanes, polystyrenes, polybutadienes, polysulfones, polyarylethers, polyarylsulfones, polyethersulfones, polyethylenes, polypropylenes, polymethylpentenes, polyphenylene sulfides, polyvinyl acetates, polyvinylbutyrals, polysiloxanes, polyacrylates, polyvinyl acetals, polyamides, polyimides, amino resins, phenylene oxide resins, A terephthalic acid resins, phenoxy resins, epoxy resins, phenolic resins, polystyrene and acrylonitrile copolymers, polyvinylchlorides, polyvinyl alcohols, poly-(N-vinylpyrrolidinone)s, vinylchloride and vinyl acetate copolymers, acrylate copolymers, alkyd resins, cellulosic film formers, poly(amideimide), styrene-butadiene copolymers, vinylidenechloride-vinylchloride copolymers, vinylacetate-vinylidenechloride copolymers, styrene-alkyd resins, polyvinylcarbazoles, and the like. These polymers may be block, random or alternating copolymers. The high performance polymers of the present invention can also be employed in the photoconductive layer of the imaging member, either alone or in combination with other materials.

When the photogenerating material is present in a binder material, the photogenerating composition or pigment may be present in the film forming polymer binder compositions in any suitable or desired amounts. For example, from about 10 percent by volume to about 60 percent by volume of the photogenerating pigment may be dispersed in about 40 percent by volume to about 90 percent by volume of the film forming polymer binder composition, and preferably from about 20 percent by volume to about 30 percent by volume of the photogenerating pigment may be dispersed in about 70 percent by volume to about 80 percent by volume of the film forming polymer binder composition. Typically, the photoconductive material is present in the photogenerating layer in an amount of from about 5 to about 80 percent by weight, and preferably from about 25 to about 75 percent by weight, and the binder is present in an amount of from about 20 to about 95 percent by weight, and preferably from about 25 to about 75 percent by weight, although the relative amounts can be outside these ranges.

The particle size of the photoconductive compositions and/or pigments preferably is less than the thickness of the deposited solidified layer, and more preferably is between about 0.01 micron and about 0.5 micron to facilitate better coating uniformity.

The photogenerating layer containing photoconductive compositions and the resinous binder material generally ranges in thickness from about 0.05 micron to about 10

microns or more, preferably being from about 0.1 micron to about 5 microns, and more preferably having a thickness of from about 0.3 micron to about 3 microns, although the thickness can be outside these ranges. The photogenerating layer thickness is related to the relative amounts of photogenerating compound and binder, with the photogenerating material often being present in amounts of from about 5 to about 100 percent by weight. Higher binder content compositions generally require thicker layers for photogeneration. Generally, it is desirable to provide this layer in a thickness sufficient to absorb about 90 percent or more of the incident radiation which is directed upon it in the imagewise or printing exposure step. The maximum thickness of this layer is dependent primarily upon factors such as mechanical considerations, the specific photogenerating compound selected, the thicknesses of the other layers, and whether a flexible photoconductive imaging member is desired.

The photogenerating layer can be applied to underlying layers by any desired or suitable method. Any suitable technique may be utilized to mix and thereafter apply the photogenerating layer coating mixture. Typical application techniques include spraying, dip coating, roll coating, wire wound rod coating, and the like. Drying of the deposited coating may be effected by any suitable technique, such as oven drying, infra red radiation drying, air drying and the like.

Any other suitable multilayer photoconductors may also be employed in the imaging member of this invention. Some multilayer photoconductors comprise at least two electrically operative layers, a photogenerating or charge generating layer and a charge transport layer. The charge generating layer and charge transport layer as well as the other layers may be applied in any suitable order to produce either positive or negative charging photoreceptors. For example, the charge generating layer may be applied prior to the charge transport layer, as illustrated in U.S. Pat. No. 4,265,990, or the charge transport layer may be applied prior to the charge generating layer, as illustrated in U.S. Pat. No. 4,346,158, the entire disclosures of these patents being incorporated herein by reference.

When present, the optional charge transport layer can comprise any suitable charge transport material. The active charge transport layer may consist entirely of the desired charge transport material, or may comprise an activating compound useful as an additive dispersed in electrically inactive polymeric materials making these materials electrically active. These compounds may be added to polymeric materials which are incapable of supporting the injection of photogenerated holes from the generation material and incapable of allowing the transport of these holes therethrough, thereby converting the electrically inactive polymeric material to a material capable of supporting the injection of photogenerated holes from the generation material and capable of allowing the transport of these holes through the active layer in order to discharge the surface charge on the active layer. An especially preferred transport layer comprises from about 25 percent to about 75 percent by weight of at least one charge transporting compound, and from about 75 percent to about 25 percent by weight of a polymeric film forming resin in which the aromatic amine is soluble.

Examples of charge transport materials include pure selenium, selenium-arsenic alloys, selenium-arsenic-halogen alloys, selenium-halogen, and the like. Generally, from about 10 parts by weight per million to about 200 parts by weight per million of halogen are present in a halogen doped selenium charge transport layer, although the amount

145

can be outside of this range. If a halogen doped transport layer free of arsenic is utilized, the halogen content preferably is less than about 20 parts by weight per million. Transport layers are well known in the art. Typical transport layers are described, for example, in U.S. Pat. No. 4,609,605 and in U.S. Pat. No. 4,297,424, the disclosures of each of these patents being totally incorporated herein by reference.

Organic charge transport materials can also be employed. Typical charge transporting materials include the following:

Diamine transport molecules of the type described in U.S. Pat. No. 4,306,008, U.S. Pat. No. 4,304,829, U.S. Pat. No. 4,233,384, U.S. Pat. No. 4,115,116, U.S. Pat. No. 4,299,897, U.S. Pat. No. 4,265,990, and U.S. Pat. No. 4,081,274, the disclosures of each of which are totally incorporated herein by reference. Typical diamine transport molecules include N,N'-diphenyl-N,N'-bis(3"-methylphenyl)-(1,1'-biphenyl)-4,4'-diamine, N,N'-diphenyl-N,N'-bis(4-methylphenyl)-(1,1'-biphenyl)-4,4'-diamine, N,N'-diphenyl-N,N'-bis(2-methylphenyl)-(1,1'-biphenyl)-4,4'-diamine, N,N'-diphenyl-N,N'-bis(3-ethylphenyl)-(1,1'-biphenyl)-4,4'-diamine, N,N'-diphenyl-N,N'-bis(4-ethylphenyl)-(1,1'-biphenyl)-4,4'-diamine, N,N'-diphenyl-N,N'-bis(4-n-butylphenyl)-(1,1'-biphenyl)-4,4'-diamine, N,N'-diphenyl-N,N'-bis(3-chlorophenyl)-(1,1'-biphenyl)-4,4'-diamine, N,N'-diphenyl-N,N'-bis(4-chlorophenyl)-(1,1'-biphenyl)-4,4'-diamine, N,N'-diphenyl-N,N'-bis(phenylmethyl)-(1,1'-biphenyl)-4,4'-diamine, N,N,N',N'-tetraphenyl-[2,2'-dimethyl-1,1'-biphenyl]-4,4'-diamine, N,N,N',N'-tetraphenyl-[2,2'-dimethyl-1,1'-biphenyl]-4,4'-diamine, N,N'-diphenyl-N,N'-bis(4-methylphenyl)-[2,2'-dimethyl-1,1'-biphenyl]-4,4'-diamine, N,N'-diphenyl-N,N'-bis(2-methylphenyl)-[2,2'-dimethyl-1,1'-biphenyl]-4,4'-diamine, N,N'-diphenyl-N,N'-bis(3-methylphenyl)-[2,2'-dimethyl-1,1'-biphenyl]-4,4'-diamine, N,N'-diphenyl-N,N'-bis(3-methylphenyl)-pyrenyl-1,6-diamine, and the like.

Pyrazoline transport molecules as disclosed in U.S. Pat. No. 4,315,982, U.S. Pat. No. 4,278,746, and U.S. Pat. No. 3,837,851, the disclosures of each of which are totally incorporated herein by reference. Typical pyrazoline transport molecules include 1-[lepidyl-(2)]-3-(p-diethylaminophenyl)-5-(p-diethylaminophenyl)pyrazoline, 1-[quinolyl-(2)]-3-(p-diethylaminophenyl)-5-(p-diethylaminophenyl) pyrazoline, 1-[pyridyl-(2)]-3-(p-diethylaminostyryl)-5-(p-diethylaminophenyl) pyrazoline, 1-[6-methoxypyridyl-(2)]-3-(p-diethylaminostyryl)-5-(p-diethylaminophenyl) pyrazoline, 1-phenyl-3-[p-dimethylaminostyryl]-5-(p-dimethylaminostyryl) pyrazoline, 1-phenyl-3-[p-diethylaminostyryl]-5-(p-diethylaminostyryl)pyrazoline, and the like.

Substituted fluorene charge transport molecules as described in U.S. Pat. No. 4,245,021, the disclosure of which is totally incorporated herein by reference. Typical fluorene charge transport molecules include 9-(4'-dimethylaminobenzylidene)fluorene, 9-(4'-methoxybenzylidene)fluorene, 9-(2',4'-dimethoxybenzylidene)fluorene, 2-nitro-9-benzylidene-fluorene, 2-nitro-9-(4'-diethylaminobenzylidene)fluorene, and the like.

Oxadiazole transport molecules such as 2,5-bis(4-diethylaminophenyl)-1,3,4-oxadiazole, pyrazoline, imidazole, triazole, and the like. Other typical oxadiazole transport molecules are described, for example, in German Patent 1,058,836, German Patent 1,060,260, and German Patent 1,120,875, the disclosures of each of which are totally incorporated herein by reference.

Hydrazone transport molecules, such as p-diethylamino-benzaldehyde-(diphenylhydrazone), o-ethoxy-p-

146

diethylaminobenzaldehyde-(diphenylhydrazone), o-methyl-p-diethylaminobenzaldehyde-(diphenylhydrazone), o-methyl-p-dimethylaminobenzaldehyde-(diphenylhydrazone), 1-naphthalene-carbaldehyde 1-methyl-1-phenylhydrazone, 1-naphthalene-carbaldehyde 1,1-phenylhydrazone, 4-methoxynaphthlene-1-carbaldehyde 1-methyl-1-phenylhydrazone, and the like. Other typical hydrazone transport molecules are described, for example in U.S. Pat. No. 4,150,987, U.S. Pat. No. 4,385,106, U.S. Pat. No. 4,338,388, and U.S. Pat. No. 4,387,147, the disclosures of each of which are totally incorporated herein by reference. Carbazole phenyl hydrazone transport molecules such as 9-methylcarbazole-3-carbaldehyde-1,1-diphenylhydrazone, 9-ethylcarbazole-3-carbaldehyde-1-methyl-1-phenylhydrazone, 9-ethylcarbazole-3-carbaldehyde-1-ethyl-1-phenylhydrazone, 9-ethylcarbazole-3-carbaldehyde-1-ethyl-1-benzyl-1-phenylhydrazone, 9-ethylcarbazole-3-carbaldehyde-1,1-diphenylhydrazone, and the like. Other typical carbazole phenyl hydrazone transport molecules are described, for example, in U.S. Pat. No. 4,256,821 and U.S. Pat. No. 4,297,426, the disclosures of each of which are totally incorporated herein by reference.

Vinyl-aromatic polymers such as polyvinyl anthracene, polycacenaphthylene; formaldehyde condensation products with various aromatics such as condensates of formaldehyde and 3-bromoprene; 2,4,7-trinitrofluorenone, and 3,6-dinitro-N-t-butylphthalimide as described, for example, in U.S. Pat. No. 3,972,717, the disclosure of which is totally incorporated herein by reference.

Oxadiazole derivatives such as 2,5-bis-(p-diethylaminophenyl)-oxadiazole-1,3,4 described in U.S. Pat. No. 3,895,944, the disclosure of which is totally incorporated herein by reference.

Tri-substituted methanes such as alkyl-bis(N,N-dialkylaminoaryl)methane, cycloalkyl-bis(N,N-dialkylaminoaryl)methane, and cycloalkenyl-bis(N,N-dialkylaminoaryl)methane as described in U.S. Pat. No. 3,820,989, the disclosure of which is totally incorporated herein by reference.

9-Fluorenylidene methylene derivatives having the formula



wherein X and Y are cyano groups or alkoxy carbonyl groups; A, B, and W are electron withdrawing groups independently selected from the group consisting of acyl, alkoxy carbonyl, nitro, alkylaminocarbonyl, and derivatives thereof; m is a number of from 0 to 2; and n is the number 0 or 1 as described in U.S. Pat. No. 4,474,865, the disclosure of which is totally incorporated herein by reference. Typical 9-fluorenylidene methylene derivatives encompassed by the above formula include (4-n-butoxycarbonyl-9-fluorenylidene)malononitrile, (4-phenethoxycarbonyl-9-fluorenylidene) malononitrile, (4-carbitoxy-9-fluorenylidene) malononitrile, (4-n-butoxycarbonyl-2,7-dinitro-9-fluorenylidene)malonate, and the like.

Other charge transport materials include poly-1-vinylpyrene, poly-9-vinylanthracene, poly-9-(4-pentenyl)-carbazole, poly-9-(5-hexyl)-carbazole, polymethylene

pyrene, poly-1-(pyrenyl)-butadiene, polymers such as alkyl, nitro, amino, halogen, and hydroxy substitute polymers such as poly-3-amino carbazole, 1,3-dibromo-poly-N-vinyl carbazole, 3,6-dibromo-poly-N-vinyl carbazole, and numerous other transparent organic polymeric or non-polymeric transport materials as described in U.S. Pat. No. 3,870,516, the disclosure of which is totally incorporated herein by reference. Also suitable as charge transport materials are phthalic anhydride, tetrachlorophthalic anhydride, benzil, mellitic anhydride, S-tricyanobenzene, picryl chloride, 2,4-dinitrochlorobenzene, 2,4-dinitrochlorobenzene, 4-nitrobiphenyl, 4,4-dinitrophenyl, 2,4,6-trinitroanisole, trichlorotrinitrobenzene, trinitro-o-toluene, 4,6-dichloro-1,3-dinitrobenzene, 4,6-dibromo-1,3-dinitrobenzene, p-dinitrobenzene, chloranil, bromanil, and mixtures thereof, 2,4,7-trinitro-9-fluorenone, 2,4,5,7-tetranitrofluorenone, trinitroanthracene, dinitroacridene, tetracyanopyrrole, dinitroanthraquinone, polymers having aromatic or heterocyclic groups with more than one strongly electron withdrawing substituent such as nitro, sulfonate, sulfonyl, carboxyl, cyano, or the like, including polyesters, polysiloxanes, polyamides, polyurethanes, and epoxies, as well as block, graft, or random copolymers containing the aromatic moiety, and the like, as well as mixtures thereof, as described in U.S. Pat. No. 4,081,274, the disclosure of which is totally incorporated herein by reference.

Also suitable are charge transport materials such as triarylamines, including triaryl amine, of the formula



and the like, as disclosed in, for example, U.S. Pat. No. 3,240,597 and U.S. Pat. No. 3,180,730, the disclosures of each of which are totally incorporated herein by reference, and substituted diarylmethane and triarylmethane compounds, including bis-(4-diethylamino-2-methylphenyl)-phenylmethane, of the formula



and the like, as disclosed in, for example, U.S. Pat. No. 4,082,551, U.S. U.S. Pat. No. 3,755,310, U.S. Pat. No. 3,647,431, British Patent 984,965, British Patent 980,879, and British Patent 1,141,666, the disclosures of each of which are totally incorporated herein by reference.

A particularly preferred charge transport molecule is one having the general formula



wherein X, Y and Z are each, independently of the others, hydrogen, alkyl groups having from 1 to about 20 carbon atoms, or chlorine, and wherein at least one of X, Y and Z is independently selected to be an alkyl group having from 1 to about 20 carbon atoms or chlorine. If Y and Z are hydrogen, the compound can be named N,N'-diphenyl-N,N'-bis(alkylphenyl)-[1,1'-biphenyl]-4,4'-diamine wherein the alkyl is, for example, methyl, ethyl, propyl, n-butyl, or the like, or the compound can be N,N'-diphenyl-N,N'-bis(chlorophenyl)-[1,1'-biphenyl]-4,4'-diamine. A particularly preferred member of this class is N,N'-diphenyl-N,N'-bis(3"-methylphenyl)-[1,1'-biphenyl]-4,4'-diamine (prepared as disclosed in U.S. Pat. No. 4,265,990, the disclosure of which is totally incorporated herein by reference).

Any suitable and conventional technique may be utilized to mix and thereafter apply the charge transport layer coating mixture to the charge generating layer. Typical application techniques include spraying, dip coating, roll coating, wire wound rod coating, and the like. Drying of the deposited coating may be effected by any suitable conventional technique such as oven drying, infra red radiation drying, air drying and the like.

The charge transport material is present in the charge transport layer in any effective amount, generally from about 5 to about 90 percent by weight, preferably from about 20 to about 75 percent by weight, more preferably from about 20 to about 60 percent by weight, and even more preferably from about 30 to about 60 percent by weight, although the amount can be outside of these ranges.

Examples of the highly insulating and transparent resinous components or inactive binder resinous material for the transport layers include materials such as those described in U.S. Pat. No. 3,121,006, the disclosure of which is totally incorporated herein by reference. Specific examples of suitable organic resinous materials include polycarbonates, acrylate polymers, vinyl polymers, cellulose polymers, polyesters, polysiloxanes, polyamides, polyurethanes, polystyrenes, polyarylates, polyethers, polysulfones, and epoxies, as well as block, random or alternating copolymers thereof. Preferred electrically inactive binder materials include polycarbonate resins having a number average molecular weight of from about 20,000 to about 100,000 with a molecular weight in the range of from about 50,000 to about 100,000 being particularly preferred. The high performance polymers of the present invention can also be employed as the binder in the charge transport layer of the imaging member, either alone or in combination with other materials. Generally, the charge transport layer contains the charge transport material in an amount of from about 5 to about 90 percent by weight, and preferably from about 20 percent to about 75 percent by weight, although the relative amounts of binder and transport material can be outside these ranges.

Generally, the thickness of the charge transport layer is from about 10 to about 50 microns, although thicknesses outside this range can also be used. Preferably, the ratio of

149

the thickness of the charge transport layer to the charge generator layer is maintained from about 2:1 to 200:1, and in some instances as great as 400:1.

At least one layer of the imaging members of the present invention, such as the adhesive layer, the protective overcoat layer, the photogenerating layer, the charge transport layer, or the like, contains a polymer of the formulae indicated hereinbelow. The polymer can be present as the sole binder in the layer, or can be present as a component of a blend of two or more binder polymers. One example of a suitable polymer with which the polymers according to the present invention can be blended is a polycarbonate resin. Any desired or suitable polycarbonate resin can be selected. For example, polycarbonates of the general formula



wherein R and R' each, independently of the other, is an alkyl group (including cycloalkyl groups and substituted alkyl groups), typically with from 1 to about 30 carbon atoms, or a phenyl group (including substituted phenyl groups) and n is an integer representing the number of repeat monomer units, typically being from about 10 to about 1,000, although the value can be outside this range. Examples of particularly preferred polycarbonates for the present invention include poly(4,4'-isopropylidene-diphenylene) carbonate (also referred to as bisphenol-A-polycarbonate), poly(4,4'-diphenyl-1,1'-cyclohexane carbonate, and the like. Preferred polycarbonate resins have a number average molecular weight of from about 20,000 to about 150,000, with a number average molecular weight in the range of from about 50,000 to about 100,000 being particularly preferred. Preferred polycarbonate resins have a weight average molecular weight of from about 20,000 to about 100,000, with a weight average molecular weight in the range of from about 50,000 to about 100,000 being particularly preferred. Within the layer, the additional binder components, such as a polycarbonate, and the polymer according to the present invention can be blended in any suitable or desired relative amounts, typically from about 1 to about 99 percent by weight of the second binder polymer and from about 1 to about 99 percent by weight of the polymer according to the present invention, preferably from about 5 to about 95 percent by weight of the second binder polymer and from about 5 to about 95 percent by weight of the polymer according to the present invention, and more preferably from about 25 to about 75 percent by weight of the second binder polymer and from about 25 to about 75 percent by weight of the polymer of the present invention, although the relative amounts can be outside these ranges.

Other layers, such as conventional electrically conductive ground strip along one edge of the belt in contact with the conductive layer, blocking layer, adhesive layer or charge generating layer to facilitate connection of the electrically conductive layer of the photoreceptor to ground or to an electrical bias, may also be included. Ground strips are well known and usually comprise conductive particles dispersed in a film forming binder.

Optionally, an overcoat layer may also be utilized to improve resistance to abrasion. In some cases an anti-curl back coating may be applied to the surface of the substrate opposite to that bearing the photoconductive layer to provide flatness and/or abrasion resistance. These overcoating and

150

anti-curl back coating layers are well known in the art and may comprise thermoplastic organic polymers or inorganic polymers that are electrically insulating or slightly semi-conductive. Overcoatings are continuous and generally have a thickness of less than about 10 micrometers. The thickness of anti-curl backing layers should be sufficient to substantially balance the total forces of the layer or layers on the opposite side of the supporting substrate layer. The total forces are substantially balanced when the belt has no noticeable tendency to curl after all the layers are dried. For example, for an electrophotographic imaging member in which the bulk of the coating thickness on the photoreceptor side of the imaging member is a transport layer containing predominantly polycarbonate resin and having a thickness of about 24 microns on a Mylar substrate having a thickness of about 76 microns, sufficient balance of forces can be achieved with a 13.5 micrometers thick anti-curl layer containing about 99 percent by weight polycarbonate resin, about 1 percent by weight polyester and between about 5 and about 20 percent of coupling agent treated crystalline particles. An example of an anti-curl backing layer is described in U.S. Pat. No. 4,654,284 the disclosure of which is totally incorporated herein by reference. A thickness between about 70 and about 160 microns is a satisfactory range for flexible photoreceptors. Polymers of the present invention are also suitable for use as overcoat layers and anticurl back coating layers.

The present invention also encompasses a method of generating images with the photoconductive imaging members disclosed herein. The method comprises the steps of generating an electrostatic latent image on a photoconductive imaging member of the present invention, developing the latent image, and transferring the developed electrostatic image to a substrate. Optionally, the transferred image can be permanently affixed to the substrate. Development of the image may be achieved by a number of methods, such as cascade, touchdown, powder cloud, magnetic brush, and the like. Transfer of the developed image to a substrate may be by any method, including those making use of a corotron or a biased charging roll. The fixing step may be performed by means of any suitable method, such as radiant flash fusing, heat fusing, pressure fusing, vapor fusing, and the like. Any material used in xerographic copiers and printers may be used as a substrate, such as paper, transparency material, or the like.

The polyarylene ether alcohols of the present invention exhibit advantages such as high thermal stability, good hydrolytic stability, high glass transition temperatures, compatibility with charge transport molecules such as N,N'-diphenyl-N,N'-bis(3"-methylphenyl)-(1,1'-biphenyl)-4,4'-diamine, good mobility of charge holes through layers comprising the material, good wear resistance, and the like.

Specific embodiments of the invention will now be described in detail. These examples are intended to be illustrative, and the invention is not limited to the materials, conditions, or process parameters set forth in these embodiments. All parts and percentages are by weight unless otherwise indicated.

151

## EXAMPLE I

A polymer of the formula



(hereinafter referred to as poly(4-FPK-FBPA)) wherein n is about 130 and represents the number of repeating monomer units was prepared as follows. A 1-liter, 3-neck round-bottom flask equipped with a Dean-Stark trap (Barrett) trap, condenser, mechanical stirrer, argon inlet, and stopper was situated in a silicone oil bath. 4,4'-Difluorobenzophenone (Aldrich Chemical Co., Milwaukee, Wis., 43.47 grams, 0.1992 mole), 9,9'-bis(4-hydroxyphenyl)fluorenone (Aldrich, 75.06 grams, 0.2145 mole) potassium carbonate (65.56 grams), anhydrous N,N-dimethylacetamide (300 milliliters), and toluene (52 milliliters) were added to the flask and heated to 175° C. (oil bath temperature) while the volatile toluene component was collected and removed. After 5 hours of heating at 175° C. with continuous stirring, the reaction mixture was allowed to cool to 25° C. The solidified mass was extracted with methylene chloride, filtered and added to methanol to precipitate the polymer, which was collected by filtration, washed with water, and washed with methanol. The yield of vacuum dried product, poly(4-FPK-FBPA), was 71.7 grams. The polymer was analyzed by gel permeation chromatography with tetrahydrofuran as the elution solvent with the following results:  $M_n=59,100$ ,  $M_{peak}=144,000$ , and  $M_w=136,100$ . The glass transition temperature of the polymer was 240° C., as determined by using differential scanning calorimetry at a heating rate of 20° C. per minute. Solution cast films from methylene chloride were clear, tough, and flexible. As a result of the stoichiometries used in the reaction, it is believed that this polymer had hydroxyl end groups derived from fluorenone bisphenol.

## EXAMPLE II

A polymer of the formula



was prepared as follows. A 1-liter, 3-neck round-bottom flask equipped with a condenser, mechanical stirrer, argon inlet, and rubber septum was situated in a silicone oil bath. Poly(4-FPK-FBPA) (10 grams, prepared as described in Example I) in tetrahydrofuran (200 grams) was added, followed by 1 molar borane-tetrahydrofuran complex (Aldrich Chemical Co., Milwaukee, Wis., 83.5 grams). The resultant solution gelled. After refluxing the gel with mechanical stirring for 2 hours, the reaction mixture was allowed to cool and remain at 25° C. for 16 hours. Methanol

152

was then cautiously added dropwise to react with residual borane. The solid residue was filtered off, washed with water, and then vacuum dried. Tetrahydrofuran (300 milliliters) was added to the solid, which did not dissolve until acetic acid (20 milliliters) was added. The solution (in portions of 25 milliliters) was added to water (750 milliliters for each 25 milliliter portion of polymer solution) using a Waring blender to precipitate a white polymer. The polymer was filtered, washed extensively with water, filtered, washed with methanol, filtered, and then vacuum dried. The polymer dissolved in tetrahydrofuran but was insoluble in methylene chloride, ethyl acetate, toluene, and methyl isobutyl ketone. When dissolved in tetrahydrofuran (8.5 grams), the hydroxylated polymer (1.2 grams) with N,N'-diphenyl-N,N'-bis(3"-methylphenyl)-(1,1'-biphenyl)-4,4'-diamine (1.2 grams) was used to coat 25 micron charge (hole) transport layers for organic photoreceptors with hydroxygallium phthalocyanine photogenerator layers. Moreover, the addition of 0.1 gram of hexane diisocyanate to the above coating solution was found to improve markedly the electrical properties of the device.

The above reaction was repeated using 19.7 grams of poly(4-FPK-FBPA) in tetrahydrofuran (400 grams) and 1 molar borane-tetrahydrofuran complex in tetrahydrofuran (215 grams). After 2 hours reflux and 16 hours at 25° C., the reaction mixture was cautiously treated with methanol and then acetic acid, followed by addition to water to reprecipitate the polymer. The polymer was filtered, washed with water, washed with methanol, and then vacuum dried.

## EXAMPLE III

A polymer of the formula



was prepared as follows. To a 5-liter 3-neck round-bottom flask equipped with a mechanical stirrer, reflux condenser, argon inlet and stopper that was situated in a silicone oil bath were added sequentially, acetyl chloride (388 grams, 320 milliliters), dimethoxymethane (450 milliliters), methanol (12.5 milliliters), tetrachloroethane (500 milliliters), and poly(4-FPK-FBPA) (100 grams, obtained from Scientific Polymer Products) in tetrachloroethane (1250 milliliters). To this mixture was then added tin tetrachloride (5 milliliters) via an air-tight syringe. The reaction mixture was heated for 2 hours at between 90 and 100° C. oil bath set temperature. After cooling to 25° C., the reaction mixture was added to methanol to reprecipitate the polymer with 0.96 chloromethyl groups per repeat unit.

153  
EXAMPLE IV

A polymer of the formula



was prepared as follows. Chloromethylated poly(4-FPK-FBPA) (prepared as described in Example III, 78.5 grams) in N,N-dimethylacetamide (1,967 grams) was added to a 5-liter, 3-neck, round-bottom flask equipped with a mechanical stirrer, argon inlet and condenser and situated in a silicone oil bath. Sodium acetate (78.5 grams) was added and the reaction mixture was heated for 24 hours at 100° C. The reaction solution was then added to water to precipitate the polymer product, which was filtered and washed with methanol. In a similar procedure, the same polymer was prepared by magnetically stirring chloromethylated poly(4-FPK-FBPA) (25 grams, prepared as described in Example III) in N,N-dimethylacetamide (700 grams) with sodium acetate (15 grams, Aldrich) for one month at 25° C. The reaction solution was then decanted from the insoluble salts that settled on centrifugation, and was added to methanol to precipitate a white polymer that was filtered, washed with water, washed with methanol, and then vacuum dried. The yield was 12.2 grams.

## EXAMPLE V

A polymer of the formula



was prepared as follows. The acetylated polymer (50 grams, prepared as described in Example IV) in tetrahydrofuran (2,000 grams) was allowed to react with 1-molar borane-tetrahydrofuran complex in tetrahydrofuran (250 milliliters, Aldrich) at reflux for 1 hour. The reaction vessel was a 5-liter, 3-neck, round-bottom flask that was situated in a silicone oil bath and equipped with a mechanical stirrer, condenser, argon inlet, and rubber septum. Methanol was added to neutralize unreacted borane and acetic acid was added to form a solution of the polymer. The reaction mixture was then added to water to precipitate a white polymer that was filtered, washed with water, washed with methanol, and then vacuum dried. The polymer product dissolved in tetrahydrofuran and in a solution of 1-part ethanol to 9-parts tetrahydrofuran.

154  
EXAMPLE VI

A polymer of the formula



10 was prepared as follows. A 5-liter, 3-neck round-bottom flask equipped with a Dean-Stark trap (Barrett) trap, condenser, mechanical stirrer, argon inlet, and stopper was situated in a silicone oil bath. 4,4'-Dichlorobenzophenone (Aldrich, 403.95 grams), bisphenol A (Aldrich, 340.87 grams), potassium carbonate (491.7 grams), anhydrous N,N-dimethylacetamide (2,250 milliliters), and toluene (412.5 milliliters, 359.25 grams) were added to the flask and heated to 170° C. (oil bath temperature) while the volatile toluene component was collected and removed. After 48 hours of heating at 170° C. with continuous stirring, the reaction mixture was allowed to cool to 25° C. The reaction mixture was thereafter filtered to remove insoluble salts, and the solution was then added to methanol to precipitate the polymer. The polymer was isolated by filtration, washed with water, washed with methanol, and then vacuum dried.

## EXAMPLE VII

A polymer of the formula



30 was prepared as follows. Poly(arylene ether ketone) (prepared as described in Example VI, 5 grams) in dioxane (50 milliliters) was treated with 1 molar borane-tetrahydrofuran complex in tetrahydrofuran (50 milliliters). 40 Heating with stirring at 70° C. was carried out for about 4 hours. The polymer solution gelled at 25° C. within 10 minutes after all the borane solution had been added. Vigorous gas evolution was observed. The polymer was treated with methanol and the polymer dissolved with gas evolution. 45 The reaction mixture was concentrated using a rotary evaporator and was added to water to precipitate a polymer that was extensively washed with water and then with methanol. After vacuum drying, the yield of polymer was 4.6 grams.

## EXAMPLE VIII

A polymer of the formula



55 was prepared by adding 2-isocyanato-ethyl methacrylate (0.18 gram, Aldrich) to the polyarylene ether alcohol (prepared in Example VII, 0.5 gram) in tetrahydrofuran (3.76 grams). A photoreceptor charge transport layer was 60 made by adding N,N'-diphenyl-N,N'-bis(3"-methylphenyl)-

**155**

(1,1'-biphenyl)-4,4'-diamine) (0.5 gram) to the solution. When coated on a hydroxygallium binder generator layer at 29 microns ( $\pm 5$  microns) and tested on a flat plate xerographic scanner, the  $V_0$  was 1,020 volts, the dark decay was 60 volts, and the residual voltage after light exposure was 60 volts.

**EXAMPLE IX**

A polymer of the formula



was prepared as follows. To a 5-liter 3-neck round-bottom flask equipped with a mechanical stirrer, reflux condenser, argon inlet and stopper that was situated in an ice bath were added sequentially, acetyl chloride (184 grams), dimethoxymethane (225 milliliters, 193 grams), methanol (6.25 milliliters), methylene chloride (500 milliliters), and poly(4-CPK-BPA) (75 grams, prepared as described in Example VIII) in methylene chloride (625 milliliters). To this mixture was then added tin tetrachloride (6.5 milliliters) via an air-tight syringe. The reaction mixture was heated for 4 hours at 55° C. oil bath set temperature. After cooling to 25° C., the reaction mixture was added to methanol to reprecipitate the polymer with 0.96 chloromethyl groups per repeat unit.

**EXAMPLE X**

A polymer of the formula



was prepared as follows. A 500-milliliter, 3-neck round-bottom flask equipped with a Dean-Stark trap (Barrett) trap, condenser, mechanical stirrer, argon inlet, and stopper was situated in a silicone oil bath. 4,4'-Difluorobenzophenone (Aldrich, 21.82 grams), bisphenol A (Aldrich, 2.64 grams), potassium carbonate (40 grams), anhydrous N,N-dimethylacetamide (300 milliliters), and toluene (52 milliliters) were added to the flask and heated to 175° C. (oil bath temperature) while the volatile toluene component was collected and removed. After 5 hours of heating at 175° C. with continuous stirring, phenol (5 grams) was added and the reaction mixture was heated and stirred at 175° C. for 30 more minutes. The reaction mixture was then allowed to cool to 25° C. The solidified mass was extracted with methylene chloride (500 milliliters) and filtered to remove insoluble salts. The solution was concentrated using a rotary evaporator and then was added to methanol to precipitate the polymer. The polymer was isolated by filtration, washed with water, washed with methanol, and then vacuum dried. The yield of vacuum dried product, poly(4-FPK-BPA) was 40 grams.

**156****EXAMPLE XI**

A polymer of the formula



5

was prepared as follows. To a 1-liter 3-neck round-bottom flask equipped with a mechanical stirrer, reflux condenser, argon inlet and stopper that was situated in a silicone oil bath were added sequentially, acetyl chloride (140.1 grams, 128 milliliters), dimethoxymethane (157.6 grams), methanol (5 milliliters), tetrachloroethane (500 milliliters), and poly(4-FPK-BPA) (40 grams, prepared as described in Example X) in tetrachloroethane (500 milliliters). To this mixture was then added tin tetrachloride (0.6 milliliter) via an air-tight syringe. The reaction mixture was heated for 2 hours at 110° C. oil bath set temperature. After cooling to 25° C., the reaction mixture was added to methanol to reprecipitate the polymer with 1.44 chloromethyl groups per repeat unit.

**EXAMPLE XII**

A polymer of the formula



35

was prepared as follows. The chloromethylated polymer (prepared as described in Example IX, 15 grams) in N,N-dimethylacetamide (300 milliliters) was magnetically stirred with sodium acetate (Aldrich, 9 grams) for one month. The reaction mixture was then centrifuged, and the reaction solution was decanted off from residual salts. The solution was added to water to precipitate a white polymer that was filtered, washed with water, washed with methanol, and then vacuum dried.

**EXAMPLE XIII**

A polymer of the formula



50

55

60

65

65

was prepared as follows. The chloromethylated polymer (1.44 CH<sub>2</sub>Cl groups per repeat unit, prepared as described in Example XI, 15 grams) in N,N-dimethylacetamide (283 grams) was magnetically stirred with sodium acetate (Aldrich, 9 grams) for one month. The reaction mixture was then centrifuged, and the reaction solution was decanted off from residual salts. The solution was added to water to precipitate a white polymer that was filtered, washed with water, washed with methanol, and then vacuum dried. The

157

polymer in methylene chloride was reprecipitated into methanol, filtered, and then vacuum dried.

## EXAMPLE XIV

A polymer of the formula



was prepared with the chloromethylated polymer (prepared as described in Example XI, 2 grams) in dioxane (50 milliliters) to which was added 1 molar borane-tetrahydrofuran complex (50 milliliters). The solution gelled within 10 minutes at 25° C. The reaction mixture was heated at between 70–80 minutes for 2 hours. Methanol was cautiously added with vigorous gas evolution, and the resultant solution was added to water to precipitate the polymer product. The white polymer was filtered, washed with water, washed with methanol, and then vacuum dried. The polymer (0.5 grams) in tetrahydrofuran (4.5 grams) was roll milled with titanium dioxide (MT500, 0.5 grams) and 60 grams of stainless steel shot for 16 hours. The dispersion was coated using a 0.5 mil Bird applicator on metallized polyethylene terephthalate film and heated from 40 to 150° C. over 40 minutes. A photogenerator layer of hydroxygallium phthalocyanine dispersed in polystyrene-vinyl pyridine in toluene was coated using a 0.25 Bird applicator, and the coating was heated for 5 minutes at 135° C. A charge transport layer solution consisting of N,N'-diphenyl-N,N'-bis(3'-methylphenyl)-(1,1'-biphenyl)-4,4'-diamine (1.2 grams) in polycarbonate (1.2 grams) in methylene chloride (13.45 grams) was coated over the binder generator layer using a 4 mil Bird applicator. The device was dried from 40 to 100° C. over 30 minutes.

## EXAMPLE XV

A polymer of the formula



was prepared as follows. The hydroxymethylated-<sup>65</sup> polyarylene ether alcohol (prepared as described in Example XIV, 1.0 gram) was allowed to react with 2-isocyanoethyl

methacrylate (1.10 grams) in N-methylpyrrolidinone (9 grams) for 16 hours.

## EXAMPLE XVI

A. Binder Generator Layer preparation

Several photogenerator layers containing hydroxygallium phthalocyanine pigment particles were prepared by forming coatings using conventional coating techniques on a substrate comprising a 200 Angstrom thick vacuum deposited titanium layer on a 3 mil thick polyethylene terephthalate film (Melinex®, obtained from ICI). The first coating was a siloxane charge blocking layer formed from hydrolyzed 5 g a m m a - a m i n o p r o p y l t r i e t h o x y s i l a n e (3-aminopropyltriethoxysilane) having a thickness of 0.03 micron (300 Angstroms). This film was coated as follows: 10 3-aminopropyltriethoxysilane (obtained from PCR Research Chemicals, Fla.) was mixed in ethanol in a 1:50 by volume ratio. A film of the resulting solution was applied to the 15 substrate in a wet thickness of 0.5 mil using a Bird applicator. The layer was then allowed to dry for 5 minutes at 25° C., followed by curing for 10 minutes at 110° C. in a forced 20 air oven. The second coating was an adhesive layer of 25 polyester resin (49,000 adhesive, obtained from E.I. Du Pont de Nemours and Co.) having a thickness of 0.04 micron (400 Angstroms) and was coated as follows: 0.5 gram of 49,000 30 polyester resin was dissolved in 70 grams of tetrahydrofuran and 29.5 grams of cyclohexanone. A film of the resulting solution was coated onto the barrier layer by a 0.5 mil Bird 35 applicator and cured in a forced air oven for 10 minutes. The adhesive interface layer was thereafter coated with a photogenerating layer containing 40 percent by volume hydroxygallium phthalocyanine and 60 percent by volume of a block copolymer of styrene (82 percent by weight)/4-vinyl pyridine (18 percent by weight) having a Mw of 11,900.

This photogenerating coating composition was prepared by dissolving 1.5 grams of the block copolymer of styrene/4-vinyl pyridine in 42 milliliters of toluene. To this solution was added 1.33 grams of hydroxygallium phthalocyanine and 300 grams of 1/8 inch diameter stainless steel shot. This mixture was then placed on a roll mill for 20 hours. The

resulting slurry was thereafter applied to the adhesive layer with a Bird applicator to form a layer having a wet thickness of 0.25 mil. This photogenerating layer was dried at 135° C.

for 5 minutes in a forced air oven to form a layer having a dry thickness of 0.5 micron.

#### B. Makrolon® Control Transport Layer Preparation

A charge transport layer was coated onto the hydroxygallium phthalocyanine generator layer of one of the imaging members thus prepared in XVIA. The transport layer was formed by using a Bird coating applicator to apply a solution containing 2 grams of N,N'-diphenyl-N,N'-bis(3"-methylphenyl)-(1,1'-biphenyl)-4,4'-diamine) (charge transport material, prepared as disclosed in U.S. Pat. No. 4,265,990, the disclosure of which is totally incorporated herein by reference) and 2 grams of polycarbonate resin [poly(4,4'-isopropylidene-diphenylene carbonate (available as MakrolonR from Farbenfabriken Bayer A.G.)] dissolved in 22.44 grams of methylene chloride. The N,N'-diphenyl-N,N'-bis(3"-methylphenyl)-(1,1'-biphenyl)-4,4'-diamine) is an electrically active aromatic diamine charge transport small molecule, and the polycarbonate resin is an electrically inactive film-forming binder. The coated device was dried at 80° C. for 30 minutes in a forced air oven to form a dry 25 micron thick charge transport layer.

#### C. Charge Transport Layer Preparation with Polymers of the Invention

Charge transport layers were coated onto the hydroxygallium phthalocyanine photogenerator layers of imaging members thus prepared in XVIA. Charge transport solutions were prepared in each instance by introducing into an amber glass bottle, 2.00 grams of N,N'-diphenyl-N,N'-bis(3"-methylphenyl)-(1,1'-biphenyl)-4,4'-diamine), 2.00 grams of one of each of the polymers of Examples I, II, V, VII, VIII, and XVIII, and 22.44 grams of the solvent indicated in the table below and admixing the contents to prepare the solutions. In some instances, hexane diisocyanate was also present in the charge transport solution in the amount indicated in the table below (number shown is percent by weight of the hexane diisocyanate present in the solution). The charge transport solutions were applied to the photogenerator layers with an 8 mil gap Bird applicator to form a coating which was heated from 40 to 100° C. over 30 minutes to dry the layer. The charge transport layers thus applied to the imaging members had dry coating thicknesses of about 25 microns.

#### D. Imaging Member Testing

The imaging members thus prepared were mounted on a cylindrical aluminum drum having a diameter of 242.6 millimeters (9.55 inches) which was rotated on a shaft. The test samples were taped onto the drum. When rotated, the drum carrying the samples produced a constant surface speed of 76.3 centimeters (30 inches) per second. A direct current pin corotron, an exposure light, an erase light, and five electrometer probes were mounted around the periphery of the mounted photoreceptor samples. The sample charging time was 33 milliseconds. Both expose and erase lights were broad band white light (400-700 nanometer) outputs, each supplied by a 300 Watt output xenon arc lamp. The relative locations of the probes and lights are indicated in the table below:

| Element    | Angle (degrees) | Position (mm) | Distance from Photoreceptor (mm) |
|------------|-----------------|---------------|----------------------------------|
| 5 Charge   | 0               | 0             | 18 pins<br>12 shield             |
| Probe 1    | 22.5            | 47.9          | 3.17                             |
| Expose     | 56.25           | 118.8         | N.A.                             |
| Probe 2    | 78.75           | 166.8         | 3.17                             |
| 10 Probe 3 | 168.75          | 356.0         | 3.17                             |
| Probe 4    | 236.25          | 489.0         | 3.17                             |
| Erase      | 258.75          | 548.0         | 125.00                           |
| Probe 5    | 303.75          | 642.9         | 3.17                             |

15 The surface potentials were measured as a function of time by the capacitively coupled probes. The probes were calibrated by applying known potentials to the drum substrate. The test samples were first rested in the dark for at least 60 minutes to ensure achievement of equilibrium with the testing conditions of 21.1° C. and 40.0 percent relative humidity. Each sample was then negatively charged in the dark to a development potential of about 900 volts. The charge acceptance of each sample and its residual potential after discharge by front erase exposure to 400 ergs per square centimeter were recorded. The test procedure was 20 repeated to determine the photoinduced discharge characteristic of each sample (PIDC) by different light energies of up to 20 ergs per square centimeter. Process speed was 60.0 imaging cycles per minute. The films on the drum were then exposed and erased by light sources located at appropriate 25 positions around the drum. The measurement consisted of charging the photoconductor devices in a constant current or voltage mode. As the drum rotated, the initial charging potential was measured by probe 1. Further rotation led to the exposure station, where the photoconductor devices 30 were exposed to monochromatic radiation of known intensity. The surface potential after exposure was measured by probes 2 and 3. The devices were finally exposed to an erase lamp of appropriate intensity and any residual potential was measured by probe 4. The process was repeated with the 35 magnitude of the exposure automatically changed during the next cycle. A photo-induced discharge characteristics curve was obtained by plotting the potentials at probes 2 and 3 as a function of exposure. The initial slope of the discharge curve is termed S in units of (volts×cm<sup>2</sup>/ergs) and the 40 residual potential after the erase step is termed V<sub>r</sub>. The devices were cycled continuously for 10,000 cycles of charge, expose, and erase steps to determine the cyclic 45 stability. Charge trapping in the transport layer results in a build up of residual potential known as cycle-up. The 50 sensitivity data and the residual cycle-up for the four samples is shown in the Table below. S represents the initial slope of the Photo-Induced Discharge Characteristics (PIDC) and is a measure of the sensitivity of the device. 55 Cycle-up is the increase in residual potential in 10,000 cycles of continuous operation. The negative numbers of the residual cycle-up resulted from an increase in sensitivity of the pigment in the generator layer as the device was cycled. Some of the residual electrical voltages of the imaging members with charge transport layers containing the polymer binders of the present invention were slightly higher 60 after flood exposure than that of the imaging member with the charge transport layer containing the polycarbonate binder. The residual voltages of the imaging members containing the polymers of the present invention, however, 65 gradually decreased during subsequent tests and aging. The results are summarized in the following table. Film peel strength and mechanical properties of the layers containing

## 161

the polymers of the present invention were good as determined by manual manipulations. The numbers indicate that the transport layers of N,N'-diphenyl-N,N'-bis(31-methylphenyl)-1,1'-biphenyl-4,4'-diamine dispersed in the binders of the present invention were trap free. The absence of traps suggest that the diamine dispersed well in all three of these binders.

| Binder                                       | S   | PIDC | 1 sec.<br>Dark<br>Decay | Cyclic<br>Charac-<br>teristics | V <sub>0</sub> |
|----------------------------------------------|-----|------|-------------------------|--------------------------------|----------------|
| Example I (THF)                              | 227 | 108  | 47                      | 330                            | 799            |
| Example I (CH <sub>2</sub> Cl <sub>2</sub> ) | 240 | 33   | 109                     | 17                             | 804            |
| Example I (THF)                              | 233 | 230  | 30                      | 41                             | 796            |
| Example I (CH <sub>2</sub> Cl <sub>2</sub> ) | 226 | 79   | 74                      | -89                            | 799            |
| Example I (CH <sub>2</sub> Cl <sub>2</sub> ) | 213 | 45   | 48                      | -39                            | 801            |
| Example I (THF) + HDI (0.1)                  | 202 | 83   | 53                      | -10                            | 804            |
| Example II (THF)                             | 209 | 47   | 42                      | -3                             | 599            |
| Example II (THF)                             | 252 | 234  | 29                      | 266                            | 797            |
| Example II (THF)                             | 285 | 98   | 93                      | 171                            | 799            |
| Example XVIII (THF) + HDI (0.1)              | 271 | 37   | 62                      | 12                             | 800            |
| Example XVIII (THF) + HDI (0.2)              | 255 | 27   | 58                      | -4                             | 800            |
| Example XVIII (THF) + HDI (0.4)              | 240 | 31   | 56                      | -18                            | 802            |
| Example XVIII (THF) + HDI (0.1)              | 289 | 5    | 85                      | 7                              | 797            |
| Example XVIII (THF) + HDI (0.2)              | 343 | 13   | 133                     | -10                            | 595            |
| Example V                                    | 162 | 163  | 85                      | 69                             | 591            |
| Example VII                                  | 164 | 74   | 102                     | -37                            | 780            |
| Example VIII                                 | 127 | 18   | 68                      | -7                             | 592            |
| Control, TBD/Makrolon                        | 363 | 30   | 66                      | -2                             | 798            |
| Control, TBD/Makrolon                        | 359 | 5    | 291                     | 2                              | 801            |
| Control, TBD/Makrolon                        | 314 | 29   | 63                      | 11                             | 801            |
| Control, TBD/Makrolon                        | 357 | 2    | 220                     | 2                              | 589            |

## EXAMPLE XVII

Four electrophotographic imaging members were prepared by applying by dip coating a charge blocking layer onto the rough surface of eight aluminum drums having a diameter of 4 centimeters and a length of 31 centimeters. The blocking layer coating mixture was a solution containing 8 weight percent polyamide (Nylon 6) dissolved in 92 weight percent butanol, methanol, and water solvent mixture. The butanol, methanol, and water mixture percentages were 55, 36, and 9 percent by weight, respectively. The coating was applied at a coating bath withdrawal rate of 300 millimeters per minute. After drying in a forced air oven, the blocking layers had thicknesses of 1.5 microns. The dried blocking layers were coated with a charge generating layer containing 2.5 weight percent hydroxygallium phthalocyanine pigment particles, 2.5 weight percent polyvinylbutyral

## 162

film forming polymer, and 95 weight percent cyclohexanone solvent. The coatings were applied at a coating bath withdrawal rate of 300 millimeters per minute. After drying in a forced air oven, the charge generating layers had thicknesses of 0.2 micrometers. The drums were subsequently coated with charge transport layers containing N,N'-diphenyl-N,N'-bis(3-methylphenyl)-1,1'-biphenyl-4,4'-diamine (TPD) dispersed in a binder of polycarbonate (PCZ200, obtained from Mitsubishi Chemical Company) (control) or one of the polymers of the present invention (one each of Example VII, Example VIII, Example XII, a polymer prepared as described in Example XII and subsequently reduced to



by the process described in Example II, and a polymer prepared as described in Example XII and subsequently reduced to



35

by the process of Example V or Example XIV). The coating mixtures contained 8 weight percent N,N'-diphenyl-N,N'-bis(3-methylphenyl)-1,1'-biphenyl-4,4'-diamine, 12 weight percent binder, and 80 weight percent monochlorobenzene solvent. The coatings were made in a Tsukiage dip coating apparatus. After drying in a forced air oven for 45 minutes at 118° C., the transport layers had thicknesses of 20 microns.

## EXAMPLE XVIII

50 A crosslinked charge transport layer with a high hole mobility, a good PIDC, and a low V<sub>r</sub> was prepared by reacting a polyarylene ether alcohol with a polyisocyanate. The chemistry was as follows:



-continued



The binder resin was compatible with the charge transport material *N,N'*-diphenyl-*N,N'*-bis(3"-methylphenyl)-(1,1'-biphenyl)-4,4'-diamine) and was soluble in tetrahydrofuran (THF) and monochlorobenzene (mCB), which are common organic photoconductor coating solvents. The formulation evaluated was a solution of the polyarylene ether alcohol (4.7 grams, prepared as described in Example II) and the charge transport material (4.7 grams) in THF (33.3 grams) (or mixtures of THF with mCB) to which had been added hexane diisocyanate (between 0.39 and 3.9 grams), coated onto imaging members prepared as described in Example XVIA to form flexible belt imaging members. The charge transport layer coating formulation with the diisocyanate crosslinking agent (hexane diisocyanate) had a reasonable potlife (that is, in excess of 2 weeks at 25° C.).

The electrical properties of these belts were tested. Sample I (a control sample) consisted of hydroxylgallium phthalocyanine binder generator layer overcoated with a solution of Makrolon (1.2 grams) and the charge transport molecule (1.2 grams) in methylene chloride (11.22 grams). Sample C consisted of the polyarylene ether alcohol (1.2 grams, with the above structure), the charge transport molecule (1.2 grams) and hexane diisocyanate (0.1 grams) in tetrahydrofuran (8.5 grams). Sample D consisted of the polyarylene ether alcohol (1.2 grams, with the above structure), the charge transport molecule (1.2 grams), and hexane diisocyanate (0.19 grams) in tetrahydrofuran (8.5 grams). Sample E consisted of the 15 polyarylene ether alcohol (1.2 grams, with the above structure), the charge transport molecule (1.2 grams), and hexane diisocyanate (0.38 grams) in tetrahydrofuran (8.5 grams). The table below summarizes the electrical results. The mobilities (cm<sup>2</sup>/V-sec) are very close to those of the charge transport molecule in polycarbonate, and are of sufficient magnitude down to small fields which ensures rapid transit times. The PIDCs soften with increasing hexane diisocyanate (HDI) content. It is believed that some of the softening should disappear if the thicknesses of the devices that contain the new transport layer (see IV slope in the table; thicknesses were around 21 microns instead of 25 to 28 microns). The different solvent system may also have promoted this tendency of PIDC softening. Other electrical properties were close to or as good as those of the control device. The only parameter that deviated significantly was the cycle-down. It should be noted, however, that (1) the new devices start with significantly lower dark decay than the control device (around 40V vs. 70V for 0.6 s dark decay (the dark decay values in the cycling experiments are not normalized)); and (2) most of the cycle-down occurs at the beginning and seems to saturate at higher cycle numbers, e.g., for C the dark decay is 48, 64, 74, 94, 94, and 90V for 0.4k, 2.4k, 4k, 6k, 8k, and 10k cycles respectively. In summary, the new transport layers affect very little the underlying generation layer and are at

15 least two orders faster than other crosslinked transport layer systems.

| Sample                                  | I   | C   | D   | E   |
|-----------------------------------------|-----|-----|-----|-----|
| Sensitivity                             | 314 | 271 | 255 | 240 |
| Expos. 3.8 ergs/cm <sup>2</sup> (volts) | 68  | 95  | 103 | 159 |
| Expos. 6 ergs/cm <sup>2</sup> (volts)   | 46  | 59  | 55  | 85  |
| Dark Decay (1 second) (volts)           | 63  | 62  | 58  | 56  |
| 25 Depletion (at 10,000)                | 38  | 6   | 1   | 8   |
| IV Slope                                | 56  | 43  | 40  | 41  |
| Cycle-up (10,000) (volts)               | 9   | 25  | 4   | -5  |
| Cycle-down (10,000) (volts)             | -16 | 41  | 49  | 62  |

Two drum imaging members were also prepared by the method described in Example XVII, with the following exceptions. The charge transport layer coating solution contained 56.25 weight percent tetrahydrofuran, 18.75 weight percent monochlorobenzene, 0.00042 weight percent silicone oil, 7.5 weight percent of a triarylamine of the formula



3.75 weight percent of the charge transport molecule employed in Example XVII, 12.5 weight percent of the binder (in one instance, the crosslinking polymer solution described hereinabove, in the other instance, PCZ 300 polycarbonate, obtained from Mitsubishi Chemical Co.), 1 weight percent 2,2'-methylenebis(6-tert-butyl-4-methylphenol) antioxidant, and 0.25 weight percent bht antioxidant. The undercoat layer coating solution contained 6.2 parts by weight gamma aminopropyl triethoxy silane, 45.8 parts by weight tributoxy zirconium acetylacetone, 3.2 parts by weight polyvinyl butyral, and 58.8 parts by weight 1-butanol, humidified during drying, with a dry thickness of 1.5 microns, as described in, for example, U.S. Pat. No. 5,449,573. The layers were coated in a Tsukiage dip coating apparatus with the crosslinkable charge transporting

solution at about 21 microns. The drums were then heated at 120° C. for 45 minutes. The electrical properties (PIDC curves) for the drum of the present invention were very good. The wear rate from a bias charging roll of the organic photoconductor drum with 3.9 grams hexane diisocyanate was 5.5 microns per 100 kilocycles. This value corresponds to a bias charging roll wear life at the standard 25 micron charge transport layer thickness of: 5

[{(25 micron original CT layer)-(12 microns maximum that can wear off and still have a useful imaging member)} $\times 100$  Kcycles] $+5.5=240$  kilocycles.

For a 30 micron thick original CT layer, the corresponding value is 330 kilocycles. When used in combination with a Luckamide® overcoat, the anticipated wear life of an overcoated crosslinked CTL device of the present invention is expected to be about 560 kilocycles. Moreover, there is the possibility of coating the crosslinked charge transport layer even thicker because the crosslinked charge transport layer will not redissolve in successive dips. 15 20

Organic photoreceptor drums were coated with charge transport layers made with polyarylene ether alcohol (4.7 grams, prepared as described in Example II) and the charge transport material N,N'-diphenyl-N,N'-bis(3"-methylphenyl)-(1,1'-biphenyl)-4,4'-diamine) (4.7 grams) in tetrahydrofuran (33.3 grams) to which had been added hexane diisocyanate respectively in the following proportions: 0.39 gram (Sample F), 0.80 (Sample G), and 3.9 (Sample H). The best drum for wear resistance was the last one (Sample H), and showed a 2 times improvement in wear to a bias charging roll compared to a control drum with a polycarbonate binder in the charge transport layer, as described in example 27.

Other embodiments and modifications of the present invention may occur to those of ordinary skill in the art subsequent to a review of the information presented herein; these embodiments and modifications, as well as equivalents thereof, are also included within the scope of this invention. 35

What is claimed is:

1. An imaging member which comprises a conductive substrate, a photogenerating material, and a binder comprising a polymer of the formula 40



wherein A is



or a mixture of



wherein R is a hydrogen atom, an alkyl group, an aryl group, or mixtures thereof, B is



**167**

wherein v is an integer of from 1 to about 20,



wherein z is an integer of from 2 to about 20,



wherein u is an integer of from 1 to about 20,



wherein w is an integer of from 1 to about 20,

**168**

-continued

wherein R<sub>1</sub> and R<sub>2</sub> each, independently of the other, are hydrogen atoms, alkyl groups, or aryl groups, and p is an integer of 0 or 1,

wherein p is an integer of 0 or 1,



wherein t is an integer of from 1 to about 20,



wherein (1) Z is



169



wherein p is 0 or 1: (2) Ar is



(3) G is an alkyl group selected from the group consisting of alkyl and isoalkyl groups containing from about 2 to about 10 carbon atoms; (4) Ar' is



(5) X is



170



wherein s is 0, 1, or 2,



and (6) q is 0 or 1; or mixtures thereof, hydroxy-substituted, 30 hydroxyalkyl-substituted, or hydroxyaryl-substituted derivatives thereof, or mixtures thereof, and n is an integer representing the number of repeating monomer units.

2. An imaging member according to claim 1 wherein the 35 imaging member comprises a photogenerating layer comprising from about 5 to about 80 percent by weight of the photogenerating material and from about 20 to about 95 percent by weight of the binder.

3. An imaging member according to claim 1 wherein the 40 imaging member comprises a photogenerating layer and a charge transport layer, said charge transport layer comprising from about 5 to about 90 percent by weight of a charge transport material and from about 10 to about 95 percent by weight of the polymeric binder.

4. An imaging member according to claim 1 wherein the 45 imaging member comprises a photogenerating layer and a charge transport layer, wherein the charge transport material is present in the charge transport layer in an amount of at least about 50 percent by weight.

5. An imaging member according to claim 1 wherein the 50 polymer is prepared by a process which comprises (1) providing a precursor polymer of the formula



60 wherein A is



B is



-continued

 $-\text{CH}_2\text{)}^v-$ ,

5 wherein v is an integer of from 1 to about 20,



wherein z is an integer of from 2 to about 20,



wherein u is an integer of from 1 to about 20,



wherein w is an integer of from 1 to about 20,



173



wherein  $R_1$  and  $R_2$  each, independently of the other, are hydrogen atoms, alkyl groups, or aryl groups, and  $p$  is an integer of 0 or 1,



wherein  $p$  is an integer of 0 or 1,



wherein  $t$  is an integer of from 1 to about 20,



wherein (1)  $Z$  is



174



wherein  $p$  is 0 or 1; (2)  $Ar$  is



40 (3)  $G$  is an alkyl group selected from the group consisting of alkyl and isoalkyl groups containing from about 2 to about 10 carbon atoms; (4)  $Ar'$  is



60 (5)  $X$  is



175

-continued



wherein s is 0, 1, or 2,



or



and (6) q is 0 or 1; or mixtures thereof, hydroxy-substituted, hydroxyalkyl-substituted, or hydroxyaryl-substituted derivatives thereof, or mixtures thereof, and n is an integer representing the number of repeating monomer units, and (2) reacting the precursor polymer with borane, resulting in formation of a polymer of the formula



wherein A is



or a mixture of



wherein R is a hydrogen atom, an alkyl group, an aryl group, or mixtures thereof.

6. An imaging member according to claim 1 wherein the polymer is prepared by a process which comprises (1)

providing a precursor polymer of the formula



10 wherein A is



B is



177

-continued



wherein v is an integer of from 1 to about 20,



wherein  $z$  is an integer of from 2 to about 20,



wherein  $u$  is an integer of from 1 to about 20,



178

wherein w is an integer of from 1 to about 20,



35 wherein  $R_1$  and  $R_2$  each, independently of the other, are hydrogen atoms, alkyl groups, or aryl groups, and  $p$  is an integer of 0 or 1,



wherein  $t$  is an integer of from 1 to about 20.



179



wherein (1) Z is



wherein p is 0 or 1; (2) Ar is



(3) G is an alkyl group selected from the group consisting of alkyl and isoalkyl groups containing from about 2 to about 10 carbon atoms; (4) Ar' is



180



15 (5) X is



45 wherein s is 0, 1, or 2,



and (6) q is 0 or 1; or mixtures thereof, hydroxy-substituted, hydroxyalkyl-substituted, or hydroxyaryl-substituted derivatives thereof, or mixtures thereof, and n is an integer representing the number of repeating monomer units, (2) reacting the precursor polymer with a reagent of the formula  $\text{RMgX}$ , wherein R is a hydrogen atom, an alkyl group, an aryl group, or mixtures thereof and X is a halogen atom, and (3) subsequent to step 2, adding water or acid to the precursor polymer, thereby resulting in formation of a polymer of the formula

181



5

wherein A is



or a mixture of



wherein R is a hydrogen atom, an alkyl group, an aryl group, or mixtures thereof.

7. An imaging member according to claim 1 wherein the number average molecular weight of the polymer is from about 10,000 to about 100,000.

8. An imaging member according to claim 1 wherein the weight average molecular weight of the polymer is from about 20,000 to about 350,000.

9. An imaging member according to claim 1 wherein the polydispersity of the polymer is from about 2 to about 9.

10. An imaging member according to claim 1 wherein the polymer is of the formula



11. An imaging member according to claim 1 wherein the polymer is of the formula



60 or a mixture of

12. An imaging member which comprises a conductive substrate, a photogenerating material, and a binder comprising a crosslinked or chain extended polymer formed by 65 crosslinking or chain extending a precursor polymer of the formula



10

20

25



15 wherein P is a substituent which enables crosslinking of the polymer, a, b, c, and d are each integers of 0, 1, 2, 3, or 4, provided that at least one of a, b, c, and d is equal to or greater than 1 in at least some of the monomer repeat units of the polymer, said crosslinking or chain extension occurring through crosslinking substituents contained on at least some of the monomer repeat units of the precursor polymer,

A is



30



183

wherein R is a hydrogen atom, an alkyl group, an aryl group, or mixtures thereof, B is



184

-continued  
 $-\text{CH}_2\text{)}_v-$ ,

5 wherein v is an integer of from 1 to about 20,



wherein z is an integer of from 2 to about 20,



wherein u is an integer of from 1 to about 20,



30



40



45



50 wherein w is an integer of from 1 to about 20,



60



65

185



wherein  $R_1$  and  $R_2$  each, independently of the other, are hydrogen atoms, alkyl groups, or aryl groups, and  $p$  is an integer of 0 or 1,



wherein  $p$  is an integer of 0 or 1,



wherein  $t$  is an integer of from 1 to about 20,



wherein (1)  $Z$  is



186



wherein  $s$  is 0 or 1; (2)  $Ar$  is



40 (3)  $G$  is an alkyl group selected from the group consisting of alkyl and isoalkyl groups containing from about 2 to about 10 carbon atoms; (4)  $Ar$ 's



60 (5)  $X$  is





and (6) a is 0 or 1; or mixtures thereof, hydroxy-substituted, hydroxyalkyl-substituted, or hydroxyaryl-substituted derivatives thereof, or mixtures thereof, and n is an integer representing the number of repeating monomer units.

13. An imaging member according to claim 12 wherein the crosslinking substituent "P" is a hydroxyalkyl group, a haloalkyl group, an unsaturated ester group, an alkylcarboxymethylene group, an ether group, an epoxy group, an allyl group, an unsaturated ammonium group, an unsaturated phosphonium group, an ethynyl group, a vinyl group, a vinyl ether group, a benzocyclobutene group, a phenolic group, a maleimide group, a biphenylene group, a 5-norbornene-2, 3-dicarboximido group, an isocyanate group, an acryloyl halide group, a vinyl benzyl halide group, an ethynyl benzyl halide group, a methacryloyl halide group, a 2-isocyanatoethyl methacrylate groups, a diisocyanate group, or a mixture thereof.

14. An imaging member according to claim 12 wherein the crosslinking substituent "P" is an acryloyl chloride group, a vinyl benzyl chloride group, an ethynyl benzyl chloride group, a methacryloyl chloride group, a toluene diisocyanate group, a hexane diisocyanate group, or a mixture thereof.

15. An imaging member according to claim 12 wherein the crosslinking substituent "P" is a hexane diisocyanate group.

16. An imaging member according to claim 12 wherein the crosslinking substituent "P" comprises a thermal sensitivity imparting group.

17. An imaging member according to claim 12 wherein the crosslinking substituent "P" comprises a photosensitivity imparting group.

18. An imaging member according to claim 12 wherein the crosslinking substituent "P" comprises a mixture of thermal sensitivity imparting groups and photosensitivity imparting groups.

19. An imaging member according to claim 12 wherein the crosslinking substituent "P" comprises a hydroxymethyl group.

20. An imaging member according to claim 12 wherein the crosslinking substituent "P" comprises a halomethyl group.

21. An imaging member according to claim 12 wherein the crosslinking substituent "P" comprises an unsaturated ester group, an alkylcarboxymethylene group, an ether group, an epoxy group, an allyl ether group, a hydroxyalkyl group, an unsaturated ammonium group, or an unsaturated phosphonium group.

22. An imaging member according to claim 12 wherein the imaging member comprises a photogenerating layer comprising from about 5 to about 80 percent by weight of the photogenerating material and from about 20 to about 95 percent by weight of the binder.

23. An imaging member according to claim 12 wherein the imaging member comprises a photogenerating layer and a charge transport layer, said charge transport layer comprising from about 5 to about 90 percent by weight of a charge transport material and from about 10 to about 95 percent by weight of the polymeric binder.

24. An imaging member according to claim 12 wherein the imaging member comprises a photogenerating layer and a charge transport layer, wherein the charge transport material is present in the charge transport layer in an amount of at least about 50 percent by weight.

25. An imaging member according to claim 12 wherein the precursor polymer is prepared by a process which comprises (1) providing a prepolymer of the formula



wherein A is



B is



189

-continued



wherein v is an integer of from 1 to about 20,



190

wherein z is an integer of from 2 to about 20,



10 wherein u is an integer of from 1 to about 20,



40 wherein w is an integer of from 1 to about 20,



191



5

wherein  $R_1$  and  $R_2$  each, independently of the other, are hydrogen atoms, alkyl groups, or aryl groups, and  $p$  is an integer of 0 or 1,



15

wherein  $p$  is an integer of 0 or 1,



wherein  $t$  is an integer of from 1 to about 20,



wherein (1)  $Z$  is



192



or  $-\text{Ar}-(\text{X})_p-\text{Ar}-$

wherein  $p$  is 0 or 1; (2)  $\text{Ar}$  is



or



20

25

30

35

40

45

50

55

60

65



or



(5)  $\text{X}$  is



193

-continued



wherein s is 0, 1, or 2,



and (6) q is 0 or 1; or mixtures thereof, hydroxy-substituted, 25 hydroxyalkyl-substituted, or hydroxyaryl-substituted derivatives thereof, or mixtures thereof, and n is an integer representing the number of repeating monomer units, (2) reacting the prepolymer with borane, resulting in formation of a polymer of the formula



wherein A is



or a mixture of



wherein R is a hydrogen atom, an alkyl group, an aryl group, or mixtures thereof, and (3) reacting the prepolymer or the 55 polymer with a reactant to form the precursor polymer having "P" substituents thereon.

26. An imaging member according to claim 12 wherein the precursor polymer is prepared by a process which comprises (1) providing a prepolymer of the formula



60

65

65

65

45

40

20

15

5

wherein A is



10 B is



194

195

-continued



wherein u is an integer of from 1 to about 20,



wherein w is an integer of from 1 to about 20,



196

-continued



wherein p is an integer of 0 or 1,

-(CH2O)t-

wherein t is an integer of from 1 to about 20,



wherein (1) Z is



wherein  $p$  is 0 or 1; (2) Ar is



(3) G is an alkyl group selected from the group consisting of alkyl and isoalkyl groups containing from about 2 to about 10 carbon atoms; (4) Ar<sup>1</sup> is



(5) X is



30 wherein s is 0, 1 or 2,



and (6) q is 0 or 1; or mixtures thereof, hydroxy-substituted, hydroxyalkyl-substituted, or hydroxyaryl-substituted derivatives thereof, or mixtures thereof, and n is an integer representing the number of repeating monomer units, (2) reacting the prepolymer with a reagent of the formula  $RMgX$ , wherein R is a hydrogen atom, an alkyl group, an aryl group, or mixtures thereof and X is a halogen atom, (3) subsequent to step 2, adding water or acid to the prepolymer, thereby resulting in formation of a polymer of the formula



60 wherein A is



199

or a mixture of



wherein R is a hydrogen atom, an alkyl group, an aryl group, or mixtures thereof, and (4) reacting the prepolymer or the polymer with a reactant to form the precursor polymer having "P" substituents thereon.

27. An imaging member according to claim 12 wherein the number average molecular weight of the precursor polymer is from about 10,000 to about 100,000.

28. An imaging member according to claim 12 wherein the weight average molecular weight of the precursor polymer is from about 20,000 to about 350,000.

29. An imaging member according to claim 12 wherein the polydispersity of the precursor polymer is from about 2 to about 9.

30. An imaging member according to claim 12 wherein the "A" group is



200

and the "B" group is



31. An imaging member according to claim 1 wherein the "A" group is



and the "B" group is



\* \* \* \* \*